# EUROPEAN PATENT SPECIFICATION

(11) **EP 1 637 924 B1**
(45) Date of publication and mention of the grant of the patent: **21.07.2010**
(21) Application number: 05019875.3
(22) Date of filing: 13.09.2005
(51) Int. Cl.: G03C 1/498, G03C 1/83

(54) **Image forming method using photothermographic material**
Bilderzeugungsverfahren, in dem ein photothermographisches Material verwendet wird
Méthode de formation d'images utilisant un matériau photothermographique

(30) Priority: 13.09.2004 JP 2004265897
(43) Date of publication of application: 22.03.2006
(73) Proprietor: FUJIFILM Corporation, Minato-ku Tokyo (JP)
(72) Inventor: Fukui, Kouta, Minami-Ashigara-shi Kanagawa (JP); Oyamada, Takayoshi, Minami-Ashigara-shi Kanagawa (JP)
(74) Representative: HOFFMANN EITLE

(56) References cited:
- EP-A- 0 803 764
- JP-A- 11 352 624

## Description

The present invention relates to a method of forming images by using a photothermographic material. More particularly, the invention relates to a method of forming images by using a photothermographic material with improved resistance to stain before exposure, improved raw stock storability, and improved resistance to defects after processing.

### Description of the Related Art

In recent years, in the medical field, there has been a strong desire for decreasing the amount of processing liquid waste from the viewpoints of protecting the environment and economy of space. Technology is therefore required for light sensitive photothermographic materials which can be exposed effectively by laser image setters or laser imagers and thermally developed to obtain clear black-toned images of high resolution and sharpness, for use in medical diagnostic applications and for use in photographic technical applications. The light sensitive photothermographic materials do not require liquid processing chemicals and can therefore therefore be supplied to customers as a simpler and environmentally friendly thermal processing system.

While similar requirements also exist in the field of general image forming materials, images for medical imaging in particular require high image quality excellent in sharpness and granularity because fine depiction is required, and further require blue-black image tone from the viewpoint of easy diagnosis. Various kinds of hard copy systems utilizing dyes or pigments, such as ink jet printers and electrophotographic systems, have been marketed as general image forming systems, but they are not satisfactory as output systems for medical images.

Thermal image forming systems utilizing organic silver salts are described in many documents. In particular, photothermographic materials generally have an image forming layer including a catalytically active amount of a photocatalyst (for example, silver halide), a reducing agent, a reducible silver salt (for example, an organic silver salt), and if necessary, a toner for controlling the color tone of developed silver images, dispersed in a binder. Photothermographic materials form black silver images by being heated to a high temperature (for example, 80°C or higher) after imagewise exposure to cause an oxidation-reduction reaction between a silver halide or a reducible silver salt (functioning as an oxidizing agent) and a reducing agent. The oxidation-reduction reaction is accelerated by the catalytic action of a latent image on the silver halide generated by exposure. As a result, a black silver image is formed on the exposed region.

Most conventional photothermographic materials have been generally produced by a process using organic solvents such as toluene, methyl ethyl ketone, and methanol as a solvent. However, use of an organic solvent as a solvent is not advantageous, not only in view of undesired effects on the human body during manufacturing steps, but also in view of the cost due to recovery of solvents and the like.

In view of the above, a manufacturing method using an aqueous dispersion of a hydrophobic polymer as a binder has been disclosed in Japanese Patent Application Laid-Open (JP-A) No. 10-10670 as a method of manufacturing a photothermographic material using a coating solution of an aqueous medium without such concern. Further, JP-A No. 11-84573 also discloses the use of a specified polymer latex as a binder of a surface protective layer.

While photothermographic materials utilizing an organic silver salt have a great merit of containing all components necessary for image formation in the film in advance and being capable of forming images only by heating, there has been demanded, on the other hand, a technique of suppressing change in photographic properties during raw stock storage since such components are also contained during raw stock storage.

Further, in the manufacturing method using the aqueous dispersion of the hydrophobic polymer as a binder described above, since a styrene-butadiene polymer which is a raw material for synthetic rubbers is used as a polymer for use in the binder, the film quality is soft and improvement has been demanded with respect to forces such as pressure, scratching, or the like.

Further, JP-A No. 11-352624 discloses a photothermographic material containing a non-photosensitive organic silver salt in a non-image-forming layer.

### SUMMARY OF THE INVENTION

An aspect of the invention is to provide an image forming method comprising: using a photothermographic material comprising, on at least one side of a support, an image forming layer comprising at least a photosensitive silver halide, a first non-photosensitive organic silver salt, a reducing agent represented by the following formula (R), and a binder, and at least one non-photosensitive layer which is disposed on the same side as the image forming layer and farther from the support than the image forming layer, and comprises a second organic silver salt which is different from the first non-photosensitive organic silver salt, wherein the first non-photosensitive organic silver salt is a silver behenate and the second organic silver salt is a silver salt of an azole compound, 50 % by weight or more of the binder in the image forming layer is formed by a hydrophobic polymer latex having a glass transition temperature of from 0°C to 80°C, 50 % by weight or more of a binder in the non-photosensitive layer is formed by a hydrophobic polymer latex, and the photothermographic material comprises a developing accelerator represented by the following formula (A-1) or (A-2); imagewise exposing the photothermographic material; and thermal developing for 5 seconds to 15 seconds at 110°C to 130°C after imagewise exposure:

Formula (A-1) Q₁-NHNH-Q₂

wherein Q₁ represents an aromatic group or a heterocyclic group which bonds to -NHNH-Q₂ at a carbon atom, and Q₂ represents a carbamoyl group: wherein R₁ represents one selected from an alkyl group,
an acyl group, an acylamino group, a sulphonamide group, an alkoxycarbonyl group, or a carbamoyl group; R₂
represents one selected from a hydrogen atom, a halogen atom, an alkyl group, an alkoxy group, an aryloxy group, an alkylthio group, an arylthio group, an acyloxy group, or a carbonate ester group; R₃ and R₄ each independently represent a group capable of substituting for a hydrogen atom on a benzene ring; and R₃ and R₄ may link together to form a condensed ring: wherein R¹¹ and R¹¹ each independently represent a tertiary alkyl group having 4 to 15 carbon atoms; R¹² and R¹² each independently represent a hydrogen atom or a substituent which can be bonded to the benzene ring; L represents an -S- group or a -CHR¹³-group; R¹³ represents a hydrogen atom or an alkyl group having 1 to 20 carbon atoms; and X¹ and X^{1'} each independently represent a hydrogen atom or a substituent which can be bonded to the benzene ring.

### DETAILED DESCRIPTION OF THE INVENTION

An object of the present invention is to provide a method of forming images by using a photothermographic material with improved resistance to stain before exposure, improved raw stock storability, and improved resistance to defects after processing.

The present invention is explained below in detail.

The photothermographic material used in the present invention has, on at least one side of a support, an image forming layer comprising at least a photosensitive silver halide, a first non-photosensitive organic silver salt, a reducing agent, and a binder and at least one non-photosensitive layer which is disposed on the same side as the image forming layer and farther from the support than the image forming layer, wherein the non-photosensitive layer comprises a second organic silver salt which is different from the first non-photosensitive organic silver salt.

The second organic silver salt a silver salt of an azole compound,

The silver salt of a fatty acid is preferably a silver salt of a saturated fatty acid having 2 to 30 carbon atoms.

The silver salt of a nitrogen-containing heterocyclic compound is preferably a silver salt of an azole compound, and more preferably a silver salt of a benzotriazole compound.

The silver salt of a mercapto compound is preferably a silver salt of a nitrogen-containing heterocyclic mercapto compound.

The silver salt of a poly-carboxylic acid is preferably a silver salt of an aliphatic carboxylic acid or a silver salt of a polymer comprising a monomer component having a carboxy group.

An aqueous dispersion of the second organic silver salt preferably has a silver potential of from +50 mV to +700 mV (with respect to a standard hydrogen electrode) at 25°C.

In the present invention, 50% by weight or more of a solvent of the coating solution for the image forming layer is preferably water. Further, 50% by weight or more of the binder in the image forming layer is a hydrophobic polymer latex.

50% by weight or more of a solvent of the coating solution for the non-photosensitive layer is water. Further, 50% by weight or more of the binder in the non-photosensitive layer is a hydrophobic polymer latex.

The photothermographic material used in the present invention preferably has a non-photosensitive intermediate layer containing 50% by weight or more of a hydrophobic polymer latex as a binder, which is disposed between the image forming layer and the non-photosensitive layer comprising the second organic silver salt.

By the means mentioned above, print-out resistance after image formation and raw stock storability are improved in the photothermographic material, and particularly, image discoloration or color fading at a portion where a fingerprint, sweat is adhered is improved.

### (Second organic silver salt incorporated in non-photosensitive layer)

The second organic silver salt which is different from the first non-photosensitive organic silver salt and incorporated in the non-photosensitive layer used in the invention is a silver salt of an azole compound.

The non-photosensitive layer containing the second organic silver salt mentioned above is at least one layer which is disposed on the same side as the image forming layer and farther from the support than the image forming layer and includes a surface protective layer, an intermediate layer between the surface protective layer and the image forming layer described below. The second organic silver salt is included in at least one layer of these non-photosensitive layers.

The silver salt of a fatty acid is a silver salt of an aliphatic carboxylic acid which has 1 to 30 carbon atoms and may be either linear or branched, saturated or unsaturated. Preferred examples of the silver salt of a fatty acid include silver lignocerate, silver behenate, silver arachidinate, silver stearate, silver oleate, silver linoleate, silver laurate, silver capronate, silver myristate, silver palmitate, silver erucate, silver acetate, silver butyrate, silver propionate, silver valerate, silver enanthate, silver caprylate, silver pelargonate, silver decanoate, and mixtures thereof. Among them, particularly preferred are silver behenate, silver stearate, silver laurate, silver oleate, silver lignocerate, and silver arachidinate.

Concerning the silver salt of a mercapto compound, preferred examples of the mercapto compound include an aliphatic mercapto compound and a heterocyclic mercapto compound. In the case of the aliphatic mercapto compound, the compound preferably has 10 to 30 carbon atoms, and more preferably 10 to 25 carbon atoms. The aliphatic mercapto compound may be either linear or branched, saturated or unsaturated, and unsubstituted or substituted. In the case where the aliphatic mercapto compound has a substituent, the substituent is not particularly limited, but an alkyl group is preferred.

Preferred aliphatic group for the aliphatic mercapto compound is an alkyl group, more preferably an alkyl group having 10 to 23 carbon atoms, which include substituted or unsubstituted, and linear or branched.

Representative examples of the silver salt of an aliphatic mercapto compound are described below, but are not limited to these compounds. For example, there are included a silver salt of an alkylthiol compound having 10 to 25 carbon atoms, and preferably a silver salt of an alkylthiol compound having 10 to 23 carbon atoms.

In the case of a silver salt of a heterocyclic mercapto compound, preferred examples of the heterocycle include a nitrogen-containing heterocycle, a sulfur-containing heterocycle, an oxygen-containing heterocycle, and a selenium-containing heterocycle, more preferred are a nitrogen-containing heterocycle, a sulfur-containing heterocycle, and an oxygen-containing heterocycle. Specific examples of the silver salt of a nitrogen-containing heterocyclic mercapto compound are described below, but are not limited to these examples.
· A silver salt of 3-mercapto-4-phenyl-1,2,4-triazole,
· a silver salt of 2-mercapto-benzimidazole,
· a silver salt of 2-mercapto-5-aminothiazole,
· a silver salt of mercaptotriazine,
· a silver salt of 2-mercaptobenzoxazole,
· a silver salt of the compound described in U.S. Patent (USP) No. 4,123,274 (Knight, et al) (for example, a silver salt of 1,2,4-mercaptothiazole derivative, a silver salt of 3-amino-5-benzylthio-1,2,4-thiazole), and a silver salt of a thione compound (for example, a silver salt of 3-(2-carboxyethyl)-4-methyl-4-thiazoline-2-thione described in USP No. 3,785,830 (Sullivan, et al)).

Concerning the silver salt of a nitrogen-containing heterocyclic compound, specific examples of the nitrogen-containing heterocyclic compound include, but are not limited to these examples, azoles, oxazoles, thiazoles, thiazolines, imidazoles, diazoles, pyridines, indolizines, and triazines. Among them, more preferred are indolizines, imidazoles, and azoles. Preferred examples of the azoles include, triazole, tetrazole, and their derivatives. More preferred are benzimidazoles and derivatives thereof, and benzotriazole and derivatives thereof. Preferred example of the indolizines is a triazaindolizine derivative.

Representative examples of the nitrogen-containing heterocyclic compound further include, but are not limited to these examples, 1,2,4-triazole, benzotriazoles and derivatives thereof, and preferred are benzotriazole, methylbenzotriazole, and 5-chlorobenzotriazole. Further, 1H-tetrazole compounds such as phenylmercaptotetrazole described in USP No. 4,220,709 (de Mauriac), and imidazole and imidazole derivatives described in USP No. 4,260,677 (Winslow, et al) can be described, and benzimidazole and nitrobenzimidazole are preferred. As a triazaindolizine derivative, preferred is 5-mehtyl-7-hydroxy-1,3,5- triazaindolizine.

Concerning the silver salt of an aromatic carboxylic acid, the aromatic carboxylic acid is an unsubstituted or substituted benzenecarboxylic acid where the substituent is not particularly limited. Preferred are benzoic acid and derivatives thereof, and salicylic acid and derivatives thereof.

The silver salt of a poly-carboxylic acid is a silver salt of a polyvalent carboxylic acid. A silver salt of a low-molecular poly-carboxylic acid is represented by the following formula (I).

Formula (I) M¹O₂C-L¹-CO₂M²

In formula (I), L¹ represents an alkylene group, an alkenylene group, an alkynylene group, a cycloalkylene group, an arylene group, a divalent heterocyclic group, a divalent group selected from -C(=O)-, -O-, -S-, -S(=O)-, -S(=O)₂-, and -N(R¹)-, or a divalent group formed by combining these groups. L¹ may further have a substituent. R¹ represents a hydrogen atom or a substituent. M¹ and M² each independently represent a hydrogen atom or a counter ion where at least one of M¹ and M² represents a silver ion (I). Furthermore, the compound represented by formula (I) may further have a carboxy group or a salt thereof.

Specific examples of the compound mentioned above include, but are not limited to these examples, the compounds represented by chemical formulae Nos. 2 to 16 in paragraph Nos. 0024 to 0044 of JP-A No. 2003-330139.

Preferred examples of the carboxylic acid used for forming a silver salt of a low-molecular poly-carboxylic acid include phthalic acid, isophthalic acid, terephthalic acid, malic acid, citric acid, malonic acid, succinic acid, maleic acid, fumaric acid, hemimellitic acid, trimellitic acid, trimesic acid, mellophanic acid, prehnitic acid, pyromellitic acid, oxalic acid, adipic acid, glutaric acid, pimelic acid, suberic acid, azelaic acid, sebacic acid, and naphthalenedicarboxylic acid. Among them, particularly preferred are phthalic acid, succinic acid, adipic acid, glutaric acid, and naphthalenedicarboxylic acid. With respect to plural carboxylic acids, at least one of the carboxylic acid forms a silver salt.

A silver salt of a high-molecular poly-carboxylic acid is a silver salt of a polymer having a repeating unit derived from a monomer containing a carboxy group. Preferred compound can be represented by the following formula (II).

In formula (II), A represents a repeating unit derived from a monomer containing a carboxy group. B represents a repeating unit derived from an ethylenic unsaturated monomer except A. a represents a number of from 5 to 100 in terms of % by weight. b represents a number of from 0 to 95 in terms of % by weight. a + b is equal to 100% by weight.

Preferably, a is a number of from 50 to 100 in terms of % by weight, b is a number of from 0 to 50 in terms of % by weight, and a + b is equal to 100% by weight.

Specifically, the detail explanation are mentioned in paragraph Nos. 0013 to 0074 of JP-A No. 2003-330137.

Specific examples of the carboxylic acid include the compounds described below, but are not limited to these examples. The silver salt formed with the said carboxylic acid is a silver salt of a high-molecular poly-carboxylic acid, which may have at least one silver carboxylate in a molecule.

Among the organic silver salts described above, preferred examples of the silver salt of a fatty acid include silver behenate, silver stearate, silver laurate, silver oleate, silver lignocerate, and silver arachidinate. Preferred examples of the silver salt of a mercapto compound include a silver salt of 3-mercapto-4-phenyl-1,2,4-triazole, a silver salt of 2-mercapto-benzimidazole, and a silver salt of 2-mercapto-5-aminothiazole. Preferred examples of the silver salt of a nitrogen-containing heterocyclic compound include a silver salt of benzotriazole, a silver salt of methylbenzotriazole, a silver salt of benzimidazole, a silver salt of nitrobenzimidazole, and a silver salt of 5-methyl-7-hydroxy-1,3,5-triazaindolizine. Preferred examples of the silver salt of a poly-carboxylic acid include silver phthalate, silver succinate, silver adipate, silver glutarate, and silver naphthalenedicarboxylate. Preferred examples of the silver salt of a high-molecular poly-carboxylic acid include a silver salt of the compound selected from P-1, P-3, and P-5 mentioned above.

Syntheses of the silver salt of a fatty acid and the silver salt of an aliphatic mercapto compound can be carried out according to the conventional methods known in the art. For example, an aliphatic mercapto compound is melted in water by heating at a temperature above the melting point (generally, from 10 °C to 90°C), and then a sodium salt thereof is formed with sodium hydroxide. Thereafter, the sodium salt is reacted with silver nitrate to form crystal of a silver salt of an aliphatic mercapto compound. The obtained silver salt can be dispersed using a suitable dispersing agent to prepare a dispersion thereof. In this preparing process for forming crystal of a silver salt of a fatty acid or a silver salt of an aliphatic mercapto compound, dispersion of the silver salt of a fatty acid or silver salt of an aliphatic mercapto compound may be performed in the presence of hydrophilic colloid such as gelatin. Another method for bringing the silver salt comprises a step of adding a fatty acid or an aliphatic mercapto compound in a reaction vessel and thereto adding silver nitrate.

A silver salt of a heterocyclic mercapto compound and a silver salt of a low-molecular poly-carboxylic acid can be prepared similarly. As an alternative method, for example, preparation can be easily performed for technician in the art, according to the method described in "Jikken Kagaku Koza" (Lecture Series on Experimental Chemistry), 4th Ed, vol. 22, pp. 1 to 43, and pp. 193 to 227. edited by the Chemical Society of Japan, and the references cited above. A silver salt of a nitrogen-containing heterocyclic compound and a silver salt of a heterocyclic mercapto compound can also be prepared by the method described in JP-A No. 1-100177.

A silver salt of a high-molecular poly-carboxylic acid can be prepared by a similar method described above.

The second organic silver salt used for the non-photosensitive layer of the present invention is added in an amount of from 0.001 g/m² to 3 g/m², in terms of a silver amount, more preferably from 0.005 g/m² to 1 g/m², and even more preferably from 0.01 g /m² to 0.5 g /m².

Measurement of silver potentials of a dispersion or an aqueous solution of the second organic silver salt used for the non-photosensitive layer used in the present invention is carried out as follows ; a silver electrode is used as an electrode, and the potential difference of the sample is measured using a saturated calomel electrode as a reference electrode at 40°C while adjusting the pH thereof at 6. Thereafter, the obtained potential is converted to the value based on a standard hydrogen electrode as a reference electrode. The silver potential is preferably from +50 mV to +700 mV (with respect to a standard hydrogen electrode), more preferably from +250 mV to +650 mV, and particularly preferably from +400 mV to +600 mV.

### (First organic silver salt in the image forming layer)

### 1) Composition

The first organic silver salt which can be used in the present invention is relatively stable to light but serves as to supply silver ions and forms silver images when heated to 80°C or higher in the presence of an exposed photosensitive silver halide and a reducing agent. The non-photosensitive organic silver salt may be any material containing a source capable of supplying silver ions that are reducible by a reducing agent. Such a non-photosensitive organic silver salt is disclosed, for example, in Japanese Patent Application Laid-Open (JP-A) No. 10-62899 (paragraph Nos. 0048 to 0049), European Patent (EP) No. 0803764A1 (page 18, line 24 to page 19, line 37), EP No. 0962812A1, JP-A Nos. 11-349591, 2000-7683, and 2000-72711. A silver salt of an organic acid, particularly, a silver salt of a long chained aliphatic carboxylic acid (having 10 to 30 carbon atoms, and preferably having 15 to 28 carbon atoms) is preferable. Preferred examples of the silver salt of a fatty acid can include, for example, silver lignocerate, silver behenate, silver arachidinate, silver stearate, silver oleate, silver laurate, silver capronate, silver myristate, silver palmitate, silver erucate, and mixtures thereof. In the invention, among these silver salts of a fatty acid, it is preferred to use a silver salt of a fatty acid with a silver behenate content of 50 mol% or higher, more preferably, 85 mol% or higher, and even more preferably, 95 mol% or higher. Further, it is preferred to use a silver salt of a fatty acid with a silver erucate content of 2 mol% or lower, more preferably, 1 mol% or lower, and even more preferably, 0.1 mol% or lower.

It is preferred that the content of silver stearate is 1 mol% or lower. When the content of silver stearate is 1 mol% or lower, a silver salt of an organic acid having low fog, high sensitivity and excellent image storability can be obtained. The above-mentioned content of silver stearate is preferably 0.5 mol% or lower, and particularly preferably, silver stearate is not substantially contained.

Further, in the case where the silver salt of an organic acid includes silver arachidinate, it is preferred that the content of silver arachidinate is 6 mol% or lower in order to obtain a silver salt of an organic acid having low fog and excellent image storability. The content of silver arachidinate is more preferably 3 mol% or lower.

### 2) Shape

There is no particular restriction on the shape of the first organic silver salt usable in the invention and it may be needle-like, bar-like, tabular, or flake shaped.

In the invention, a flake shaped organic silver salt is preferred. Short needle-like, rectangular, cuboidal, or potato-like indefinite shaped particles with the major axis to minor axis ratio being lower than 5 are also used preferably. Such organic silver particles suffer less from fogging during thermal development compared with long needle-like particles with the major axis to minor axis length ratio of 5 or higher. Particularly, a particle with the major axis to minor axis ratio of 3 or lower is preferred since it can improve the mechanical stability of the coating film. In the present specification, the flake shaped organic silver salt is defined as described below. When an organic silver salt is observed under an electron microscope, calculation is made while approximating the shape of an organic silver salt particle to a rectangular body and assuming each side of the rectangular body as a, b, c from the shorter side (c may be identical with b) and determining x based on numerical values a, b for the shorter side as below. $x = b / a$

As described above, x is determined for the particles by the number of about 200 and those capable of satisfying the relation: x (average) ≧ 1.5 as an average value x is defined as a flake shape. The relation is preferably: 30 ≧ × (average) ≧ 1.5 and, more preferably, 15 ≧ x (average) ≧ 1.5. By the way, needle-like is expressed as 1 ≦ x (average) < 1.5.

In the flake shaped particle, a can be regarded as a thickness of a tabular particle having a major plane with b and c being as the sides. a in average is preferably from 0.01 µm to 0.3 µm and, more preferably, from 0.1 µm to 0.23 µm. c/b in average is preferably from 1 to 9, more preferably from 1 to 6, even more preferably from 1 to 4 and, most preferably from 1 to 3.

By controlling the equivalent spherical diameter being from 0.05 µm to 1 µm, it causes less agglomeration in the photothermographic material and image storability is improved. The equivalent spherical diameter is preferably from 0.1 µm to 1 µm. In the invention, an equivalent spherical diameter can be measured by a method of photographing a sample directly by using an electron microscope and then image processing the negative images.

In the flake shaped particle, the equivalent spherical diameter of the particle/a is defined as an aspect ratio. The aspect ratio of the flake particle is preferably from 1.1 to 30 and, more preferably, from 1.1 to 15 with a viewpoint of causing less agglomeration in the photothermographic material and improving the image storability.

As the particle size distribution of the organic silver salt, monodispersion is preferred. In the monodispersion, the percentage for the value obtained by dividing the standard deviation for the length of minor axis and major axis by the minor axis and the major axis respectively is, preferably, 100% or less, more preferably, 80% or less and, even more preferably, 50% or less. The shape of the organic silver salt can be measured by analyzing a dispersion of an organic silver salt as transmission type electron microscopic images. Another method of measuring the monodispersion is a method of determining of the standard deviation of the volume weighted mean diameter of the organic silver salt in which the percentage for the value defined by the volume weight mean diameter (variation coefficient), is preferably, 100% or less, more preferably, 80% or less and, even more preferably, 50% or less. The monodispersion can be determined from particle size (volume weighted mean diameter) obtained, for example, by a measuring method of irradiating a laser beam to organic silver salts dispersed in a liquid, and determining a self correlation function of the fluctuation of scattered light to the change of time.

### 3) Preparation

Methods known in the art can be applied to the method for producing the first organic silver salt used in the invention and to the dispersing method thereof. For example, reference can be made to JP-A No. 10-62899, EP Nos. 0803763A1 and 0962812A1, JP-A Nos. 11-349591, 2000-7683, 2000-72711, 2001-163889, 2001-163890, 2001-163827, 2001-33907, 2001-188313, 2001-83652, 2002-6442, 2002-49117, 2002-31870, and 202-107868.

When a photosensitive silver salt is present together during dispersion of the organic silver salt, fog increases and sensitivity becomes remarkably lower, so that it is more preferred that the photosensitive silver salt is not substantially contained during dispersion. In the invention, the amount of the photosensitive silver salt to be dispersed in the aqueous dispersion is preferably 1 mol% or less, more preferably 0.1 mol% or less, per 1 mol of the organic silver salt in the solution and, even more preferably, positive addition of the photosensitive silver salt is not conducted.

In the invention, the photothermographic material can be prepared by mixing an aqueous dispersion of the first organic silver salt and an aqueous dispersion of a photosensitive silver salt and the mixing ratio between the first organic silver salt and the photosensitive silver salt can be selected depending on the purpose. The ratio of the photosensitive silver salt relative to the organic silver salt is preferably in a range of from 1 mol% to 30 mol%, more preferably, from 2 mol% to 20 mol% and, particularly preferably, 3 mol% to 15 mol%. A method of mixing two or more kinds of aqueous dispersions of organic silver salts and two or more kinds of aqueous dispersions of photosensitive silver salts upon mixing is used preferably for controlling the photographic properties.

### 4) Addition amount

While the first organic silver salt according to the invention can be used in a desired amount, a total amount of coated silver including silver halide is preferably in a range of from 0.1 g/m² to 5.0 g/m², more preferably from 0.3 g/m² to 3.0 g/m², and even more preferably from 0.5 g/m² to 2.0 g/m². In particular, in order to improve image storability, the total amount of coated silver is preferably 1.8 mg/m² or less, more preferably 1.6 mg/m² or less. In the case where a preferable reducing agent in the invention is used, it is possible to obtain a sufficient image density by even such a low amount of silver.

### (Reducing agent)

The photothermographic material of the present invention contains a reducing agent for organic silver salts as a thermal developing agent. Reducing agents for organic silver salts can be any substance (preferably, organic substance) capable of reducing silver ions into metallic silver. Examples of reducing agents are described in JP-A No. 11-65021 (column Nos. 0043 to 0045) and EP No. 0803764 (p.7, line 34 to p. 18, line 12).

The reducing agent used in the invention is a reducing agent represented by the following formula (R).

In formula (R), R¹¹ and R¹¹ each independently represent a tertiary alkyl group having 4 to 15 carbon atom.

R¹² and R^{12'} each independently represent a hydrogen atom or a group capable of substituting for a hydrogen atom on a benzene ring. L represents an -S- group or a -CHR¹³- group. R¹³ represents a hydrogen atom or an alkyl group having 1 to 20 carbon atoms. X¹ and X^{1'} each independently represent a hydrogen atom or a group capable of substituting for a hydrogen atom on a benzene ring.

Formula (R) is to be described in detail.

In the following description, when referred to as an alkyl group, it means that the alkyl group contains a cycloalkyl group, as far as it is not mentioned specifically.

### 1) R¹¹ and R^{11'}

R¹¹ and R¹¹ each independently represent a tertiary alkyl group having 4 to 15 carbon atoms. The substituent for the alkyl group has no particular restriction and can include, preferably, an aryl group, a hydroxy group, an alkoxy group, an aryloxy group, an alkylthio group, an arylthio group, an acylamino group, a sulfonamide group, a sulfonyl group, a phosphoryl group, an acyl group, a carbamoyl group, an ester group, a ureido group, a urethane group, a halogen atom.

### 2) R¹² and R^{12'}, X¹ and X^{1'}

R¹² and R^{12'} each independently represent a hydrogen atom or a group capable of substituting for a hydrogen atom on a benzene ring. X¹ and X^{1'} each independently represent a hydrogen atom or a group capable of substituting for a hydrogen atom on a benzene ring. As each of the groups capable of substituting for a hydrogen atom on the benzene ring, an alkyl group, an aryl group, a halogen atom, an alkoxy group, and an acylamino group are described preferably.

### 3) L

L represents an -S- group or a -CHR¹³- group. R¹³ represents a hydrogen atom or an alkyl group having 1 to 20 carbon atoms in which the alkyl group may have a substituent. Specific examples of the unsubstituted alkyl group for R¹³ can include, for example, a methyl group, an ethyl group, a propyl group, a butyl group, a heptyl group, an undecyl group, an isopropyl group, a 1-ethylpentyl group, a 2,4,4-trimethylpentyl group, cyclohexyl group, 2,4-dimethyl-3-cyclohexenyl group, 3,5-dimethyl-3-cyclohexenyl group. Examples of the substituent for the alkyl group can include, similar to the substituent of R¹¹, a halogen atom, an alkoxy group, an alkylthio group, an aryloxy group, an arylthio group, an acylamino group, a sulfonamide group, a sulfonyl group, a phosphoryl group, an oxycarbonyl group, a carbamoyl group, a sulfamoyl group

### 4) Preferred substituents

R¹¹ and R^{11'} are preferably a tertiary alkyl group having 4 to 15 carbon atoms and can include, specifically, a t-butyl group, a t-amyl group, a t-octyl group, R¹¹ and R^{11'} each represent, more preferably, an alkyl group having 4 to 8 carbon atoms and, among them, a t-butyl group, a t-amyl group.

R¹² and R^{12'} are preferably an alkyl group having 1 to 20 carbon atoms and can include, specifically, a methyl group, an ethyl group, a propyl group, a butyl group, an isopropyl group, a t-butyl group, a t-amyl group, a cyclohexyl group, a 1-methylcyclohexyl group, a benzyl group, a methoxymethyl group, a methoxyethyl group. More preferred are a methyl group, an ethyl group, a propyl group, an isopropyl group, and a t-butyl group, and particularly preferred are a methyl group and an ethyl group.

X¹ and X^{1'} are preferably a hydrogen atom, a halogen atom, or an alkyl group, and more preferably a hydrogen atom.

L is preferably a -CHR¹³- group.

R¹³ is preferably a hydrogen atom or an alkyl group having 1 to 15 carbon atoms. The alkyl group is preferably a chain or a cyclic alkyl group. And, a group which has a C=C bond in these alkyl group is also preferably used. Preferable examples of the alkyl group can include a methyl group, an ethyl group, a propyl group, an isopropyl group, a 2,4,4-trimethylpentyl group, a cyclohexyl group, a 2,4-dimethyl-3-cyclohexenyl group, a 3,5-dimetyl-3-cyclohexenyl group. Particularly preferable R¹³ is a hydrogen atom, a methyl group, an ethyl group, a propyl group, an isopropyl group, or a 2,4-dimethyl-3-cyclohexenyl group.

In the case where R¹¹ and R^{11'} are a tertiary alkyl group and R¹² and R^{12'} are a methyl group, R¹³ preferably is a primary or secondary alkyl group having 1 to 8 carbon atoms (a methyl group, an ethyl group, a propyl group, an isopropyl group, a 2,4-dimethyl-3-cyclohexenyl group).

In the case where R¹¹ and R^{11'} are a tertiary alkyl group and R¹² and R^{12'} are an alkyl group other than a methyl group, R¹³ preferably is a hydrogen atom.

In the case where R¹¹ and R^{11'} are not a tertiary alkyl group, R¹³ preferably is a hydrogen atom or a secondary alkyl group, and particularly preferably a secondary alkyl group. As the secondary alkyl group for R¹³, an isopropyl group and a 2,4-dimethyl-3-cyclohexenyl group are preferred.

The reducing agent described above shows different thermal developing performances, color tones of developed silver images depending on the combination of R¹¹, R^{11'}, R¹², R^{12'}, and R¹³. Since these performances can be controlled by using two or more kinds of reducing agents in combination, it is preferred to use two or more kinds of reducing agents in combination depending on the purpose.

Specific examples of the reducing agents of the invention including the compounds represented by formula (R) according to the invention are shown below.

As preferred reducing agents of the invention other than those above, there can be mentioned compounds disclosed in JP-A Nos. 2001-188314, 2001-209145, 2001-350235, and 2002-156727, and EP No. 1278101A2.

The addition amount of the reducing agent is preferably from 0.1 g/m² to 3.0 g/m², more preferably from 0.2 g/m² to 2.0 g/m² and, even more preferably from 0.3 g/m² to 1.0 g/m². It is preferably contained in a range of from 5 mol% to 50 mol%, more preferably from 8 mol% to 30 mol% and, even more preferably from 10 mol% to 20 mol%, per 1 mol of silver in the image forming layer. The reducing agent is preferably contained in the image forming layer.

In the invention, the reducing agent may be incorporated into a photothermographic material by being added into the coating solution, such as in the form of a solution, an emulsion dispersion, a solid fine particle dispersion.

As well known emulsion dispersing method, there can be mentioned a method comprising dissolving the reducing agent in an oil such as dibutylphthalate, tricresylphosphate, dioctylsebacate, tri(2-ethylhexyl)phosphate, using an auxiliary solvent such as ethyl acetate, cyclohexanone, and then adding a surfactant such as sodium dodecylbenzenesulfonate, sodium oleoil-N-methyltaurinate, sodium di(2-ethylhexyl)sulfosuccinate, from which an emulsion dispersion is mechanically produced. During the process, for the purpose of controlling viscosity of oil droplet and refractive index, the addition of polymer such as α -methylstyrene oligomer, poly(t-butylacrylamide), or the like is preferable.

As solid particle dispersing method, there can be mentioned a method comprising dispersing the powder of the reducing agent in a proper solvent such as water, by means of ball mill, colloid mill, vibrating ball mill, sand mill, jet mill, roller mill, or ultrasonics, thereby obtaining solid dispersion. In this case, there may be used a protective colloid (such as poly(vinyl alcohol)), or a surfactant (for instance, an anionic surfactant such as sodium triisopropylnaphthalenesulfonate (a mixture of compounds having the three isopropyl groups in different substitution sites)). In the mills enumerated above, generally used as the dispersion media are beads made of zirconia, and Zr eluting from the beads may be incorporated in the dispersion. Although depending on the dispersing conditions, the amount of Zr incorporated in the dispersion is generally in a range of from 1 ppm to 1000 ppm. It is practically acceptable so long as Zr is incorporated in an amount of 0.5 mg or less per 1 g of silver.

Preferably, an antiseptic (for instance, benzisothiazolinone sodium salt) is added in an aqueous dispersion.

The reducing agent is particularly preferably used as solid particle dispersion, and is added in the form of fine particles having average particle size of from 0.01 µm to 10 µm, preferably from 0.05 µm to 5 µm and, more preferably from 0.1 µm to 2 µm. In the invention, other solid dispersions are preferably used with this particle size range.

### (Development accelerator)

In the photothermographic material of the invention, a development accelerator is used. As a development accelerator, sulfonamide phenolic compounds described in the specification of JP-A No. 2000-267222, and represented by formula (A) described in the specification of JP-A No. 2000-330234; hindered phenolic compounds represented by formula (II) described in JP-A No. 2001-92075; hydrazine compounds described in the specification of JP-A No. 10-62895, represented by formula (I) described in the specification of JP-A No. 11-15116, represented by formula (D) described in the specification of JP-A No. 2002-156727, and represented by formula (1) described in the specification of JP-A No. 2002-278017; and phenolic or naphthalic compounds represented by formula (2) described in the specification of JP-A No. 2001-264929 are used preferably provided that they satisfy formula (4-1) or (A-2) described below. Further, phenolic compounds described in JP-A Nos. 2002-311533 and 2002-341484 are also preferable provided that they satisfy formula (4-1) or (A-2) described below. Naphthalic compounds described in JP-A No. 2003-66558 are particularly preferable provided that they satisfy formula (4-1) or (A-2) described below. The development accelerator described above is used in a range of from 0.1 mol% to 20 mol%, preferably, in a range of from 0.5 mol% to 10 mol% and, more preferably in a range of from 1 mol% to 5 mol%, with respect to the reducing agent. The introducing methods to the photothermographic material can include similar methods as those for the reducing agent and, it is particularly preferred to add as a solid dispersion or an emulsion dispersion. In the case of adding as an emulsion dispersion, it is preferred to add as an emulsion dispersion dispersed by using a high boiling solvent which is solid at a normal temperature and an auxiliary solvent at a low boiling point, or to add as a so-called oilless emulsion dispersion not using the high boiling solvent.

In the present invention, among the development accelerators described above, it is more preferred to use hydrazine compounds described in the specification of JP-A Nos. 2002-156727 and 2002-278017, and naphtholic compounds described in the specification of JP-A No. 2003-66558provided that they satisfy formula (4-1) or (A-2) described below.

The development accelerators used in the invention are compounds represented by the following formulae (A-1) or (A-2).

Formula (A-1) Q₁-NHNH-Q₂

wherein Q₁ represents an aromatic group or a heterocyclic group which bonds to -NHNH-Q₂ at a carbon atom, and Q₂ represents a carbamoyl group.

In formula (A-1), the aromatic group or the heterocyclic group represented by Q₁ is preferably a 5 to 7-membered unsaturated ring. Preferred examples include a benzene ring, a pyridine ring, a pyrazine ring, a pyrimidine ring, a pyridazine ring, a 1,2,4-triazine ring, a 1,3,5-triazine ring, a pyrrole ring, an imidazole ring, a pyrazole ring, a 1,2,3-triazole ring, a 1,2,4-triazole ring, a tetrazole ring, a 1,3,4-thiadiazole ring, a 1,2,4-thiadiazole ring, a 1,2,5-thiadiazole ring, a 1,3,4-oxadiazole ring, a 1,2,4-oxadiazole ring, a 1,2,5-oxadiazole ring, a thiazole ring, an oxazole ring, an isothiazole ring, an isooxazole ring, a thiophene ring. Condensed rings in which the rings described above are condensed to each other are also preferred.

The rings described above may have substituents and in a case where they have two or more substituents, the substituents may be identical or different from each other. Examples of the substituents can include a halogen atom, an alkyl group, an aryl group, a carbonamide group, an alkylsulfonamide group, an arylsulfonamide group, an alkoxy group, an aryloxy group, an alkylthio group, an arylthio group, a carbamoyl group, a sulfamoyl group, a cyano group, an alkylsulfonyl group, an arylsulfonyl group, an alkoxycarbonyl group, an aryloxycarbonyl group, and an acyl group. In the case where the substituents are groups capable of substitution, they may have further substituents and examples of preferred substituents can include a halogen atom, an alkyl group, an aryl group, a carbonamide group, an alkylsulfonamide group, an arylsulfonamide group, an alkoxy group, an aryloxy group, an alkylthio group, an arylthio group, an acyl group, an alkoxycarbonyl group, an aryloxycarbonyl group, a carbamoyl group, a cyano group, a sulfamoyl group, an alkylsulfonyl group, an arylsulfonyl group, and an acyloxy group.

The carbamoyl group represented by Q₂ is a carbamoyl group preferably having 1 to 50 carbon atoms and, more preferably having 6 to 40 carbon atoms, and examples can include unsubstituted carbamoyl, methyl carbamoyl, N-ethylcarbamoyl, N-propylcarbamoyl, N-sec-butylcarbamoyl, N-octylcarbamoyl, N-cyclohexylcarbamoyl, N-tert-butylcarbamoyl, N-dodecylcarbamoyl, N-(3-dodecyloxypropyl)carbamoyl, N-octadecylcarbamoyl, N-{3-(2,4-tert-pentylphenoxy)propyl}carbamoyl, N-(2-hexyldecyl)carbamoyl, N-phenylcarbamoyl, N-(4-dodecyloxyphenyl)carbamoyl, N-(2-chloro-5-dodecyloxycarbonylphenyl)carbamoyl, N-naphthylcarbamoyl, N-3-pyridylcarbamoyl, and N-benzylcarbamoyl.

Next, preferred range for the compound represented by formula (A-1) is to be described. A 5 or 6-membered unsaturated ring is preferred for Q₁, and a benzene ring, a pyrimidine ring, a 1,2,3-triazole ring, a 1,2,4-triazole ring, a tetrazole ring, a 1,3,4-thiadiazole ring, a 1,2,4-thiadiazole ring, a 1,3,4-oxadiazole ring, a 1,2,4-oxadiazole ring, a thioazole ring, an oxazole ring, an isothiazole ring, an isooxazole ring, and a ring in which the ring described above is condensed with a benzene ring or unsaturated hetero ring are more preferred. Further, Q₂ is preferably, a carbamoyl group having a hydrogen atom on the nitrogen atom.

In formula (A-2), R₁ represents one selected from an alkyl group, an acyl group, an acylamino group, a sulfonamide group, an alkoxycarbonyl group, or a carbamoyl group. R₂ represents one selected from a hydrogen atom, a halogen atom, an alkyl group, an alkoxy group, an aryloxy group, an alkylthio group, an arylthio group, an acyloxy group, or a carbonate ester group. R₃ and R₄ each independently represent a group capable of substituting for a hydrogen atom on a benzene ring which is mentioned as the example of the substituent for formula (A-1). R₃ and R₄ may link together to form a condensed ring.

R₁ is preferably an alkyl group having 1 to 20 carbon atoms (for example, a methyl group, an ethyl group, an isopropyl group, a butyl group, a tert-octyl group, a cyclohexyl group), an acylamino group (for example, an acetylamino group, a benzoylamino group, a methylureido group, a 4-cyanophenylureido group), or a carbamoyl group (for example, a n-butylcarbamoyl group, an N,N-diethylcarbamoyl group, a phenylcarbamoyl group, a 2-chlorophenylcarbamoyl group, a 2,4-dichlorophenylcarbamoyl group). An acylamino group (including a ureido group and a urethane group) is more preferred. R₂ is preferably a halogen atom (more preferably, a chlorine atom or a bromine atom), an alkoxy group (for example, a methoxy group, a butoxy group, an n-hexyloxy group, an n-decyloxy group, a cyclohexyloxy group, a benzyloxy group), or an aryloxy group (for example, a phenoxy group, a naphthoxy group.

R₃ is preferably a hydrogen atom, a halogen atom, or an alkyl group having 1 to 20 carbon atoms, and most preferably a halogen atom. R₄ is preferably a hydrogen atom, an alkyl group, or an acylamino group, and more preferably an alkyl group or an acylamino group. Examples of the preferred substituent thereof are similar to those for R₁. In the case where R₄ is an acylamino group, R₄ may preferably link with R₃ to form a carbostyryl ring.

In the case where R₃ and R₄ in formula (A-2) link together to form a condensed ring, a naphthalene ring is particularly preferred as the condensed ring. The same substituent as the example of the substituent referred to for formula (A-1) may bond to the naphthalene ring. In the case where formula (A-2) is a naphtholic compound, R₁ is preferably a carbamoyl group. Among them, a benzoyl group is particularly preferred. R₂ is preferably an alkoxy group or an aryloxy group and, particularly preferably an alkoxy group.

Preferred specific examples for the development accelerator used in the invention are to be described below.

### (Hydrogen bonding compound)

In the invention, in the case where the reducing agent has an aromatic hydroxy group (-OH) or an amino group (-NHR, R represents a hydrogen atom or an alkyl group), particularly in the case where the reducing agent is a bisphenol described above, it is preferred to use in combination, a nonreducing compound having a group capable of reacting with these groups of the reducing agent, and that is also capable of forming a hydrogen bond therewith.

As a group forming a hydrogen bond with a hydroxyl group or an amino group, there can be mentioned a phosphoryl group, a sulfoxide group, a sulfonyl group, a carbonyl group, an amide group, an ester group, a urethane group, a ureido group, a tertiary amino group, a nitrogen-containing aromatic group. Particularly preferred among them is a phosphoryl group, a sulfoxide group, an amide group (not having >N-H moiety but being blocked in the form of >N-Ra (where, Ra represents a substituent other than H)), a urethane group (not having >N-H moiety but being blocked in the form of >N-Ra (where, Ra represents a substituent other than H)), and a ureido group (not having >N-H moiety but being blocked in the form of >N-Ra (where, Ra represents a substituent other than H)).

In the invention, particularly preferable as the hydrogen bonding compound is the compound expressed by formula (D) shown below.

In formula (D), R²¹ to R²³ each independently represent one selected from an alkyl group, an aryl group, an alkoxy group, an aryloxy group, an amino group, or a heterocyclic group, which may be substituted or unsubstituted.

In the case where R²¹ to R²³ contain a substituent, examples of the substituent include a halogen atom, an alkyl group, an aryl group, an alkoxy group, an amino group, an acyl group, an acylamino group, an alkylthio group, an arylthio group, a sulfonamide group, an acyloxy group, an oxycarbonyl group, a carbamoyl group, a sulfamoyl group, a sulfonyl group, a phosphoryl group, in which preferred as the substituents are an alkyl group or an aryl group, e.g., a methyl group, an ethyl group, an isopropyl group, a t-butyl group, a t-octyl group, a phenyl group, a 4-alkoxyphenyl group, a 4-acyloxyphenyl group.

Specific examples of an alkyl group expressed by R²¹ to R²³ include a methyl group, an ethyl group, a butyl group, an octyl group, a dodecyl group, an isopropyl group, a t-butyl group, a t-amyl group, a t-octyl group, a cyclohexyl group, a 1-methylcyclohexyl group, a benzyl group, a phenetyl group, a 2-phenoxypropyl group.

As an aryl group, there can be mentioned a phenyl group, a cresyl group, a xylyl group, a naphthyl group, a 4-t-butylphenyl group, a 4-t-octylphenyl group, a 4-anisidyl group, a 3,5-dichlorophenyl group,

As an alkoxyl group, there can be mentioned a methoxy group, an ethoxy group, a butoxy group, an octyloxy group, a 2-ethylhexyloxy group, a 3,5,5-trimethylhexyloxy group, a dodecyloxy group, a cyclohexyloxy group, a 4-methylcyclohexyloxy group, a benzyloxy group.

As an aryloxy group, there can be mentioned a phenoxy group, a cresyloxy group, an isopropylphenoxy group, a 4-t-butylphenoxy group, a naphthoxy group, a biphenyloxy group.

As an amino group, there can be mentioned are a dimethylamino group, a diethylamino group, a dibutylamino group, a dioctylamino group, an N-methyl-N-hexylamino group, a dicyclohexylamino group, a diphenylamino group, an N-methyl-N-phenylamino group.

Preferred as R²¹ to R²³ is an alkyl group, an aryl group, an alkoxy group, or an aryloxy group. Concerning the effect of the invention, it is preferred that at least one of R²¹ to R²³ is an alkyl group or an aryl group, and more preferably, two or more of them are an alkyl group or an aryl group. From the viewpoint of low cost availability, it is preferred that R²¹ to R²³ are of the same group.

Specific examples of hydrogen bonding compounds represented by formula (D) and others are shown below.

Specific examples of hydrogen bonding compounds other than those enumerated above can be found in those described in EP No. 1,096,310 and in JP-A Nos. 2002-156727 and 2002-318431.

The compound expressed by formula (D) used in the invention can be used in the photothermographic material by being incorporated into the coating solution in the form of solution, emulsion dispersion, or solid fine particle dispersion, similar to the case of reducing agent. However, it is preferably used in the form of solid dispersion. In the solution, the compound expressed by formula (D) forms a hydrogen-bonded complex with a compound having a phenolic hydroxyl group or an amino group, and can be isolated as a complex in crystalline state depending on the combination of the reducing agent and the compound expressed by formula (D).

It is particularly preferred to use the crystal powder thus isolated in the form of solid fine particle dispersion, because it provides stable performance. Further, it is also preferred to use a method of leading to form complex during dispersion by mixing the reducing agent and the compound expressed by formula (D) in the form of powders and dispersing them with a proper dispersion agent using sand grinder mill.

The compound expressed by formula (D) is preferably used in a range from 1 mol% to 200 mol%, more preferably from 10 mol% to 150 mol%, and even more preferably, from 20 mol% to 100 mol%, with respect to the reducing agent.

### (Binder)

Any kind of polymer may be used as the binder for the image forming layer of the invention provided that 50% by weight or mose is formed by a hydrophobic polymer latex, as far as it has a glass transition temperature in a range of from 0°C to 80°C. Suitable as the binder are those that are transparent or translucent, and that are generally colorless, such as natural resin or polymer and their copolymers; synthetic resin or polymer and their copolymer; or media forming a film; for example, included are gelatins, rubbers, poly(vinyl alcohols), hydroxyethyl celluloses, cellulose acetates, cellulose acetate butyrates, poly(vinyl pyrrolidones), casein, starch, poly(acrylic acids), poly(methylmethacrylic acids), poly(vinyl chlorides), poly(methacrylic acids), styrene-maleic anhydride copolymers, styreneacrylonitrile copolymers, styrene-butadiene copolymers, poly(vinyl acetals) (e.g., poly(vinyl formal) or poly(vinyl butyral)), polyesters, polyurethanes, phenoxy resin, poly(vinylidene chlorides), polyepoxides, polycarbonates, poly(vinyl acetates), polyolefins, cellulose esters, and polyamides. A binder may be used with water, an organic solvent or emulsion to form a coating solution.

The glass transition temperature (Tg) of the binder is in a range of from 0°C to 80°C, preferably from 10°C to 70°C and, more preferably from 15°C to 60°C.

In the specification, Tg is calculated according to the following equation. $1 / Tg = Σ \left(Xi/Tgi\right)$
where the polymer is obtained by copolymerization of n monomer compounds (from i=1 to i=n); Xi represents the mass fraction of the ith monomer (ΣXi=1), and Tgi is the glass transition temperature (absolute temperature) of the homopolymer obtained with the ith monomer. The symbol E stands for the summation from i=1 to i=n. Values for the glass transition temperature (Tgi) of the homopolymers derived from each of the monomers were obtained from J. Brandrup and E. H. Immergut, Polymer Handbook (3rd Edition) (Wiley-Interscience, 1989).

The binder may be of two or more kinds of polymers depending on needs. And, the polymer having Tg of 20°C or more and the polymer having Tg of less than 20°C can be used in combination. In the case where two or more kinds of polymers differing in Tg may be blended for use, it is preferred that the weight-average Tg is in the range mentioned above.

In the invention, the image forming layer is preferably formed by applying a coating solution containing 30% by weight or more of water in the solvent and by then drying.

In the invention, in the case where the image forming layer is formed by first applying a coating solution containing 30% by weight or more of water in the solvent and by then drying, furthermore, in the case where the binder of the image forming layer is soluble or dispersible in an aqueous solvent (water solvent), and particularly in the case where a polymer latex having an equilibrium water content of 2% by weight or lower under 25°C and 60%RH is used, the performance can be enhanced. Most preferred embodiment is such prepared to yield an ion conductivity of 2.5 mS/cm or lower, and as such a preparing method, there can be mentioned a refining treatment using a separation function membrane after synthesizing the polymer.

The aqueous solvent in which the polymer is soluble or dispersible, as referred herein, signifies water or water containing mixed therein 70% by weight or less of a water-miscible organic solvent. As water-miscible organic solvents, there can be used, for example, alcohols such as methyl alcohol, ethyl alcohol, propyl alcohol; cellosolves such as methyl cellosolve, ethyl cellosolve, butyl cellosolve; ethyl acetate, dimethylformamide.

The term "aqueous solvent" is also used in the case the polymer is not thermodynamically dissolved, but is present in a so-called dispersed state.

The term "equilibrium water content under 25°C and 60%RH" as referred herein can be expressed as follows: $E ⁢ q ⁢ u ⁢ i ⁢ l ⁢ i ⁢ b ⁢ r ⁢ i ⁢ u ⁢ m w ⁢ a ⁢ t ⁢ e ⁢ r c ⁢ o ⁢ n ⁢ t ⁢ e ⁢ n ⁢ t u ⁢ n ⁢ d ⁢ e ⁢ r 25 ⁢ ° ⁢ C a ⁢ n ⁢ d 60 % R ⁢ H = \left[\left(W⁢1-W⁢0\right)/W⁢0\right] \times 100 \left(% b⁢y w⁢e⁢i⁢g⁢h⁢t\right)$
wherein, W1 is the weight of the polymer in moisture-controlled equilibrium under the atmosphere of 25°C and 60%RH, and W0 is the absolutely dried weight at 25°C of the polymer.

For the definition and the method of measurement for water content, reference can be made to Polymer Engineering Series 14, "Testing methods for polymeric materials" (The Society of Polymer Science, Japan, published by Chijin Shokan).

The equilibrium water content under 25°C and 60%RH is preferably 2% by weight or lower, but is more preferably, in a range of from 0.01% by weight to 1.5% by weight, and is most preferably, from 0.02% by weight to 1% by weight.

The binders used in the invention are, particularly preferably, polymers capable of being dispersed in an aqueous solvent. Examples of dispersed states may include a latex, in which water-insoluble fine particles of hydrophobic polymer are dispersed, or such in which polymer molecules are dispersed in molecular states or by forming micelles, but preferred are latex-dispersed particles. The average particle diameter of the dispersed particles is in a range of from 1 nm to 50,000 nm, preferably from 5 nm to 1,000 nm, more preferably from 10 nm to 500 nm, and even more preferably from 50 nm to 200 nm. There is no particular limitation concerning particle diameter distribution of the dispersed particles, and they may be widely distributed or may exhibit a monodisperse particle diameter distribution.

From the viewpoint of controlling the physical properties of the coating solution, preferred mode of usage includes mixing two or more types of dispersed particles each having monodisperse particle diameter distribution.

In the invention, preferred embodiment of the polymers capable of being dispersed in aqueous solvent includes hydrophobic polymers such as acrylic polymers, polyesters, rubbers (e.g., SBR resin), polyurethanes, poly(vinyl chlorides), poly(vinyl acetates), poly(vinylidene chlorides), polyolefins. As the polymers above, usable are straight chain polymers, branched polymers, or crosslinked polymers; also usable are the so-called homopolymers in which one kind of monomer is polymerized, or copolymers in which two or more kinds of monomers are polymerized. In the case of a copolymer, it may be a random copolymer or a block copolymer.

The molecular weight of these polymers is, in number average molecular weight, in a range of from 5,000 to 1,000,000, preferably from 10,000 to 200,000. Those having too small a molecular weight exhibit insufficient mechanical strength on forming the image forming layer, and those having too large a molecular weight are also not preferred because the resulting film-forming properties are poor. Further, crosslinking polymer latexes are particularly preferred for use.

### <Examples of latex>

Specific examples of preferred polymer latexes are given below, which are expressed by the starting monomers with % by weight given in parenthesis. The molecular weight is given in number average molecular weight. In the case polyfunctional monomer is used, the concept of molecular weight is not applicable because they build a crosslinked structure. Hence, they are denoted as "crosslinking", and the molecular weight is omitted. Tg represents glass transition temperature.

P-1; Latex of -MMA(70) -EA(27) -MAA(3) - (molecular weight 37000, Tg 61°C)

P-2; Latex of -MMA(70) -2EHA(20) -St(5) -AA(5) - (molecular weight 40000, Tg 59 °C)

P-3; Latex of -St(50) -Bu(47) -MAA(3) - (crosslinking, Tg -17°C)

P-4; Latex of -St(68) -Bu(29) -AA(3) - (crosslinking, Tg 17°C)

P-5; Latex of -St(71) -Bu(26) -AA(3) - (crosslinking, Tg 24°C)

P-6; Latex of -St(70) -Bu(27) -1A(3) - (crosslinking)

P-7; Latex of -St(75) -Bu(24) -AA(1) - (crosslinking, Tg 29°C)

P-8; Latex of -St(60) -Bu(35) -DVB(3) -MAA(2) - (crosslinking)

P-9; Latex of -St(70) -Bu(25) -DVB(2) -AA(3) - (crosslinking)

P-10; Latex of -VC(50) -MMA(20) -EA(20) -AN(5) -AA(5) - (molecular weight 80000)

P-11; Latex of -VDC(85) -MMA(5) -EA(5) -MAA(5) - (molecular weight 67000)

P-12; Latex of - Et(90) -MAA(10) - (molecular weight 12000)

P-13; Latex of -St(70) -2EHA(27) -AA(3) - (molecular weight 130000, Tg 43°C)

P-14; Latex of -MMA(63) -EA(35) -AA(2) - (molecular weight 33000, Tg 47°C)

P-15; Latex of -St(70.5) -Bu(26.5) -AA(3) - (crosslinking, Tg 23°C)

P-16; Latex of -St(69.5) -Bu(27.5) -AA(3) - (crosslinking, Tg 20.5°C)

In the structures above, abbreviations represent monomers as follows. MMA: methyl methacrytate, EA: ethyl acrylate, MAA: methacrylic acid, 2EHA: 2-ethylhexyl acrylate, St: styrene, Bu: butadiene, AA: acrylic acid, DVB: divinylbenzene, VC: vinyl chloride, AN: acrylonitrile, VDC: vinylidene chloride, Et: ethylene, IA: itaconic acid.

The polymer latexes above are commercially available, and polymers below are usable. As examples of acrylic polymers, there can be mentioned Cevian A-4635, 4718, and 4601 (all manufactured by Daicel Chemical Industries, Ltd.), Nipol Lx811, 814, 821, 820, and 857 (all manufactured by Nippon Zeon Co., Ltd.); as examples of polyester, there can be mentioned FINETEX ES650, 611, 675, and 850 (all manufactured by Dainippon Ink and Chemicals, Inc.), WD-size and WMS (all manufactured by Eastman Chemical Co.); as examples of polyurethane, there can be mentioned HYDRAN AP10, 20, 30, and 40 (all manufactured by Dainippon Ink and Chemicals, Inc.); as examples of rubber, there can be mentioned LACSTAR 7310K, 3307B, 4700H, and 7132C (all manufactured by Dainippon Ink and Chemicals, Inc.), Nipol Lx416, 410, 438C, and 2507 (all manufactured by Nippon Zeon Co., Ltd.); as examples of poly(vinyl chloride), there can be mentioned G351 and G576 (all manufactured by Nippon Zeon Co., Ltd.); as examples of poly(vinylidene chloride), there can be mentioned L502 and L513 (all manufactured by Asahi Chemical Industry Co., Ltd.); as examples of polyolefin, there can be mentioned Chemipearl S120 and SA100 (all manufactured by Mitsui Petrochemical Industries, Ltd.).

The polymer latex above may be used alone, or may be used by blending two or more kinds depending on needs.

### <Preferable latexes>

Particularly preferable as the polymer latex for use in the invention are that of styrene-butadiene copolymer. The mass ratio of monomer unit for styrene to that of butadiene constituting the styrene-butadiene copolymer is preferably in a range of from 40:60 to 95:5. Further, the monomer unit of styrene and that of butadiene preferably account for 60% by weight to 99% by weight with respect to the copolymer.

Further, the polymer latex used in the invention preferably contains acrylic acid or methacrylic acid in a range of from 1% by weight to 6% by weight with respect to the sum of styrene and butadiene, and more preferably from 2% by weight to 5% by weight. The polymer latex used in the invention preferably contains acrylic acid. Preferable range of molecular weight is similar to that described above.

As the latex of styrene-butadiene copolymer preferably used in the invention, there can be mentioned P-3 to P-8, and P-15, or commercially available LACSTAR 3307B, LACSTAR 7132C, Nipol Lx416.

In the image forming layer of the photothermographic material according to the invention, if necessary, there can be added hydrophilic polymers such as gelatin, poly(vinyl alcohol), methyl cellulose, hydroxypropyl cellulose, carboxymethyl cellulose. These hydrophilic polymers are added at an amount of 30% by weight or less, and preferably 20% by weight or less, with respect to the total weight of the binder incorporated in the image forming layer.

According to the invention, the layer containing organic silver salt (image forming layer) is preferably formed by using polymer latex for the binder. According to the amount of the binder for the image forming layer, the mass ratio of total binder to organic silver salt (total binder/organic silver salt) is preferably in a range of from 1/10 to 10/1, more preferably from 1/3 to 5/1, and even more preferably from 1/1 to 3/1.

The image forming layer is, in general, a photosensitive layer (image forming layer) containing a photosensitive silver halide, i.e., the photosensitive silver salt; in such a case, the mass ratio of total binder to silver halide (total binder/silver halide) is in a range of 400 or lower and 5 or higher, and more preferably, 200 or lower and 10 or higher.

The total amount of binder in the image forming layer used in the invention is preferably in a range of from 0.2 g/m² to 30 g/m², more preferably from 1 g/m² to 15 g/m², and even more preferably from 2 g/m² to 10 g/m². As for the image forming layer of the invention, there may be added a crosslinking agent for crosslinking, or a surfactant or the like to improve coating properties.

### (Preferred solvent of coating solution)

In the invention, a solvent of a coating solution for the image forming layer in the photothermographic material used in the invention (wherein a solvent and water are collectively described as a solvent for simplicity) is preferably an aqueous solvent containing water at 50% by weight or more. Examples of solvents other than water may include any of water-miscible organic solvents such as methyl alcohol, ethyl alcohol, isopropyl alcohol, methyl cellosolve, ethyl cellosolve, dimethylformamide and ethyl acetate. A water content in a solvent is preferably 50% by weight or higher, and more preferably 70% by weight or higher. Concrete examples of a preferable solvent composition, in addition to water= 100, are compositions in which methyl alcohol is contained at ratios of water/methyl alcohol = 90/10 and 70/30, in which dimethylformamide is further contained at a ratio of water/methyl alcohol/dimethylformamide = 80/15/5, in which ethyl cellosolve is further contained at a ratio of water/methyl alcohol/ethyl cellosolve = 85/10/5, and in which isopropyl alcohol is further contained at a ratio of water/methyl alcohol/isopropyl alcohol = 85/10/5 (wherein the numerals presented above are values in % by weight).

### (Photosensitive silver halide)

### 1) Halogen composition

For the photosensitive silver halide used in the invention, there is no particular restriction on the halogen composition and silver chloride, silver bromochloride, silver bromide, silver iodobromide, silver iodochlorobromide, and silver iodide can be used. Among them, silver bromide, silver iodobromide, and silver iodide are preferred. The distribution of the halogen composition in a grain may be uniform or the halogen composition may be changed stepwise, or it may be changed continuously. Further, a silver halide grain having a core/shell structure can be used preferably. Preferred structure is a twofold to fivefold structure and, more preferably, core/shell grain having a twofold to fourfold structure can be used. Further, a technique of localizing silver bromide or silver iodide to the surface of a silver chloride, silver bromide or silver chlorobromide grains can also be used preferably.

### 2) Method of grain formation

The method of forming photosensitive silver halide is well-known in the relevant art and, for example, methods described in Research Disclosure No. 10729, June 1978 and USP No. 3,700,458 can be used. Specifically, a method of preparing a photosensitive silver halide by adding a silver-supplying compound and a halogen-supplying compound in a gelatin or other polymer solution and then mixing them with an organic silver salt is used. Further, a method described in JP-A No. 11-119374 (paragraph Nos. 0217 to 0224) and methods described in JP-A Nos. 11-352627 and 2000-347335 are also preferred.

### 3) Grain size

The grain size of the photosensitive silver halide is preferably small with an aim of suppressing clouding after image formation and, specifically, it is 0.20 µm or less, more preferably, in a range of from 0.01 µm to 0.15 µm and, even more preferably, from 0.02 µm to 0.12 µm. The grain size as used herein means an average diameter of a circle converted such that it has a same area as a projected area of the silver halide grain (projected area of a major plane in a case of a tabular grain).

### 4) Grain shape

The shape of the silver halide grain can include, for example, cubic, octahedral, tabular, spherical, rod-like, or potato-like shape. The cubic grain is particularly preferred in the invention. A silver halide grain rounded at corners can also be used preferably. The surface indices (Miller indices) of the outer surface of a photosensitive silver halide grain is not particularly restricted, and it is preferable that the ratio occupied by the {100} face is large, because of showing high spectral sensitization efficiency when a spectral sensitizing dye is adsorbed. The ratio is preferably 50% or higher, more preferably, 65% or higher and, even more preferably, 80% or higher. The ratio of the {100} face, Miller indices, can be determined by a method described in T. Tani; J. Imaging Sci., vol. 29, page 165, (1985) utilizing adsorption dependency of the {111} face and {100} face in adsorption of a sensitizing dye.

### 5) Heavy metal

The photosensitive silver halide grain used in the invention can contain metals or complexes of metals belonging to groups 6 to 13 of the periodic table (showing groups 1 to 18). Preferred are metals or complexes of metals belonging to groups 6 to 10. The metal or the center metal of the metal complex from groups 6 to 10 of the periodic table is preferably rhodium, ruthenium, iridium, or ferrum. The metal complex may be used alone, or two or more kinds of complexes comprising identical or different species of metals may be used together. A preferred content is in a range from 1 × 10⁻⁹ mol to 1 × 10⁻³ mol per 1 mol of silver. The heavy metals, metal complexes and the adding method thereof are described in JP-A No. 7-225449, in paragraph Nos. 0018 to 0024 of JP-A No.11-65021 and in paragraph Nos. 0227 to 0240 of JP-A No. 11-119374.

In the present invention, a silver halide grain having a hexacyano metal complex present on the outermost surface of the grain is preferred. The hexacyano metal complex includes, for example, [Fe(CN)₆]⁴⁻, [Fe(CN)₆]³⁻, [Ru(CN)₆]⁴⁻, [Os(CN)₆]⁴⁻, [Co(CN)₆]³⁻, [Rh(CN)₆]³⁻, [Ir(CN)₆]³⁻, [Cr(CN)₆]³⁻, and [Re(CN)₆]³⁻. In the invention, hexacyano Fe complex is preferred.

Since the hexacyano complex exists in ionic form in an aqueous solution, paired cation is not important and alkali metal ion such as sodium ion, potassium ion, rubidium ion, cesium ion and lithium ion, ammonium ion, alkyl ammonium ion (for example, tetramethyl ammonium ion, tetraethyl ammonium ion, tetrapropyl ammonium ion, and tetra(n-butyl) ammonium ion), which are easily miscible with water and suitable to precipitation operation of a silver halide emulsion are preferably used.

The hexacyano metal complex can be added while being mixed with water, as well as a mixed solvent of water and an appropriate organic solvent miscible with water (for example, alcohols, ethers, glycols, ketones, esters, amides) or gelatin.

The addition amount of the hexacyano metal complex is preferably from 1 × 10⁻⁵ mol to 1 × 10⁻² mol and, more preferably, from 1 × 10⁻⁴ mol to 1 × 10⁻³ mol, per 1 mol of silver in each case.

In order to allow the hexacyano metal complex to be present on the outermost surface of a silver halide grain, the hexacyano metal complex is directly added in any stage of: after completion of addition of an aqueous solution of silver nitrate used for grain formation, before completion of an emulsion formation step prior to a chemical sensitization step, of conducting chalcogen sensitization such as sulfur sensitization, selenium sensitization and tellurium sensitization or noble metal sensitization such as gold sensitization, during a washing step, during a dispersion step and before a chemical sensitization step. In order not to grow fine silver halide grains, the hexacyano metal complex is rapidly added preferably after the grain is formed, and it is preferably added before completion of the emulsion formation step.

Addition of the hexacyano complex may be started after addition of 96% by weight of an entire amount of silver nitrate to be added for grain formation, more preferably started after addition of 98% by weight and, particularly preferably, started after addition of 99% by weight.

When any of the hexacyano metal complex is added after addition of an aqueous silver nitrate just before completion of grain formation, it can be adsorbed to the outermost surface of the silver halide grain and most of them form an insoluble salt with silver ions on the surface of the grain. Since the hexacyano iron (II) silver salt is a less soluble salt than Agl, re-dissolution with fine grains can be prevented and fine silver halide grains with smaller grain size can be prepared.

Metal atoms that can be contained in the silver halide grain used in the invention (for example, [Fe(CN)₆]⁴⁻), desalting method of a silver halide emulsion and chemical sensitizing method are described in paragraph Nos. 0046 to 0050 of JP-A No.11-84574, in paragraph Nos. 0025 to 0031 of JP-A No. 11-65021, and paragraph Nos. 0242 to 0250 of JP-A No.11-119374.

### 6) Gelatin

As the gelatin contained the photosensitive silver halide emulsion used in the invention, various kinds of gelatins can be used. It is necessary to maintain an excellent dispersion state of a photosensitive silver halide emulsion in an organic silver salt containing coating solution, and gelatin having a molecular weight of 10,000 to 1,000,000 is preferably used. Phthalated gelatin is also preferably used. These gelatins may be used at grain formation step or at the time of dispersion after desalting treatment and it is preferably used at grain formation step.

### 7) Sensitizing dye

As the sensitizing dye applicable in the invention, those capable of spectrally sensitizing silver halide grains in a desired wavelength region upon adsorption to silver halide grains having spectral sensitivity suitable to the spectral characteristic of an exposure light source can be advantageously selected. The sensitizing dyes and the adding method are disclosed, for example, JP-A No. 11-65021 (paragraph Nos. 0103 to 0109), as a compound represented by the formula (II) in JP-A No. 10-186572, dyes represented by the formula (I) in JP-A No. 11-119374 (paragraph No. 0106), dyes described in USP Nos. 5,510,236 and 3,871,887 (Example 5), dyes disclosed in JP-A Nos. 2-96131 and 59-48753, as well as in page 19, line 38 to page 20, line 35 of EP No. 0803764A1, and in JP-A Nos. 2001-272747, 2001-290238 and 2002-23306. The sensitizing dyes described above may be used alone or two or more of them may be used in combination. In the invention, sensitizing dye can be added preferably after a desalting step and before coating, and more preferably after a desalting step and before the completion of chemical ripening.

In the invention, the sensitizing dye may be added at any amount according to the property of sensitivity and fogging, but it is preferably added from 10⁻⁶ mol to 1 mol, and more preferably from 10⁻⁴ mol to 10⁻¹ mol, per 1 mol of silver halide in the image forming layer.

The photothermographic material used in the invention can contain super sensitizers in order to improve the spectral sensitizing effect. The super sensitizers usable in the invention can include those compounds described in EP-A No. 587338, USP Nos. 3,877,943 and 4,873,184, JP-A Nos. 5-341432, 11-109547, and 10-111543.

### 8) Chemical sensitization

The photosensitive silver halide grain in the invention is preferably chemically sensitized by sulfur sensitizing method, selenium sensitizing method or tellurium sensitizing method. As the compound used preferably for sulfur sensitizing method, selenium sensitizing method and tellurium sensitizing method, known compounds, for example, compounds described in JP-A No. 7-128768 can be used. Particularly, tellurium sensitization is preferred in the invention and compounds described in the literature cited in paragraph No. 0030 in JP-A No. 11-65021 and compounds shown by formulae (II), (III), and (IV) in JP-A No. 5-313284 are preferred.

The photosensitive silver halide grain in the invention is preferably chemically sensitized by gold sensitizing method alone or in combination with the chalcogen sensitization described above. As the gold sensitizer, those having an oxidation number of gold of either +1 or +3 are preferred and those gold compounds used usually as the gold sensitizer are preferred.

As typical examples, chloroauric acid, bromoauric acid, potassium chloroaurate, potassium bromoaurate, auric trichloride, potassium auric thiocyanate, potassium iodoaurate, tetracyanoauric acid, ammonium aurothiocyanate and pyridyl trichloro gold are preferred. Further, gold sensitizers described in USP No. 5,858,637 and JP-A No. 2002-278016 are also used preferably.

In the invention, chemical sensitization can be applied at any time so long as it is after grain formation and before coating and it can be applied, after desalting, (1) before spectral sensitization, (2) simultaneously with spectral sensitization, (3) after spectral sensitization, (4) just before coating.

The amount of sulfur, selenium, or tellurium sensitizer used in the invention may vary depending on the silver halide grain used, the chemical ripening condition and it is used by 10⁻⁸ mol to 10⁻² mol, preferably, 10⁻⁷ mol to 10⁻³ mol, per 1 mol of silver halide.

The addition amount of the gold sensitizer may vary depending on various conditions and it is generally from 10⁻⁷ mol to 10⁻³ mol and, preferably from 10⁻⁶ mol to 5 × 10⁻⁴ mol, per 1 mol of silver halide.

There is no particular restriction on the condition for the chemical sensitization in the invention and, appropriately, the pH is from 5 to 8, the pAg is from 6 to 11, and the temperature is from 40°C to 95°C.

In the silver halide emulsion used in the invention, a thiosulfonic acid compound may be added by the method shown in EP-A No. 293,917.

A reductive compound is used preferably for the photosensitive silver halide grain in the invention. As the specific compound for the reduction sensitization, ascorbic acid or thiourea dioxide is preferred, as well as use of stannous chloride, aminoimino methane sulfonic acid, hydrazine derivatives, borane compounds, silane compounds and polyamine compounds are preferred. The reduction sensitizer may be added at any stage in the photosensitive emulsion producing process from crystal growth to the preparation step just before coating. Further, it is preferred to apply reduction sensitization by ripening while keeping the pH to 7 or higher or the pAg to 8.3 or lower for the emulsion, and it is also preferred to apply reduction sensitization by introducing a single addition portion of silver ions during grain formation.

### 9) Compound that can be one-electron-oxidized to provide a one-electron oxidation product which releases one or more electrons

The photothermographic material used in the invention preferably contains a compound that can be one-electron-oxidized to provide a one-electron oxidation product which releases one or more electrons. The said compound can be used alone or in combination with various chemical sensitizers described above to increase the sensitivity of silver halide.

As the compound that can be one-electron-oxidized to provide a one-electron oxidation product which releases one or more electrons is preferably a compound selected from the following Groups 1 or 2.

(Group 1) a compound that can be one-electron-oxidized to provide a one-electron oxidation product which further releases one or more electrons, due to being subjected to a subsequent bond cleavage reaction;

(Group 2) a compound that can be one-electron-oxidized to provide a one-electron oxidation product, which further releases one or more electrons after being subjected to a subsequent bond formation reaction.

The compound of Group 1 will be explained below.

In the compound of Group 1, as for a compound that can be one-electron-oxidized to provide a one-electron oxidation product which further releases one electron, due to being subjected to a subsequent bond cleavage reaction, specific examples include examples of compound referred to as "one photon two electrons sensitizer" or "deprotonating electron-donating sensitizer" described in JP-A No. 9-211769 (Compound PMT-1 to S-37 in Tables E and F, pages 28 to 32); JP-A No. 9-211774; JP-A No. 11-95355 (Compound INV 1 to 36); JP-W No. 2001-500996 (Compound 1 to 74, 80 to 87, and 92 to 122); USP Nos. 5747235 and 5747236; EP No. 786692A1 (Compound INV 1 to 35); EP No. 893732A1; USP Nos. 6054260 and 5994051; etc. Preferred ranges of these compounds are the same as the preferred ranges described in the quoted specifications.

In the compound of Group 1, as for a compound that can be one-electron-oxidized to provide a one-electron oxidation product which further releases one or more electrons, due to being subjected to a subsequent bond cleavage reaction, specific examples include the compounds represented by formula (1) (same as formula (1) described in JP-A No. 2003-114487), formula (2) (same as formula (2) described in JP-A No. 2003-114487), formula (3) (same as formula (1) described in JP-A No. 2003-114488), formula (4) (same as formula (2) described in JP-A No. 2003-114488), formula (5) (same as formula (3) described in JP-A No. 2003-114488), formula (6) (same as formula (1) described in JP-A No. 2003-75950), formula (7) (same as formula (2) described in JP-A No. 2003-75950), and formula (8), and the compound represented by formula (9) among the compounds which can undergo the chemical reaction represented by reaction formula (1). And the preferable range of these compounds is the same as the preferable range described in the quoted specification.

In formulae (I) and (2), RED₁ and RED₂ each independently represent a reducing group. R₁ represents a nonmetallic atomic group forming a cyclic structure equivalent to a tetrahydro derivative or an octahydro derivative of a 5 or 6-membered aromatic ring (including a hetero aromatic ring) with a carbon atom (C) and RED₁. R₂, R₃, and R₄ each independently represent a hydrogen atom or a substituent. Lv₁ and Lv₂ each independently represent a leaving group. ED represents an electron-donating group.

In formulae (3), (4), and (5), Z₁ represents an atomic group capable to form a 6-membered ring with a nitrogen atom and two carbon atoms of a benzene ring. R₅, R₆, R₇, R₉, R₁₀, R₁₁, R₁₃, R₁₄, R₁₅, R₁₆, R₁₇, R₁₈, and R₁₉ each independently represent a hydrogen atom or a substituent. R₂₀ represents a hydrogen atom or a substituent, however, in the case where R₂₀ represents a group other than an aryl group, R₁₆ and R₁₇ bond to each other to form an aromatic ring or a hetero aromatic ring. R₈ and R₁₂ represent a substituent capable of substituting for a hydrogen atom on a benzene ring. m₁ represents an integer of 0 to 3, and m2 represents an integer of 0 to 4. Lv₃, Lv₄, and Lv₅ each independently represent a leaving group. In formulae (6) and (7), RED₃ and RED₄ each independently represent a reducing group. R₂₁ to R₃₀ each independently represent a hydrogen atom or a substituent. Z₂ represents one selected from -CR₁₁₁R₁₁₂-, -NR₁₁₃-, or -O-. R₁₁₁, and R₁₁₂ each independently represent a hydrogen atom or a substituent. R₁₁₃ represents one selected from a hydrogen atom, an alkyl group, an aryl group, or a heterocyclic group.

In formula (8), RED₅ is a reducing group and represents an arylamino group or a heterocyclic amino group. R₃₁ represents a hydrogen atom or a substituent. X represents one selected from an alkoxy group, an aryloxy group, a heterocyclic oxy group, an alkylthio group, an arylthio group, a heterocyclic thio group, an alkylamino group, an arylamino group, or a heterocyclic amino group. Lv₆ is a leaving group and represents a carboxy group or a salt thereof, or a hydrogen atom.

The compound represented by formula (9) is a compound that undergoes a bonding reaction represented by reaction fomula (1) after undergoing two-electrons-oxidation accompanied by decarbonization and further oxidized. In reaction formula (1), R₃₂ and R₃₃ represent a hydrogen atom or a substituent. Z₃ represents a group to form a 5 or 6-membered heterocycle with C=C. Z₄ represents a group to form a 5 or 6-membered aryl group or heterocyclic group with C=C. M represents one selected from a radical, a radical cation, and a cation. In formula (9), R₃₂, R₃₃, and Z₃ are the same as those in reaction formula (1). Z₅ represents a group to form a 5 or 6-membered cyclic aliphatic hydrocarbon group or heterocyclic group with C-C.

Next, the compound of Group 2 is explained.

In the compound of Group 2, as for a compound that can be one-electron-oxidized to provide a one-electron oxidation product which further releases one or more electrons, after being subjected to a subsequent bond cleavage reaction, specific examples can include the compound represented by formula (10) (same as formula (1) described in JP-A No.2003-140287), and the compound represented by formula (11) which can undergo the chemical reaction represented by reaction formula (1). The preferable range of these compounds is the same as the preferable range described in the quoted specification.

Formula (10) RED₆-Q-Y

In formula (10), RED₆ represents a reducing group which can be one-electron-oxidized. Y represents a reactive group containing a carbon-carbon double bond part, a carbon-carbon triple bond part, an aromatic group part, or benzo-condensed nonaromatic heterocyclic part which can react with one-electron-oxidized product formed by one-electron-oxidation of RED₆ to form a new bond. Q represents a linking group to link RED₆ and Y.

The compound represented by formula (11) is a compound that undergoes a bonding reaction represented by reaction formula (1) by being oxidized. In reaction formula (1), R₃₂ and R₃₃ each independently represent a hydrogen atom or a substituent. Z₃ represents a group to form a 5 or 6-membered heterocycle with C=C. Z₄ represents a group to form a 5 or 6-membered aryl group or heterocyclic group with C=C. Z₅ represents a group to form a 5 or 6-membered cyclic aliphatic hydrocarbon group or heterocyclic group with C-C. M represents one selected from a radical, a radical cation, and a cation. In formula (11), R₃₂, R₃₃, Z₃, and Z₄ are the same as those in reaction formula (1).

The compounds of Groups 1 or 2 preferably are "the compound having an adsorptive group to silver halide in a molecule" or "the compound having a partial structure of a spectral sensitizing dye in a molecule". The representative adsorptive group to silver halide is the group described in JP-A No. 2003-156823, page 16 right, line 1 to page 17 right, line 12. A partial structure of a spectral sensitizing dye is the structure described in JP-A No. 2003-156823, page 17 right, line 34 to page 18 right, line 6.

As the compound of Groups 1 or 2, "the compound having at least one adsorptive group to silver halide in a molecule" is more preferred, and "the compound having two or more adsorptive groups to silver halide in a molecule" is further preferred. In the case where two or more adsorptive groups exist in a single molecule, those adsorptive groups may be identical or different from each other.

As preferable adsorptive group, a mercapto-substituted nitrogen-containing heterocyclic group (e.g., a 2-mercaptothiazole group, a 3-mercapto-1,2,4-triazole group, a 5-mercaptotetrazole group, a 2-mercapto-1,3,4-oxadiazole group, a 2-mercaptobenzoxazole group, a 2-mercaptobenzothiazole group, a 1,5-dimethyl-1,2,4-triazolium-3-thiolate group) or a nitrogen-containing heterocyclic group having -NH-group as a partial structure of heterocycle capable to form a silver imidate (>NAg) (e.g., a benzotriazole group, a benzimidazole group, an indazole group) are described. A 5-mercaptotetrazole group, a 3-mercapto-1, 2,4-triazole group and a benzotriazole group are particularly preferable and a 3-mercapto-1,2,4-triazole group and a 5-mercaptotetrazole group are most preferable.

As an adsorptive group, the group which has two or more mercapto groups as a partial structure in a molecule is also particularly preferable. Herein, a mercapto group (-SH) may become a thione group in the case where it can tautomerize. Preferred examples of an adsorptive group having two or more mercapto groups as a partial structure (dimercapto-substituted nitrogen-containing heterocyclic group) are a 2,4-dimercaptopyrimidine group, a 2,4-dimercaptotriazine group and a 3,5-dimercapto-1,2,4-triazole group.

Further, a quaternary salt structure of nitrogen or phosphorus is also preferably used as an adsorptive group. As typical quaternary salt structure of nitrogen, an ammonio group (a trialkylammonio group, a dialkylarylammonio group, a dialkylheteroarylammonio group, an alkyldiarylammonio group, an alkyldiheteroarylammonio group) and a nitrogen-containing heterocyclic group containing quaternary nitrogen atom can be used. As a quaternary salt structure of phosphorus, a phosphonio group (a trialkylphosphonio group, a dialkylarylphosphonio group, a dialkylheteroarylphosphonio group, an alkyldiarylphosphonio group, an alkyldiheteroarylphosphonio group, a triarylphosphonio group, a triheteroarylphosphonio group) is described. A quaternary salt structure of nitrogen is more preferably used and a 5 or 6-membered aromatic heterocyclic group containing a quaternary nitrogen atom is further preferably used. Particularly preferably, a pyridinio group, a quinolinio group and an isoquinolinio group are used. These nitrogen-containing heterocyclic groups containing a quaternary nitrogen atom may have any substituent.

Examples of counter anions of quaternary salt are a halogen ion, carboxylate ion, sulfonate ion, sulfate ion, perchlorate ion, carbonate ion, nitrate ion, BF₄⁻, PF₆⁻, Ph₄B⁻. In the case where the group having negative charge at carboxylate group exists in a molecule, an inner salt may be formed with it. As a counter ion outside of a molecule, chloro ion, bromo ion, and methanesulfonate ion are particularly preferable.

The preferred structure of the compound represented by Groups 1 or 2 having a quaternary salt of nitrogen or phosphorus as an adsorptive group is represented by formula (X).

Formula (X) (P-Q₁-)ᵢ-R(-Q₂-S)ⱼ

In formula (X), P and R each independently represent a quaternary salt structure of nitrogen or phosphorus, which is not a partial structure of a spectral sensitizing dye. Q₁ and Q₂ each independently represent a linking group and typically represent a single bond, an alkylene group, an arylene group, a heterocyclic group, -O-, -S-, -NR_{N}, -C(=O)-, -SO₂- -SO-, -P(=O)- or combinations of these groups. Herein, R_{N} represents one selected from a hydrogen atom, an alkyl group, an aryl group, or a heterocyclic group. S represents a residue which is obtained by removing one atom from the compound represented by Group 1 or 2. i and j are an integer of one or more and are selected in a range of i+j= 2 to 6. The case where i is 1 to 3 and j is 1 to 2 is preferable, the case where i is 1 or 2 and j is 1 is more preferable, and the case where i is 1 and j is 1 is particularly preferable. The compound represented by formula (X) preferably has 10 to 100 carbon atoms in total, more preferably 10 to 70 carbon atoms, further preferably 11 to 60 carbon atoms, and particularly preferably 12 to 50 carbon atoms in total.

The compounds of Groups 1 or 2 may be used at any time during preparation of the photosensitive silver halide emulsion and production of the photothermographic material. For example, the compound may be used in a photosensitive silver halide grain formation step, in a desalting step, in a chemical sensitization step, before coating. The compound may be added in several times during these steps. The compound is preferably added after the photosensitive silver halide grain formation step and before the desalting step; at the chemical sensitization step (just before the chemical sensitization to immediately after the chemical sensitization); or before coating. The compound is more preferably added from at the chemical sensitization step to before being mixed with non-photosensitive organic silver salt.

It is preferred that the compound of Groups 1 or 2 according to the invention is dissolved in water, a water-soluble solvent such as methanol and ethanol, or a mixed solvent thereof. In the case where the compound is dissolved in water and solubility of the compound is increased by increasing or decreasing a pH value of the solvent, the pH value may be increased or decreased to dissolve and add the compound.

The compound of Groups 1 or 2 according to the invention is preferably used in the image forming layer which contains the photosensitive silver halide and the non-photosensitive organic silver salt. The compound may be added to a surface protective layer, or an intermediate layer, as well as the image forming layer containing the photosensitive silver halide and the non-photosensitive organic silver salt, to be diffused to the image forming layer in the coating step. The compound may be added before or after addition of a sensitizing dye. Each compound is contained in the image forming layer preferably in an amount of from 1 × 10⁻⁹ mol to 5 × 10⁻¹ mol, more preferably from 1 × 10⁻⁸ mol to 5 × 10⁻² mol, per 1 mol of silver halide.

### 10) Compound having adsorptive group and reducing group

The photothermographic material of the present invention preferably comprises a compound having an adsorptive group to silver halide and a reducing group in a molecule. It is preferred that the compound is represented by the following formula (I).

Formula (I) A-(W)n-B

In formula (I), A represents a group capable of adsorption to a silver halide (hereafter, it is called an adsorptive group); W represents a divalent linking group; n represents 0 or 1; and B represents a reducing group.

In formula (I), the adsorptive group represented by A is a group to adsorb directly to a silver halide or a group to promote adsorption to a silver halide. As typical examples, a mercapto group (or a salt thereof), a thione group (-C(=S)-), a nitrogen atom, a heterocyclic group containing at least one atom selected from a nitrogen atom, a sulfur atom, a selenium atom, or a tellurium atom, a sulfide group, a disulfide group, a cationic group, an ethynyl group are described.

The mercapto group as an adsorptive group means a mercapto group (and a salt thereof) itself and simultaneously more preferably represents a heterocyclic group or an aryl group or an alkyl group substituted by at least one mercapto group (or a salt thereof). Herein, as the heterocyclic group, a monocyclic or a condensed aromatic or nonaromatic heterocyclic group having at least a 5 to 7-membered ring, for example, an imidazole ring group, a thiazole ring group, an oxazole ring group, a benzimidazole ring group, a benzothiazole ring group, a benzoxazole ring group, a triazole ring group, a thiadiazole ring group, an oxadiazole ring group, a tetrazole ring group, a purine ring group, a pyridine ring group, a quinoline ring group, an isoquinoline ring group, a pyrimidine ring group, a triazine ring group are described. A heterocyclic group having a quaternary nitrogen atom may also be adopted, wherein a mercapto group as a substituent may dissociate to form a mesoion. When the mercapto group forms a salt, a counter ion of the salt may be a cation of an alkaline metal, an alkaline earth metal, a heavy metal, such as Li⁺, Na⁺, K⁺, Mg²⁺, Ag⁺ and Zn²⁺; an ammonium ion; a heterocyclic group containing a quaternary nitrogen atom; a phosphonium ion.

Further, the mercapto group as an adsorptive group may become a thione group by a tautomerization.

The thione group used as the adsorptive group also include a linear or cyclic thioamide group, thiouredide group, thiourethane group, and dithiocarbamate ester group.

The heterocyclic group, as an adsorptive group, which contains at least one atom selected from a nitrogen atom, a sulfur atom, a selenium atom, or a tellurium atom represents a nitrogen-containing heterocyclic group having -NH- group, as a partial structure of a heterocycle, capable to form a silver iminate (>NAg) or a heterocyclic group, having an -S- group, a -Se- group, a -Te- group or a =N- group as a partial structure of a heterocycle, and capable to coordinate to a silver ion by a chelate bonding. As the former examples, a benzotriazole group, a triazole group, an indazole group, a pyrazole group, a tetrazole group, a benzimidazole group, an imidazole group, a purine group are described. As the latter examples, a thiophene group, a thiazole group, an oxazole group, a benzophthiophene group, a benzothiazole group, a benzoxazole group, a thiadiazole group, an oxadiazole group, a triazine group, a selenoazole group, a benzoselenazole group, a tellurazole group, a benzotellurazole group are described.

The sulfide group or disulfide group as an adsorptive group contains all groups having "-S-" or "-S-S-" as a partial structure.

The cationic group as an adsorptive group means the group containing a quaternary nitrogen atom, such as an ammonio group or a nitrogen-containing heterocyclic group including a quaternary nitrogen atom. As examples of the heterocyclic group containing a quaternary nitrogen atom, a pyridinio group, a quinolinio group, an isoquinolinio group, an imidazolio group are described.

The ethynyl group as an adsorptive group means -C≡CH group and the said hydrogen atom may be substituted.

The adsorptive group described above may have any substituent.

Further, as typical examples of an adsorptive group, the compounds described in pages 4 to 7 in the specification of JP-A No. 11-95355 are described.

As an adsorptive group represented by A in formula (I), a heterocyclic group substituted by a mercapto group (e.g., a 2-mercaptothiadiazole group, a 2-mercapto-5-aminothiadiazole group, a 3-mercapto-1,2,4-triazole group, a 5-mercaptotetrazole group, a 2-mercapto-1,3,4-oxadiazole group, a 2-mercaptobenzimidazole group, a 1,5-dimethyl-1,2,4-triazorium-3-thiolate group, a 2,4-dimercaptopyrimidine group, a 2,4- dimercaptotriazine group, a 3,5-dimercapto-1,2,4-triazole group, a 2,5-dimercapto-1,3-thiazole group and a nitrogen atom containing heterocyclic group having an -NH- group capable to form an imino-silver (>NAg) as a partial structure of heterocycle (e.g., a benzotriazole group, a benzimidazole group, an indazole group) are preferable, and more preferable as an adsorptive group are a 2-mercaptobenzimidazole group and a 3,5-dimercapto-1,2,4-triazole group.

In formula (I), W represents a divalent linking group. The said linking group may be any divalent linking group, as far as it does not give a bad effect toward photographic properties. For example, a divalent linking group which includes a carbon atom, a hydrogen atom, an oxygen atom, a nitrogen atom, or a sulfur atom, can be used. As typical examples, an alkylene group having 1 to 20 carbon atoms (e.g., a methylene group, an ethylene group, a trimethylene group, a tetramethylene group, a hexamethylene group), an alkenylene group having 2 to 20 carbon atoms, an alkynylene group having 2 to 20 carbon atoms, an arylene group having 6 to 20 carbon atoms (e.g., a phenylene group, a naphthylene group), -CO-, -SO₂-, -O-, -S-, -NR₁-, and the combinations of these linking groups are described. Herein, R₁ represents a hydrogen atom, an alkyl group, a heterocyclic group, or an aryl group.

The linking group represented by W may have any substituent.

In formula (I), a reducing group represented by B represents the group capable to reduce a silver ion. As the examples, a formyl group, an amino group, a triple bond group such as an acetylene group, a propargyl group, a mercapto group, and residues which are obtained by removing one hydrogen atom from hydroxylamines, hydroxamic acids, hydroxyureas, hydroxyurethanes, hydroxysemicarbazides, reductones (reductone derivatives are contained), anilines, phenols (chroman-6-ols, 2,3-dihydrobenzofuran-5-ols, aminophenols, sulfonamidophenols, and polyphenols such as hydroquinones, catechols, resorcinols, benzenetriols, bisphenols are included), acylhydrazines, carbamoylhydrazines, 3-pyrazolidones can be described. They may have any substituent.

The oxidation potential of a reducing group represented by B in formula (I), can be measured by using the measuring method described in Akira Fujishima, "DENKIKAGAKU SOKUTEIHO", pages 150 to 208, GIHODO SHUPPAN and The Chemical Society of Japan, "ZIKKEN KAGAKUKOZA", 4th ed., vol. 9, pages 282 to 344, MARUZEN. For example, the method of rotating disc voltammetry can be used; namely the sample is dissolved in the solution (methanol : pH 6.5 Britton-Robinson buffer = 10% : 90% (% by volume)) and after bubbling with nitrogen gas during 10 minutes the voltamograph can be measured under the conditions of 1000 rotations/minute, the sweep rate 20 mV/second, at 25°C by using a rotating disc electrode (RDE) made by glassy carbon as a working electrode, a platinum electrode as a counter electrode and a saturated calomel electrode as a reference electrode. The half wave potential (E1/2) can be calculated by that obtained voltamograph.

When a reducing group represented by B in the present invention is measured by the method described above, an oxidation potential is preferably in a range of from about -0.3 V to about 1.0 V, more preferably from - 0.1 V to 0.8 V, and particularly preferably from 0 V to 0.7 V.

In formula (I), a reducing group represented by B is preferably a residue which is obtained by removing one hydrogen atom from hydroxylamines, hydroxamic acids, hydroxyureas, hydroxysemicarbazides, reductones, phenols, acylhydrazines, carbamoylhydrazines, or 3-pyrazolidones.

The compound of formula (I) according to the present invention may have the ballasted group or polymer chain in it generally used in the non-moving photographic additives as a coupler. And as a polymer, for example, the polymer described in JP-A No. 1-100530 can be selected.

The compound of formula (I) according to the present invention may be bis or tris type of compound. The molecular weight of the compound represented by formula (I) according to the present invention is preferably from 100 to 10000, more preferably from 120 to 1000, and particularly preferably from 150 to 500.

The examples of the compound represented by formula (I) according to the present invention are shown below.

Further, example compounds 1 to 30 and 1"-1 to 1"-77 shown in EP No. 1308776A2, pages 73 to 87 are also described as preferable examples of the compound having an adsorptive group and a reducing group according to the invention.

These compounds can be easily synthesized by any known method. The compound of formula (I) in the present invention can be used alone, but it is preferred to use two or more kinds of the compounds in combination. When two or more kinds of the compounds are used in combination, those may be added to the same layer or the different layers, whereby adding methods may be different from each other.

The compound represented by formula (I) according to the present invention is preferably added to an image forming layer and more preferably is to be added at an emulsion preparing process. In the case, where these compounds are added at an emulsion preparing process, these compounds may be added at any step in the process. For example, the compounds may be added during the silver halide grain formation step, the step before starting of desalting step, the desalting step, the step before starting of chemical ripening, the chemical ripening step, the step before preparing a final emulsion. The compound can be added in several times during these steps. It is preferred to be added in the image forming layer. But the compound may be added to a surface protective layer or an intermediate layer, in combination with its addition to the image forming layer, to be diffused to the image forming layer in the coating step.

The preferred addition amount is largely dependent on the adding method described above or the kind of the compound, but generally from 1 × 10⁻⁶ mol to 1 mol, preferably from 1 × 10⁻⁵ mol to 5 × 10⁻¹ mol, and more preferably from 1 × 10⁻⁴ mol to 1 × 10⁻¹ mol, per 1 mol of photosensitive silver halide in each case.

The compound represented by formula (I) according to the present invention can be added by dissolving in water or water-soluble solvent such as methanol, ethanol or a mixed solution thereof. At this time, the pH may be arranged suitably by an acid or an alkaline and a surfactant can coexist. Further, these compounds can be added as an emulsified dispersion by dissolving them in an organic solvent having a high boiling point and also can be added as a solid dispersion.

### 11) Combined use of a plurality of silver halides

The photosensitive silver halide emulsion in the photothermographic material used in the invention may be used alone, or two or more kinds of them (for example, those of different average particle sizes, different halogen compositions, of different crystal habits and of different conditions for chemical sensitization) may be used together. Gradation can be controlled by using plural kinds of photosensitive silver halides of different sensitivity. The relevant techniques can include those described, for example, in JP-A Nos. 57-119341, 53-106125, 47-3929, 48-55730, 46-5187, 50-73627, and 57-150841. It is preferred to provide a sensitivity difference of 0.2 or more in terms of log E between each of the emulsions.

### 12) Coating amount

The addition amount of the photosensitive silver halide, when expressed by the amount of coated silver per 1 m² of the photothermographic material, is preferably from 0.03 g/m² to 0.6 g/m², more preferably, from 0.05 g/m² to 0.4 g/m² and, even more preferably, from 0.07 g/m² to 0.3 g/m². The photosensitive silver halide is used in a range of from 0.01 mol to 0.5 mol, preferably, from 0.02 mol to 0.3 mol, and even more preferably from 0.03 mol to 0.2 mol, per 1 mol of the organic silver salt.

### 13) Mixing photosensitive silver halide and organic silver salt

The method of mixing separately prepared the photosensitive silver halide and the organic silver salt can include a method of mixing prepared photosensitive silver halide grains and organic silver salt by a high speed stirrer, ball mill, sand mill, colloid mill, vibration mill, or homogenizer, or a method of mixing a photosensitive silver halide completed for preparation at any timing in the preparation of an organic silver salt and preparing the organic silver salt. The effect of the invention can be obtained preferably by any of the methods described above. Further, a method of mixing two or more kinds of aqueous dispersions of organic silver salts and two or more kinds of aqueous dispersions of photosensitive silver salts upon mixing is used preferably for controlling the photographic properties.

### 14) Mixing silver halide into coating solution

In the invention, the time of adding silver halide to the coating solution for the image forming layer is preferably in a range of from 180 minutes before to just prior to the coating, more preferably, 60 minutes s before to 10 seconds before coating. But there is no restriction for mixing method and mixing condition as long as the effect of the invention is sufficient. As an embodiment of a mixing method, there is a method of mixing in a tank and controlling an average residence time. The average residence time herein is calculated from addition flux and the amount of solution transferred to the coater. And another embodiment of mixing method is a method using a static mixer, which is described in 8th edition of "Ekitai Kongo Gijutu" by N. Harnby and M. F. Edwards, translated by Koji Takahashi (Nikkan Kogyo Shinbunsha, 1989).

### (Antifoggant)

As an antifoggant, stabilizer and stabilizer precursor usable in the invention, there can be mentioned those disclosed as patents in paragraph number 0070 of JP-A No. 10-62899 and in line 57 of page 20 to line 7 of page 21 of EP-A No. 0803764A1, the compounds described in JP-A Nos. 9-281637 and 9-329864, USP No. 6083681, and EP No. 1048975.

### 1) Organic polyhalogen compound

Preferable organic polyhalogen compound that can be used in the invention is explained specifically below. In the invention, preferred organic polyhalogen compound is the compound expressed by the following formula (H).

Formula (H) Q-(Y)n-C(Z₁)(Z₂)X

In formula (H), Q represents one selected from an alkyl group, an aryl group, or a heterocyclic group; Y represents a divalent linking group; n represents 0 or 1; Z₁ and Z₂ each represent a halogen atom; and X represents a hydrogen atom or an electron-attracting group.

In formula (H), Q is preferably an alkyl group having 1 to 6 carbon atoms, an aryl group having 6 to 12 carbon atoms, or a heterocyclic group comprising at least one nitrogen atom (pyridine, quinoline).

In the case where Q is an aryl group in formula (H), Q preferably is a phenyl group substituted by an electron-attracting group whose Hammett substituent constant σp yields a positive value. For the details of Hammett substituent constant, reference can be made to Journal of Medicinal Chemistry, vol. 16, No. 11 (1973), pp. 1207 to 1216. As such electron-attracting groups, examples include, halogen atoms, an alkyl group substituted by an electron-attracting group, an aryl group substituted by an electron-attracting group, a heterocyclic group, an alkylsulfonyl group, an arylsulfonyl group, an acyl group, an alkoxycarbonyl group, a carbamoyl group, sulfamoyl group. Preferable as the electron-attracting group is a halogen atom, a carbamoyl group, or an arylsulfonyl group, and particularly preferred among them is a carbamoyl group.

X is preferably an electron-attracting group. As the electron-attracting group, preferable are a halogen atom, an aliphatic arylsulfonyl group, a heterocyclic sulfonyl group, an aliphatic arylacyl group, a heterocyclic acyl group, an aliphatic aryloxycarbonyl group, a heterocyclic oxycarbonyl group, a carbamoyl group, and a sulfamoyl group; more preferable are a halogen atom and a carbamoyl group; and particularly preferable is a bromine atom.

Z₁ and Z₂ each are preferably a bromine atom or an iodine atom, and more preferably, a bromine atom.

Y preferably represents -C(=O)-, -SO-, -SO₂-, -C(=O)N(R)-, or - SO₂N(R)-; more preferably, -C(=O)-, -SO₂-, or -C(=O)N(R)-; and particularly preferably, -SO₂- or -C(=O)N(R)-. Herein, R represents a hydrogen atom, an aryl group, or an alkyl group, preferably a hydrogen atom or an alkyl group, and particularly preferably a hydrogen atom.

n represents 0 or 1, and is preferably 1.

In formula (H), in the case where Q is an alkyl group, Y is preferably -C(=O)N(R)-. And, in the case where Q is an aryl group or a heterocyclic group, Y is preferably -SO₂-.

In formula (H), the form where the residues, which are obtained by removing a hydrogen atom from the compound, bind to each other (generally called bis type, tris type, or tetrakis type) is also preferably used.

In formula (H), the form having a substituent of a dissociative group (for example, a COOH group or a salt thereof, an SO₃H group or a salt thereof, a PO₃H group or a salt thereof like), a group containing a quaternary nitrogen cation (for example, an ammonium group, a pyridinium group, or the like), a polyethyleneoxy group, a hydroxy group is also preferable.

Specific examples of the compound expressed by formula (H) are shown below.

As preferred organic polyhalogen compounds used in the invention other than those above, there can be mentioned compounds disclosed in USP Nos. 3874946, 4756999, 5340712, 5369000, 5464737, and 6506548, JP-A Nos. 50-137126, 50-89020, 50-119624, 59-57234, 7-2781, 7-5621, 9-160164, 9-244177, 9-244178, 9-160167, 9-319022, 9-258367, 9-265150, 9-319022, 10-197988, 10-197989, 11-242304, 2000-2963, 2000-112070, 2000-284410, 2000-284412, 2001-33911, 2001-31644, 2001-312027, and 2003-50441. Particularly, compounds disclosed in JP-A Nos. 7-2781, 2001-33911 and 20001-312027 are preferable.

The compound expressed by formula (H) of the invention is preferably used in an amount of from 10⁻⁴ mol to 1 mol, more preferably, from 10⁻³ mol to 0.5 mol, and further preferably, from 1 × 10⁻² mol to 0.2 mol, per 1 mol of non-photosensitive silver salt incorporated in the image forming layer.

In the invention, usable methods for incorporating the antifoggant into the photothermographic material are those described above in the method for incorporating the reducing agent, and also for the organic polyhalogen compound, it is preferably added in the form of a solid fine particle dispersion.

### 2) Other antifoggants

As other antifoggants, there can be mentioned a mercury (II) salt described in paragraph number 0113 of JP-A No. 11-65021, benzoic acids described in paragraph number 0114 of the same literature, a salicylic acid derivative described in JP-A No. 2000-206642, a formaline scavenger compound expressed by formula (S) in JP-A No. 2000-221634, a triazine compound related to Claim 9 of JP-A No. 11-352624, a compound expressed by formula (III), 4-hydroxy-6-methyl-1,3,3a,7-tetrazaindene, described in JP-A No. 6-11791.

The photothermographic material of the invention may further contain an azolium salt in order to prevent fogging. Azolium salts useful in the present invention include a compound expressed by formula (XI) described in JP-A No. 59-193447, a compound described in Japanese Patent Application Publication (JP-B) No. 55-12581, and a compound expressed by formula (II) in JP-A No. 60-153039. The azolium salt may be added to any part of the photothermographic material, but as an additional layer, it is preferred to select a layer on the side having thereon the image forming layer, and more preferred is to select the image forming layer itself. The azolium salt may be added at any time of the process of preparing the coating solution; in the case where the azolium salt is added into the image forming layer, any time of the process may be selected, from the preparation of the organic silver salt to the preparation of the coating solution, but preferred is to add the salt after preparing the organic silver salt and just before coating. As the method for adding the azolium salt, any method using a powder, a solution, a fine-particle dispersion, may be used. Furthermore, it may be added as a solution having mixed therein other additives such as sensitizing agents, reducing agents, toners. In the invention, the azolium salt may be added at any amount, but preferably, it is added in a range of from 1 × 10⁻⁶ mol to 2 mol, and more preferably, from 1 × 10⁻³ mol to 0.5 mol, per 1 mol of silver.

### (Other additives)

### 1) Mercapto compounds, disulfides and thiones

In the invention, mercapto compounds, disulfide compounds, and thione compounds can be added in order to control the development by suppressing or enhancing development, to improve spectral sensitization efficiency, and to improve storage properties before and after development. Descriptions can be found in paragraph numbers 0067 to 0069 of JP-A No. 10-62899, a compound expressed by formula (I) of JP-A No. 10-186572 and specific examples thereof shown in paragraph numbers 0033 to 0052, in lines 36 to 56 in page 20 of EP No. 0803764A1. Among them, mercapto-substituted heterocyclic aromatic compounds described in JP-A Nos. 9-297367, 9-304875, 2001-100358, 2002-303954, 2002-303951 are preferred.

### 2) Toner

In the photothermographic material of the present invention, the addition of a toner is preferred. The description of the toner can be found in JP-A No.10-62899 (paragraph numbers 0054 to 0055), EP No.0803764A1 (page21, lines 23 to 48), JP-A Nos.2000-356317 and 2000-187298. Preferred are phthalazinones (phthalazinone, phthalazinone derivatives and metal salts thereof, (e.g., 4-(1-naphthyl)phthalazinone, 6-chlorophthalazinone, 5,7-dimethoxyphthalazinone, and 2,3-dihydro-1,4-phthalazinedione); combinations of phthalazinones and phthalic acids (e.g., phthalic acid, 4-methylphthalic acid, 4-nitrophthalic acid, diammonium phthalate, sodium phthalate, potassium phthalate, and tetrachlorophthalic anhydride); phthalazines (phthalazine, phthalazine derivatives and metal salts thereof, (e.g., 4-(1-naphthyl)phthalazine, 6-isopropylphthalazine, 6-tert-butylphthalazine, 6-chlorophthalazine, 5,7-dimethoxyphthalazine, and 2,3-dihydrophthalazine); combinations of phthalazines and phthalic acids. Particularly preferred is a combination of phthalazines and phthalic acids. Among them, particularly preferable are the combination of 6-isopropylphthalazine and phthalic acid, and the combination of 6-isopropylphthalazine and 4-methylphthalic acid.

### 3) Plasticizer and lubricant

In the invention, well-known plasticizer and lubricant can be used to improve physical properties of film. Particularly, to improve handling facility during manufacturing process or scratch resistance during thermal development, it is preferred to use a lubricant such as a liquid paraffin, a long chain fatty acid, an amide of fatty acid, an ester of fatty acid and the like. Paticularly preferred are a liquid paraffin obtained by removing components having low boiling point and an ester of fatty acid having a branch structure and a molecular weight of 1000 or more.

Concerning plasticizers and lubricants usable in the image forming layer and in the non-photosensitive layer, compounds described in paragraph No. 0117 of JP-A No. 11-65021 and in JP-A Nos. 2000-5137, 2004-219794, 2004-219802, and 2004-334077 are preferable.

### 4) Dyes and pigments

From the viewpoint of improving color tone, preventing the generation of interference fringes and preventing irradiation on laser exposure, various kinds of dyes and pigments (for instance, C.I. Pigment Blue 60, C.I. Pigment Blue 64, and C.I. Pigment Blue 15:6) can be used in the image forming layer used in the invention. Detailed description can be found in WO No. 98/36322, JP-A Nos. 10-268465 and 11-338098, and the like.

### 5) Nucleator

Concerning the photothermographic material used in the invention, it is preferred to add a nucleator into the image forming layer. Details on the nucleators, method for their addition and addition amount can be found in paragraph No. 0118 of JP-A No. 11-65021, paragraph Nos. 0136 to 0193 of JP-A No. 11-223898, as compounds expressed by formulae (H), (1) to (3), (A), and (B) in JP-A No. 2000-284399; as for a nucleation accelerator, description can be found in paragraph No. 0102 of JP-A No. 11-65021, and in paragraph Nos. 0194 to 0195 of JP-A No. 11-223898.

In the case of using formic acid or formates as a strong fogging agent, it is preferably incorporated into the side having thereon the image forming layer containing photosensitive silver halide at an amount of 5 mmol or less, and more preferably 1 mmol or less, per 1 mol of silver.

In the case of using a nucleator in the photothermographic material used in the invention, it is preferred to use an acid resulting from hydration of diphosphorus pentaoxide, or a salt thereof in combination. Acids resulting from the hydration of diphosphorus pentaoxide or salts thereof include metaphosphoric acid (salt), pyrophosphoric acid (salt), orthophosphoric acid (salt), triphosphoric acid (salt), tetraphosphoric acid (salt), hexametaphosphoric acid (salt). Particularly preferred acids obtainable by the hydration of diphosphorus pentaoxide or salts thereof include orthophosphoric acid (salt) and hexametaphosphoric acid (salt). Specifically mentioned as the salts are sodium orthophosphate, sodium dihydrogen orthophosphate, sodium hexametaphosphate, ammonium hexametaphosphate

The addition amount of the acid obtained by hydration of diphoshorus pentaoxide or the salt thereof (i.e., the coating amount per 1 m² of the photothermographic material) may be set as desired depending on sensitivity and fogging, but preferred is an amount of from 0.1 mg/m² to 500 mg/m², and more preferably, from 0.5 mg/m² to 100 mg/m².

### (Preparation of coating solution and coating)

The temperature for preparing the coating solution for the image forming layer used in the invention is preferably from 30°C to 65°C, more preferably, 35°C or more and less than 60°C, and further preferably, from 35°C to 55°C. Furthermore, the temperature of the coating solution for the image forming layer immediately after adding the polymer latex is preferably maintained in the temperature range from 30°C to 65°C.

### (Layer constitution and constituting components)

The photothermographic material used in the invention has one or more image forming layers constructed on a support. In the case of constituting the image forming layer from one layer, the image forming layer comprises an organic silver salt, a photosensitive silver halide, a reducing agent, and a binder, and may further comprise additional materials as desired and necessary, such as an antifoggant, a toner, a film-forming promoting agent, and other auxiliary agents. In the case of constituting the image forming layer from two or more layers, the first image forming layer (in general, a layer placed nearer to the support) contains an organic silver salt and a photosensitive silver halide. Some of the other components are incorporated in the second image forming layer or in both of the layers.

The photothermographic material according to the invention has a non-photosensitive layer in addition to the image forming layer. In general, non-photosensitive layers can be classified depending on the layer arrangement into (a) a surface protective layer provided on the image forming layer (on the side farther from the support), (b) an intermediate layer provided among plural image forming layers or between the image forming layer and the protective layer, (c) an undercoat layer provided between the image forming layer and the support, and (d) a back layer which is provided on the side opposite to the image forming layer.

Furthermore, a layer that functions as an optical filter may be provided as (a) or (b) above. An antihalation layer may be provided as (c) or (d) to the photothermographic material.

### 1) Surface protective layer

The photothermographic material of the invention may further comprise a surface protective layer with an object to prevent adhesion of the image forming layer. The surface protective layer may be a single layer, or plural layers.

Description on the surface protective layer may be found in paragraph Nos. 0119 to 0120 of JP-A No. 11-65021 and in JP-A No. 2000-171936.

Preferred as the binder of the surface protective layer used in the invention is gelatin, but poly(vinyl alcohol) (PVA) may be used preferably instead, or in combination. As gelatin, there can be used an inert gelatin (e.g., Nitta gelatin 750), a phthalated gelatin (e.g., Nitta gelatin 801). Usable as PVA are those described in paragraph Nos. 0009 to 0020 of JP-A No. 2000-171936, and preferred are the completely saponified product PVA-105, the partially saponified PVA-205, and PVA-335, as well as modified poly(vinyl alcohol) MP-203 (all trade name of products from Kuraray Ltd.). The amount of coated poly(vinyl alcohol) (per 1 m² of support) in the surface protective layer (per one layer) is preferably in a range from 0.3 g/m² to 4.0 g/m², and more preferably, from 0.3 g/m² to 2.0 g/m².

The total amount of the coated binder (including water-soluble polymer and latex polymer) (per 1 m² of support) in the surface protective layer (per one layer) is preferably in a range from 0.3 g/m² to 5.0 g/m², and more preferably, from 0.3 g/m² to 2.0 g/m².

Further, it is preferred to use a lubricant such as a liquid paraffin and an ester of fatty acid in the surface protective layer. The addition amount of the lubricant is in a range of from 1 mg/m² to 200 mg/m², preferably 10 mg/m² to 150 mg/m² and, more preferably 20 mg/m² to 100 mg/m².

### 2) Antihalation layer

The photothermographic material of the present invention can comprise an antihalation layer provided to the side farther from the light source than the image forming layer.

Descriptions on the antihalation layer can be found in paragraph Nos. 0123 to 0124 of JP-A No. 11-65021, in JP-A Nos. 11-223898, 9-230531, 10-36695, 10-104779, 11-231457, 11-352625, 11-352626.

The antihalation layer contains an antihalation dye having its absorption at the wavelength of the exposure light. In the case where the exposure wavelength is in the infrared region, an infrared-absorbing dye may be used, and in such a case, preferred are dyes having no absorption in the visible region.

In the case of preventing halation from occurring by using a dye having absorption in the visible region, it is preferred that the color of the dye would not substantially reside after image formation, and is preferred to employ a means for bleaching color by the heat of thermal development; in particular, it is preferred to add a thermal bleaching dye and a base precursor to the non-photosensitive layer to impart function as an antihalation layer. Those techniques are described in JP-A No. 11-231457.

The addition amount of the thermal bleaching dye is determined depending on the usage of the dye. In general, it is used at an amount as such that the optical density (absorbance) exceeds 0.1 when measured at the desired wavelength. The optical density is preferably in a range of from 0.15 to 2, and more preferably from 0.2 to 1. The addition amount of dyes to obtain optical density in the above range is generally from 0.001 g/m² to 1 g/m².

By decoloring the dye in such a manner, the optical density after thermal development can be lowered to 0.1 or lower. Two or more types of thermal bleaching dyes may be used in combination in a photothermographic material. Similarly, two or more types of base precursors may be used in combination.

In the case of thermal decolorization by the combined use of a decoloring dye and a base precursor, it is advantageous from the viewpoint of thermal decoloring efficiency to further use a substance capable of lowering the melting point by at least 3°C when mixed with the base precursor (e.g., diphenylsulfone, 4-chlorophenyl(phenyl)sulfone, 2-naphthylbenzoate, or the like) as disclosed in JP-A No. 11-352626.

### 3) Back layer

Back layers usable in the invention are described in paragraph Nos. 0128 to 0130 of JP-A No. 11-65021.

In the invention, coloring matters having maximum absorption in the wavelength range from 300 nm to 450 nm can be added in order to improve color tone of developed silver images and a deterioration of the images during aging. Such coloring matters are described in, for example, JP-A Nos. 62-210458, 63-104046, 63-103235, 63-208846, 63-306436, 63-314535, 01-61745, 2001-100363.

Such coloring matters are generally added in a range of from 0.1 mg/m² to 1 g/m², preferably to the back layer which is provided on the side opposite to the image forming layer.

Further, in order to control the basic color tone, it is preferred to use a dye having an absorption peak in a wavelength range from 580 nm to 680 nm. As a dye satisfying this purpose, preferred are oil-soluble azomethine dyes described in JP-A Nos. 4-359967 and 4-359968, or water-soluble phthalocyanine dyes described in JP-A No. 2003-295388, which have low absorption intensity on the short wavelength side. The dyes for this purpose may be added to any of the layers, but more preferred is to add them in the non-photosensitive layer on the image forming layer side, or in the backside.

The photothermographic material used in the invention is preferably a so-called single-sided photosensitive material, which comprises at least one layer of a image forming layer containing silver halide emulsion on one side of the support, and a back layer on the other side.

### 4) Matting agent

A matting agent is preferably added to the photothermographic material of the invention in order to improve transportability. Description on the matting agent can be found in paragraphs Nos. 0126 to 0127 of JP-A No.11-65021. The addition amount of the matting agent is preferably in a range from 1 mg/m² to 400 mg/m², and more preferably, from 5 mg/m² to 300 mg/m², with respect to the coating amount per 1 m² of the photothermographic material.

The shape of the matting agent usable in the invention may fixed form or non-fixed form. Preferred is to use those having fixed form and globular shape.

Volume weighted mean equivalent spherical diameter of the matting agent used in the image forming layer surface is preferably in a range of from 0.3 µm to 10 µm, and more preferably, from 0.5 µm to 7 µm. Further, the particle distribution of the matting agent is preferably set as such that the variation coefficient becomes from 5% to 80%, and more preferably, from 20% to 80%. The variation coefficient, herein, is defined by (the standard deviation of particle diameter)/(mean diameter of the particle) × 100. Furthermore, two or more kinds of matting agents having different mean particle size can be used in the image forming layer surface. In this case, it is preferred that the difference between the mean particle size of the biggest matting agent and the mean particle size of the smallest matting agent is from 2 µm to 8 µm, and more preferred, from 2 µm to 6 µm.

Volume weighted mean equivalent spherical diameter of the matting agent used in the back surface is preferably in a range from 1 µm to 15 µm, and more preferably, from 3 µm to 10 µm. Further, the particle distribution of the matting agent is preferably set as such that the variation coefficient may become from 3% to 50%, and more preferably, from 5% to 30%. Furthermore, two or more kinds of matting agents having different mean particle size can be used in the back surface. In this case, it is preferred that the difference between the mean particle size of the biggest matting agent and the mean particle size of the smallest matting agent is from 2 µm to 14 µm, and more preferred, from 2 µm to 9 µm.

The level of matting on the image forming layer surface is not restricted as far as star-dust trouble occurs, but the level of matting of 30 seconds to 2000 seconds is preferred, particularly preferred, 40 seconds to 1500 seconds as Beck's smoothness. Beck's smoothness can be calculated easily, using Japan Industrial Standared (JIS) P8119 "The method of testing Beck's smoothness for papers and sheets using Beck's test apparatus", or TAPPI standard method T479.

The level of matting of the back layer in the invention is preferably in a range of 1200 seconds or less and 10 seconds or more; more preferably, 800 seconds or less and 20 seconds or more; and even more preferably, 500 seconds or less and 40 seconds or more when expressed by Beck's smoothness.

In the present invention, a matting agent is preferably contained in an outermost layer, in a layer which can function as an outermost layer, or in a layer nearer to outer surface, and also preferably is contained in a layer which can function as a so-called protective layer.

### 5) Polymer latex

A polymer latex is preferably used in the surface protective layer and the back layer of the photothermographic material in the present invention. As such polymer latex, descriptions can be found in "Gosei Jushi Emulsion (Synthetic resin emulsion)" (Taira Okuda and Hiroshi Inagaki, Eds., published by Kobunshi Kankokai (1978)), "Gosei Latex no Oyo (Application of synthetic latex)" (Takaaki Sugimura, Yasuo Kataoka, Soichi Suzuki, and Keiji Kasahara, Eds., published by Kobunshi Kankokai (1993)), and "Gosei Latex no Kagaku (Chemistry of synthetic latex)" (Soichi Muroi, published by Kobunshi Kankokai (1970)). More specifically, there can be mentioned a latex of methyl methacrylate (33.5% by weight)/ ethyl acrylate (50% by weight)/ methacrylic acid (16.5% by weight) copolymer, a latex of methyl methacrylate (47.5% by weight)/ butadiene (47.5% by weight)/ itaconic acid (5% by weight) copolymer, a latex of ethyl acrylate/ methacrylic acid copolymer, a latex of methyl methacrylate (58.9% by weight)/ 2-ethylhexyl acrylate (25.4% by weight)/ styrene (8.6% by weight)/ 2-hydroethyl methacrylate (5.1% by weight)/ acrylic acid (2.0% by weight) copolymer, a latex of methyl methacrylate (64.0% by weight)/ styrene (9.0% by weight)/butyl acrylate (20.0% by weight)/ 2-hydroxyethyl methacrylate (5.0% by weight)/ acrylic acid (2.0% by weight) copolymer

Furthermore, as the binder for the surface protective layer, there can be applied the technology described in paragraph Nos. 0021 to 0025 of the specification of JP-A No. 2000-267226, and the technology described in paragraph Nos. 0023 to 0041 of the specification of JP-A No. 2000-19678. The polymer latex in the surface protective layer is preferably contained in an amount of from 10% by weight to 90% by weight, particularly preferably from 20% by weight to 80% by weight, of the total weight of binder.

### 6) Surface pH

The surface pH of the photothermographic material according to the invention preferably yields a pH of 7.0 or lower, and more preferably 6.6 or lower, before thermal developing process. Although there is no particular restriction concerning the lower limit, the lower limit of pH value is about 3. The most preferred surface pH range is from 4 to 6.2. From the viewpoint of reducing the surface pH, it is preferred to use an organic acid such as phthalic acid derivative or a non-volatile acid such as sulfuric acid, or a volatile base such as ammonia for the adjustment of the surface pH. In particular, ammonia can be used favorably for the achievement of low surface pH, because it can easily vaporize to remove it before the coating step or before applying thermal development. It is also preferred to use a non-volatile base such as sodium hydroxide, potassium hydroxide, lithium hydroxide, and the like, in combination with ammonia. The method of measuring surface pH value is described in paragraph No. 0123 of the specification of JP-A No. 2000-284399.

### 7) Hardener

A hardener may be used in each of image forming layer, protective layer, back layer, used in the invention. As examples of the hardener, descriptions of various methods can be found in pages 77 to 87 of T. H. James, "THE THEORY OF THE PHOTOGRAPHIC PROCESS, FOURTH EDITION" (Macmillan Publishing Co., Inc., 1977). Preferably used are, in addition to chromium alum, sodium salt of 2,4-dichloro-6-hydroxy-s-triazine, N,N-ethylene bis(vinylsulfonacetamide), and N,N-propylene bis(vinylsulfonacetamide), polyvalent metal ions described in page 78 of the above literature, polyisocyanates described in USP No. 4,281,060, JP-A No. 6-208193, epoxy compounds of USP No. 4,791,042, and vinylsulfone compounds of JP-A No. 62-89048.

The hardener is added as a solution, and the solution is added to a coating solution 180 minutes before coating to just before coating, preferably 60 minutes before to 10 seconds before coating. However, so long as the effect of the invention is sufficiently exhibited, there is no particular restriction concerning the mixing method and the conditions of mixing. As specific mixing methods, there can be mentioned a method of mixing in the tank, in which the average stay time calculated from the flow rate of addition and the feed rate to the coater is controlled to yield a desired time, or a method using static mixer as described in Chapter 8 of N. Harnby, M. F. Edwards, A. W. Nienow (translated by Koji Takahashi) "Ekitai Kongo Gijutu (Liquid Mixing Technology)" (Nikkan Kogyo Shinbunsha, 1989).

### 8) Surfactant

Concerning the surfactant, the solvent, the support, antistatic agent and the electrically conductive layer, and the method for obtaining color images applicable in the invention, there can be used those disclosed in paragraph numbers 0132, 0133, 0134, 0135, and 0136, respectively, of JP-A No. 11-65021. Concerning lubricants, there can be used those disclosed in paragraph numbers 0061 to 0064 of JP-A No. 11-84573 and in paragraph numbers 0049 to 0062 of JP-A No. 2001-83679.

In the invention, it is preferred to use a fluorocarbon surfacant. Specific examples of fluorocarbon surfacants can be found in those described in JP-A Nos. 10-197985, 2000-19680, and 2000-214554. Polymer fluorocarbon surfacants described in JP-A 9-281636 can be also used preferably.

For the photothermographic material in the invention, the fluorocarbon surfacants described in JP-A Nos. 2002-82411, 2003-57780, and 2003-149766 are preferably used. Especially, the usage of the fluorocarbon surfacants described in JP-A Nos. 2003-57780 and 2003-149766 in an aqueous coating solution is preferred viewed from the standpoint of capacity in static control, stability of the coated surface state and sliding facility. The fluorocarbon surfactant described in JP-A No. 2003-149766 is preferred because of high capacity in static control and that it needs small amount to use. A fluorocarbon compound which has two or more fluoroalkyl groups having two or more carbon atoms and 11 or fewer fluorine atoms, and at least one of an anionic or nonionic hydrophilic group is more preferred. Most preferred is the compound represented by formula (A) described in JP-A No. 2003-149766, and specifically, the compounds (FS-1) to (FS-66) described in JP-A No. 2003-149766.

According to the invention, the fluorocarbon surfactant can be used on either side of image forming layer side or backside, but is preferred to use on the both sides. Further, it is particularly preferred to use in combination with electrically conductive layer including metal oxides described below. In this case the amount of the fluorocarbon surfactant on the side of the electrically conductive layer can be reduced or removed.

The addition amount of the fluorocarbon surfactant is preferably in a range of from 0.1 mg/m² to 100 mg/m² on each side of image forming layer and back layer, more preferably from 0.3 mg/m² to 30 mg/m², and even more preferably from 1 mg/m² to 10 mg/m². Especially, the fluorocarbon surfactant described in JP-A No. 2003-149766 is effective, and used preferably in a range of from 0.01 mg/m² to 10 mg/m², and more preferably from 0.1 mg/m² to 5 mg/m².

### 9) Antistatic agent

The photothermographic material used in the invention preferably contains an electrically conductive layer including metal oxides or electrically conductive polymers. The antistatic layer may serve as an undercoat layer, or a back surface protective layer, but can also be placed specially. As an electrically conductive material of the antistatic layer, metal oxides having enhanced electric conductivity by the method of introducing oxygen defects or different types of metallic atoms into the metal oxides are preferable for use. Examples of metal oxides are preferably selected from ZnO, TiO₂, or SnO₂. As the combination of different types of atoms, preferred are ZnO combined with A1, or In; SnO₂ with Sb, Nb, P, halogen atoms; TriO₂ with Nb, Ta.

Particularly preferred for use is SnO₂ combined with Sb. The addition amount of different types of atoms is preferably in a range of from 0.01 mol% to 30 mol%, and more preferably, in a range of from 0.1 mol% to 10 mol%. The shape of the metal oxides can include, for example, spherical, needle-like, or tabular. The needle-like particles, with the rate of (the major axis)/(the minor axis) is 2.0 or more, and more preferably in a range of from 3.0 to 50, is preferred viewed from the standpoint of the electric conductivity effect. The metal oxides is preferably used in a range of from 1 mg/m² to 1000 mg/m², more preferably from 10 mg/m² to 500 mg/m², and even more preferably from 20 mg/m² to 200 mg/m².

The antistatic layer can be laid on either side of the image forming layer side or the backside, it is preferred to set between the support and the back layer. Specific examples of the antistatic layer in the invention include described in paragraph Nos. 0135 of JP-A No. 11-65021, in JP-A Nos. 56-143430, 56-143431, 58-62646, and 56-120519, and in paragraph Nos. 0040 to 0051 of JP-A No. 11-84573, in USP No. 5,575,957, and in paragraph Nos. 0078 to 0084 of JP-A No. 11-223898.

### 10) Support

As the transparent support, preferably used is polyester, particularly, polyethylene terephthalate, which is subjected to heat treatment in the temperature range of from 130°C to 185°C in order to relax the internal strain caused by biaxial stretching and remaining inside the film, and to remove strain ascribed to heat shrinkage generated during thermal development. In the case of a photothermographic material for medical use, the transparent support may be colored with a blue dye (for instance, dye-1 described in the Example of JP-A No. 8-240877), or may be uncolored. As to the support, it is preferred to apply undercoating technology, such as water-soluble polyester described in JP-A No. 11-84574, a styrene-butadiene copolymer described in JP-A No. 10-186565, a vinylidene chloride copolymer described in JP-A No. 2000-39684. The moisture content of the support is preferably 0.5% by weight or lower when coating for image forming layer and back layer is conducted on the support.

### 11) Other additives

Furthermore, an antioxidant, stabilizing agent, plasticizer, UV absorbent, or film-forming promoting agent may be added to the photothermographic material. Each of the additives is added to either of the image forming layer or the non-photosensitive layer. Reference can be made to WO No. 98/36322, EP No. 803764A1, JP-A Nos. 10-186567 and 10-18568.

### 12) Coating method

The photothermographic material used in the invention may be coated by any method. Specifically, various types of coating operations including extrusion coating, slide coating, curtain coating, immersion coating, knife coating, flow coating, or an extrusion coating using the type of hopper described in USP No. 2,681,294 are used. Preferably used is extrusion coating or slide coating described in pages 399 to 536 of Stephen F. Kistler and Petert M. Shweizer, "LIQUID FILM COATING" (Chapman & Hall, 1997), and particularly preferably used is slide coating. Example of the shape of the slide coater for use in slide coating is shown in Figure 11b.1, page 427, of the same literature. If desired, two or more layers can be coated simultaneously by the method described in pages 399 to 536 of the same literature, or by the method described in USP No. 2,761,791 and British Patent No. 837,095. Particularly preferred in the invention is the method described in JP-A Nos. 2001-194748, 2002-153808, 2002-153803, and 2002-182333.

The coating solution for the image forming layer in the invention is preferably a so-called thixotropic fluid. For the details of this technology, reference can be made to JP-A No. 11-52509. Viscosity of the coating solution for the image forming layer in the invention at a shear velocity of 0.1S⁻¹ is preferably from 400 mPa·s to 100,000 mPa·s, and more preferably, from 500 mPa·s to 20,000 mPa·s. At a shear velocity of 1000S⁻¹, the viscosity is preferably from 1 mPa·s to 200 mPa·s, and more preferably, from 5 mPa·s to 80 mPa·s.

In the case of mixing two types of liquids on preparing the coating solution used in the invention, known in-line mixer and in-plant mixer can be used favorably. Preferred in-line mixer of the invention is described in JP-A No. 2002-85948, and the in-plant mixer is described in JP-A No. 2002-90940.

The coating solution used in the invention is preferably subjected to defoaming treatment to maintain the coated surface in a fine state. Preferred defoaming treatment method in the invention is described in JP-A No. 2002-66431.

In the case of applying the coating solution used in the invention to the support, it is preferred to perform diselectrification in order to prevent the adhesion of dust, particulates due to charge up. Preferred example of the method of diselectrification for use in the invention is described in JP-A No. 2002-143747.

Since a non-setting coating solution is used for the image forming layer in the invention, it is important to precisely control the drying wind and the drying temperature. Preferred drying method for use in the invention is described in detail in JP-A Nos. 2001-194749 and 2002-139814.

In order to improve the film-forming properties in the photothermographic material used in the invention, it is preferred to apply a heat treatment immediately after coating and drying. The temperature of the heat treatment is preferably in a range of from 60°C to 100°C at the film surface, and time period for heating is preferably in a range of from 1 second to 60 seconds. More preferably, heating is performed in a temperature range of from 70°C to 90°C at the film surface, and the time period for heating is from 2 seconds to 10 seconds. A preferred method of heat treatment for the invention is described in JP-A No. 2002-107872.

Furthermore, the producing methods described in JP-A Nos. 2002-156728 and 2002-182333 are favorably used in the invention in order to stably and successively produce the photothermographic material used in the invention.

The photothermographic material is preferably of mono-sheet type (i.e., a type which can form image on the photothermographic material without using other sheets such as an image-receiving material).

### 13) Wrapping material.

In order to suppress fluctuation from occurring on the photographic property during a preservation of the photothermographic material used in the invention before thermal development, or in order to improve curling or winding tendencies when the photothermographic material is manufactured in a roll state, it is preferred that a wrapping material having low oxygen transmittance and/or vapor transmittance is used. Preferably, oxygen transmittance is 50 mL·atm⁻¹m⁻²day⁻¹ or lower at 25°C, more preferably, 10 mL·atm⁻¹m⁻²day⁻¹ or lower, and even more preferably, 1.0 mL·atm⁻¹m⁻²day⁻¹ or lower. Preferably, vapor transmittance is 10 g·atm⁻¹m⁻²day⁻¹ or lower, more preferably, 5 g·atm⁻¹m⁻²day⁻¹ or lower, and even more preferably, 1 g. atm⁻¹m⁻²day⁻¹ or lower.

As specific examples of a wrapping material having low oxygen transmittance and/or vapor transmittance, reference can be made to, for instance, the wrapping material described in JP-A Nos.8-254793 and 2000-206653.

### 14) Other applicable techniques

Techniques which can be used for the photothermographic material of the invention also include those in EP No. 803764A1, EP No. 883022A1, WO No. 98/36322, JP-A Nos. 56-62648, and 58-62644, JP-A Nos. 09-43766, 09-281637, 09-297367, 09-304869, 09-311405, 09-329865, 10-10669, 10-62899, 10-69023, 10-186568, 10-90823, 10-171063, 10-186565, 10-186567, 10-186569 to 10-186572, 10-197974, 10-197982, 10-197983, 10-197985 to 10-197987, 10-207001, 10-207004, 10-221807, 10-282601, 10-288823, 10-288824, 10-307365, 10-312038, 10-339934, 11-7100, 11-15105, 11-24200, 11-24201, 11-30832, 11-84574, 11-65021, 11-109547, 11-125880, 11-129629, 11-133536 to 11-133539, 11-133542, 11-133543, 11-223898, 11-352627, 11-305377, 11-305378, 11-305384, 11-305380, 11-316435, 11-327076, 11-338096, 11-338098, 11-338099, 11-343420, 2001-200414, 2001-234635, 2002-020699, 2001-275471, 2001-275461, 2000-313204, 2001-292844, 2000-324888, 2001-293864, 2001-348546, and 2000-187298.

In the case of multicolor photothermographic material, each of the image forming layers is maintained distinguished from each other by incorporating functional or non-functional barrier layer between each of the image forming layers as described in USP No. 4,460,681.

The constitution of a multicolor photothermographic material may include combinations of two layers for those for each of the colors, or may contain all the components in a single layer as described in USP No. 4,708,928.

### (Image forming method)

### 1) Imagewise exposure

The photothermographic material of the invention may be subjected to imagewise exposure by any known methods.

Preferred is scanning exposure using laser beam. As laser beam, He-Ne laser of red through infrared emission, red laser diode, or Ar⁺, He-Ne, He-Cd laser of blue through green emission, or blue laser diode can be used. Preferred is red to infrared laser diode and the peak wavelength of laser beam is 600 nm to 900 nm, and preferably 620 nm to 850 nm.

In recent years, development has been made particularly on a light source module with an SHG (a second harmonic generator) and a laser diode integrated into a single piece whereby a laser output apparatus in a short wavelength region has become popular. A blue laser diode enables high definition image recording and makes it possible to obtain an increase in recording density and a stable output over a long lifetime, which results in expectation of an expanded demand in the future. The peak wavelength of blue laser beam is preferably from 300 nm to 500 nm, and particularly preferably from 400 nm to 500 nm.

Laser beam which oscillates in a longitudinal multiple modulation by a method such as high frequency superposition is also preferably employed.

### 2) Thermal development

Although any method may be used for this thermal developing process, development is usually performed by elevating the temperature of the photothermographic material exposed imagewise. The temperature of development is preferably from 80°C to 250°C, more preferably from 100°C to 140°C, and even more preferably from 110°C to 130°C.

Time period for development is preferably from 3 second to 20 seconds, more preferably from 4 seconds to 18 seconds and, even more preferably from 5 seconds to 15 seconds.

In the process of thermal development, either a drum type heater or a plate type heater may be used, but a plate type heater is preferred. A preferable process of thermal development by a plate type heater is a process described in JP-A No. 11-133572, which discloses a thermal developing apparatus in which a visible image is obtained by bringing a photothermographic material with a formed latent image into contact with a heating means at a thermal developing section, wherein the heating means comprises a plate heater, and a plurality of pressing rollers are oppositely provided along one surface of the plate heater, the thermal developing apparatus is characterized in that thermal development is performed by passing the photothermographic material between the pressing rollers and the plate heater. It is preferred that the plate heater is divided into 2 to 6 steps, with the leading end having a lower temperature by 1°C to 10°C. For example, 4 sets of plate heaters which can be independently subjected to the temperature control are used, and are controlled so that they respectively become 112°C,119°C, 121°C, and 120°C. Such a process is also described in JP-A No. 54-30032, which allows for passage of moisture and organic solvents included in the photothermographic material out of the system, and also allows for suppressing the change of shapes of the support of the photothermographic material upon rapid heating of the photothermographic material.

For downsizing the thermal developing apparatus and for reducing the time period for thermal development, it is preferred that the heater is more stably controlled, and a top part of one sheet of the photothermographic material is exposed and thermal development of the exposed part is started before exposure of the end part of the sheet has completed,. Preferable imagers which enable a rapid process according to the invention are described in, for example, JP-A Nos. 2002-289804 and 2002-287668. Using such imagers, thermal development within 14 seconds is possible with a plate type heater having three heating plates which are controlled, for example, at 107°C, 121°C and 121 °C, respectively. Thus, the output time period for the first sheet can be reduced to about 60 seconds. For such a rapid developing process, there exist various problems described above, so it is particularly preferred to use the photothermographic materials used in the invention in combination with the process.

### 3) System

Examples of a medical laser imager equipped with an exposing portion and a thermal developing portion include Fuji Medical Dry Laser Imager FM-DPL and DRYPIX 7000. In connection with FM-DPL, description is found in Fuji Medical Review No. 8, pages 39 to 55. The described techniques may be applied as the laser imager for the photothermographic material of the invention. In addition, the present photothermographic material can be also applied as a photothermographic material for the laser imager used in "AD network" which was proposed by Fuji Film Medical Co., Ltd. as a network system accommodated to DICOM standard.

### (Application of the invention)

The photothermographic material used in the invention is preferably used for photothermographic materials for use in medical diagnosis, photothermographic materials for use in industrial photographs, photothermographic materials for use in graphic arts, as well as for COM, through forming black and white images by silver imaging.

### EXAMPLES

The present invention is specifically explained by way of Examples below, which should not be construed as limiting the invention thereto.

### EXAMPLE 1

### (Preparation of PET Support)

### 1) Film Manufacturing

PET having IV (intrinsic viscosity) of 0.66 (measured in phenol/tetrachloroethane = 6/4 (mass ratio) at 25°C) was obtained according to a conventional manner using terephthalic acid and ethylene glycol. The product was pelletized, dried at 130°C for 4 hours, and melted at 300°C. Thereafter, the mixture was extruded from a T-die and rapidly cooled to form a non-tentered film.

The film was stretched along the longitudinal direction by 3.3 times using rollers of different peripheral speeds, and then stretched along the transverse direction by 4.5 times using a tenter machine. The temperatures used for these operations were 110°C and 130°C, respectively. Then, the film was subjected to thermal fixation at 240°C for 20 seconds, and relaxed by 4% along the transverse direction at the same temperature. Thereafter, the chucking part was slit off, and both edges of the film were knurled. Then the film was rolled up at the tension of 4 kg/cm² to obtain a roll having the thickness of 175 µm.

### 2) Surface Corona Discharge Treatment

Both surfaces of the support were treated at room temperature at 20 m/minute using Solid State Corona Discharge Treatment Machine Model 6KVA manufactured by Piller GmbH. It was proven that treatment of 0.375 kV-A minute/m² was executed, judging from the readings of current and voltage on that occasion. The frequency upon this treatment was 9.6 kHz, and the gap clearance between the electrode and dielectric roll was 1.6 mm.

### 3) Undercoating

| Formula (1) (for undercoat layer on the image forming layer side) | |
|---|---|
| Pesresin A-520 manufactured by Takamatsu Oil & Fat Co., Ltd. (30% by weight solution) | 46.8 g |
| BAIRONAARU MD-1200 manufactured by Toyo Boseki Co., Ltd. | 10.4 g |
| Polyethyleneglycol monononylphenylether (average ethylene oxide number = 8.5) 1% by weight solution | 11.0 g |
| MP-1000 manufactured by Soken Chemical & Engineering Co., Ltd.(PMMA polymer fine particle, mean particle diameter of 0.4 µm) | 0.91 g |
| Distilled water | 931 mL |
| Formula (2) (for first layer on the backside) | |
| Styrene-butadiene copolymer latex (solid content of 40% by weight, styrene/butadiene mass ratio = 68/32) | 130.8 g |
| Sodium salt of 2,4-dichloro-6-hydroxy-S-triazine (8% by weight aqueous solution) | 5.2 g |
| 1% by weight aqueous solution of sodium laurylbenzenesulfonate | 10 mL |
| Polystyrene particle dispersion (mean particle diameter of 2 µm, 20% by weight) | 0.5 g |
| Distilled water | 854 mL |
| Formula (3) (for second layer on the backside) | |
| SnO₂/SbO (9/1 mass ratio, mean particle diameter of 0.5 µm, 17% by weight dispersion) | 84 g |
| Gelatin | 7.9 g |
| METOLOSE TC-5 manufactured by Shin-Etsu Chemical Co., Ltd. (2% by weight aqueous solution) | 10 g |
| 1% by weight aqueous solution of sodium dodecylbenzenesulfonate | 10 mL |
| NaOH (1% by weight) | 7 g |
| Proxel (manufactured by imperial Chemical Industries PLC) | 0.5 g |
| Distilled water | 881 mL |

Both surfaces of the biaxially tentered polyethylene terephthalate support having the thickness of 175 µm were subjected to the corona discharge treatment as described above, respectively. Thereafter, the aforementioned formula (1) of the coating solution for the undercoat was coated on one surface (image forming layer side) with a wire bar so that the amount of wet coating became 6.6 mL/m² (per one side), and dried at 180°C for 5 minutes. Then, the aforementioned formula (2) of the coating solution for the undercoat was coated on the reverse side (backside) with a wire bar so that the amount of wet coating became 5.7 mL/m², and dried at 180°C for 5 minutes. Furthermore, the aforementioned formula (3) of the coating solution for the undercoat was coated on the reverse side (backside) with a wire bar so that the amount of wet coating became 8.4 mL/m², and dried at 180°C for 6 minutes. Thus, an undercoated support was produced.

### (Back Layer)

### 1) Preparation of Coating Solution for Back Layer

### <Preparation of Dispersion of Solid Fine Particles (a) of Base Precursor>

2.5 kg of base precursor-1, 300 g of a surfactant (trade name: DEMOL N, manufactured by Kao Corporation), 800 g of diphenylsulfone, and 1.0 g of benzoisothiazolinone sodium salt were mixed with distilled water to give the total amount of 8.0 kg. This mixed liquid was subjected to beads dispersion using a horizontal sand mill (UVM-2: manufactured by AIMEX Co., Ltd.). Process of dispersion includs feeding the mixed liquid to UVM-2 packed with zirconia beads having a mean particle diameter of 0.5 mm with a diaphragm pump, followed by the dispersion at the inner pressure of 50 hPa or higher until desired mean particle diameter could be achieved.

Dispersion was continued until the ratio of the optical density at 450 nm to the optical density at 650 nm for the spectral absorption of the dispersion (D₄₅₀/ D₆₅₀) became 3.0 upon spectral absorption measurement. The resulting dispersion was diluted with distilled water so that the concentration of the base precursor became 25% by weight, and filtrated (with a polypropylene filter having a mean fine pore diameter of 3 µm) for eliminating dust to put into practical use.

### 2) Preparation of Solid Fine Particle Dispersion of Dye

Cyanine dye-1 in an amount of 6.0 kg, 3.0 kg of sodium p-dodecylbenzenesulfonate, 0.6 kg of DEMOL SNB (a surfactant manufactured by Kao Corporation), and 0.15 kg of a defoaming agent (trade name: SURFYNOL 104E, manufactured by Nissin Chemical Industry Co., Ltd.) were mixed with distilled water to give the total amount of 60 kg. The mixed liquid was subjected to dispersion with 0.5 mm zirconia beads using a horizontal sand mill (UVM-2: manufactured by AIMEX Co., Ltd.).

Dispersion was continued until the ratio of the optical density at 650 nm to the optical density at 750 nm for the spectral absorption of the dispersion (D₆₅₀/ D₇₅₀) became 5.0 or higher upon spectral absorption measurement. The resulting dispersion was diluted with distilled water so that the concentration of the cyanine dye became 6% by weight, and filtrated with a filter (mean fine pore diameter: 1 µm) for eliminating dust to put into practical use.

### 3) Preparation of Coating Solution for Antihalation Layer

A vessel was kept at 40°C, and thereto were added 37 g of gelatin having an isoelectric point of 6.6 (ABA gelatin, manufactured by Nippi Co., Ltd.), 0.1 g of benzoisothiazolinone, and water to allow gelatin to be dissolved. Additionally, 36 g of the above-mentioned dispersion of the solid fine particles of the dye, 73 g of the above-mentioned dispersion of the solid fine particles (a) of the base precursor, 43 mL of a 3% by weight aqueous solution of sodium polystyrenesulfonate, and 82 g of a 10% by weight solution of SBR latex (styrene/ butadiene/ acrylic acid copolymer; mass ratio of the copolymerization of 68.3/ 28.7/ 3.0) were admixed to give a coating solution for the antihalation layer in an amount of 773 mL. The pH of the resulting coating solution was 6.3.

### 4) Preparation of Coating Solution for Back Surface Protective Layer

A vessel was kept at 40°C, and thereto were added 43 g of gelatin having an isoelectric point of 4.8 (PZ gelatin, manufactured by Miyagi Chemical Industry Co., Ltd.), 0.21 g of benzoisothiazolinone, and water to allow gelatin to be dissolved. Additionally, 8.1 mL of a 1 mol/L sodium acetate aqueous solution, 0.93 g of monodispersed fine particles of poly(ethylene glycol dimethacrylate-co-methylmethacrylate) (mean particle diameter of 7.7 µm, standard deviation of particle diameter of 0.3), 5 g of a 10% by weight emulsion of liquid paraffin, 10 g of a 10% by weight emulsion of dipentaerythritol hexaisostearate, 10 mL of a 5% by weight aqueous solution of sodium di(2-ethylhexyl)sulfosuccinate, 17 mL of a 3% by weight aqueous solution of sodium polystyrenesulfonate, 2.4 mL of a 2% by weight solution of a fluorocarbon surfactant (F-1), 2.4 mL of a 2% by weight solution of another fluorocarbon surfactant (F-2), and 30 mL of a 20% by weight solution of ethyl acrylate/ acrylic acid copolymer (mass ratio of the copolymerization of 96.4/ 3.6) latex were admixed. Just prior to the coating, 50 mL of a 4% by weight aqueous solution of N,N-ethylenebis(vinylsulfone acetamide) was admixed to give a coating solution for the back surface protective layer in an amount of 855 mL. The pH of the resulting coating solution was 6.2.

### 5) Coating of Back Layer

The backside of the undercoated support described above was subjected to simultaneous double coating so that the coating solution for the antihalation layer gave the coating amount of gelatin of 0.54 g/m², and so that the coating solution for the back surface protective layer gave the coating amount of gelatin of 1.85 g/m², followed by drying to produce a back layer.

### (Image Forming Layer, Intermediate Layer, and Surface Protective Layer)

### 1. Preparations of Coating Material

### 1) Preparation of Silver Halide Emulsion

### <<Preparation of Silver Halide Emulsion 1>>

A liquid was prepared by adding 3.1 mL of a 1% by weight potassium bromide solution, and then 3.5 mL of 0.5 mol/L sulfuric acid and 31.7 g of phthalated gelatin to 1421 mL of distilled water. The liquid was kept at 30°C while stirring in a stainless steel reaction vessel, and thereto were added total amount of: solution A prepared through diluting 22.22 g of silver nitrate by adding distilled water to give the volume of 95.4 mL; and solution B prepared through diluting 15.3 g of potassium bromide and 0.8 g of potassium iodide with distilled water to give the volume of 97.4 mL, over 45 seconds at a constant flow rate. Thereafter, 10 mL of a 3.5% by weight aqueous solution of hydrogen peroxide was added thereto, and 10.8 mL of a 10% by weight aqueous solution of benzimidazole was further added. Moreover, a solution C prepared through diluting 51.86 g of silver nitrate by adding distilled water to give the volume of 317.5 mL and a solution D prepared through diluting 44.2 g of potassium bromide and 2.2 g of potassium iodide with distilled water to give the volume of 400 mL were added. A controlled double jet method was executed through adding total amount of the solution C at a constant flow rate over 20 minutes, accompanied by adding the solution D while maintaining the pAg at 8.1. Potassium hexachloroiridate (III) was added in its entirely to give 1 × 10⁻⁴ mol per 1 mol of silver, at 10 minutes post initiation of the addition of the solution C and the solution D. Moreover, at 5 seconds after completing the addition of the solution C, a potassium hexacyanoferrate (II) in an aqueous solution was added in its entirety to give 3 × 10⁻⁴ mol per I mol of silver. The mixture was adjusted to the pH of 3.8 with 0.5 mol/L sulfuric acid. After stopping stirring, the mixture was subjected to precipitation/ desalting/ water washing steps. The mixture was adjusted to the pH of 5.9 with 1 mol/L sodium hydroxide to produce a silver halide dispersion having the pAg of 8.0.

The above-described silver halide dispersion was kept at 38°C with stirring, and thereto was added 5 mL of a 0.34% by weight methanol solution of 1,2-benzisothiazoline-3-one, followed by elevating the temperature to 47°C at 40 minutes thereafter. At 20 minutes after elevating the temperature, sodium benzene thiosulfonate in a methanol solution was added at 7.6 × 10⁻⁵ mol per 1 mol of silver. At additional 5 minutes later, a tellurium sensitizer C in a methanol solution was added at 2.9 × 10⁻⁴ mol per 1 mol of silver and subjected to ripening for 91 minutes. Thereafter, a methanol solution of a spectral sensitizing dye A and a spectral sensitizing dye B with a molar ratio of 3 : 1 was added thereto at 1.2 × 10⁻³ mol in total of the spectral sensitizing dye A and B per 1 mol of silver. At 1 minute later, 1.3 mL of a 0.8% by weight methanol solution of N,N'-dihydroxy-N",N"-diethylmelamine was added thereto, and at additional 4 minutes thereafter, 5-methyl-2-mercaptobenzimidazole in a methanol solution at 4.8 × 10⁻³ mol per 1 mol of silver, 1-phenyl-2-heptyl-5-mercapto-1,3,4-triazole in a methanol solution at 5.4 × 10⁻³ mol per 1 mol of silver, and 1-(3-methylureidophenyl)-5-mercaptotetrazole in an aqueous solution at 8.5 × 10⁻³ mol per 1 mol of silver were added to produce a silver halide emulsion 1.

Grains in thus prepared silver halide emulsion were silver iodobromide grains having a mean equivalent spherical diameter of 0.042 µm, a variation coefficient of an equivalent spherical diameter distribution of 20%, which uniformly include iodine at 3.5 mol%. Grain size and the like were determined from the average of 1000 grains using an electron microscope. The {100} face ratio of these grains was found to be 80% using a Kubelka-Munk method.

### <<Preparation of Silver Halide Emulsion 2>>

Preparation of silver halide dispersion 2 was conducted in a similar manner to the process in the preparation of the silver halide emulsion 1 except that: the temperature of the liquid upon the grain forming process was altered from 30°C to 47°C; the solution B was changed to that prepared through diluting 15.9 g of potassium bromide with distilled water to give the volume of 97.4 mL; the solution D was changed to that prepared through diluting 45.8 g of potassium bromide with distilled water to give the volume of 400 mL; time period for adding the solution C was changed to 30 minutes; and potassium hexacyanoferrate (II) was deleted; further the precipitation/desalting/ water washing/ dispersion were carried out similar to the silver halide emulsion 1. Furthermore, the spectral sensitization, chemical sensitization, and addition of 5-methyl-2-mercaptobenzimidazole and 1-phenyl-2-heptyl-5-mercapto-1,3,4-triazole were executed to the silver halide dispersion 2 similar to the silver halide emulsion 1 except that: the amount of the tellurium sensitizer C to be added was changed to 1.1 × 10⁻⁴ mol per 1 mol of silver; the amount of the methanol solution of the spectral sensitizing dye A and a spectral sensitizing dye B with a molar ratio of 3 : 1 to be added was changed to 7.0 × 10⁻⁴ mol in total of the spectral sensitizing dye A and the spectral sensitizing dye B per 1 mol of silver; the addition of 1-phenyl-2-heptyl-5-mercapto-1,3,4-triazole was changed to give 3.3 × 10⁻³ mol per 1 mol of silver; and the addition of 1-(3-methylureidophenyl)-5-mercaptotetrazole was changed to give 4.7 × 10⁻³ mol per 1 mol of silver, to produce silver halide emulsion 2. Grains in the silver halide emulsion 2 were cubic pure silver bromide grains having a mean equivalent spherical diameter of 0.080 µm and a variation coefficient of an equivalent spherical diameter distribution of 20%.

### «Preparation of Silver Halide Emulsion 3»

Preparation of silver halide dispersion 3 was conducted in a similar manner to the process in the preparation of the silver halide emulsion 1 except that the temperature of the liquid upon the grain forming process was altered from 30°C to 27°C, and in addition, the precipitation/ desalting/ water washing/ dispersion were carried out similarly to the silver halide emulsion 1. Silver halide emulsion 3 was obtained similarly to the silver halide emulsion 1 except that: to the silver halide dispersion 3, the addition of the methanol solution of the spectral sensitizing dye A and the spectral sensitizing dye B was changed to the solid dispersion (aqueous gelatin solution) at a molar ratio of 1 : 1 with the amount to be added being 6 × 10⁻³ mol in total of the spectral sensitizing dye A and spectral sensitizing dye B per 1 mol of silver; the amount of the tellurium sensitizer C to be added was changed to 5.2 × 10⁻⁴ mol per 1 mol of silver; and bromoauric acid at 5 × 10⁻⁴ mol per 1 mol of silver and potassium thiocyanate at 2 × 10⁻³ mol per 1 mol of silver were added at 3 minutes following the addition of the tellurium sensitizer. Grains in the silver halide emulsion 3 were silver iodobromide grains having a mean equivalent spherical diameter of 0.034 µm and a variation coefficient of an equivalent spherical diameter distribution of 20%, which uniformly include iodine at 3.5 mol%.

### «Preparation of Mixed Emulsion A for Coating Solution»

The silver halide emulsion 1 at 70% by weight, the silver halide emulsion 2 at 15% by weight, and the silver halide emulsion 3 at 15% by weight were dissolved, and thereto was added benzothiazolium iodide in a 1% by weight aqueous solution to give 7 × 10⁻³ mol per 1 mol of silver.

Further, as "a compound that can be one-electron-oxidized to provide a one-electron oxidation product, which releases one or more electrons", the compounds Nos. 1, 2, and 3 were added respectively in an amount of 2 × 10⁻³ mol per 1 mol of silver in silver halide.

Thereafter, as "a compound having an adsorptive group and a reducing group", the compound Nos. 1 and 2 were added respectively in an amount of 5 × 10⁻³ mol per 1 mol of silver halide.

Further, water was added thereto to give the content of silver of 38.2 g per 1 kg of the mixed emulsion for a coating solution, and 1-(3-methylureidophenyl)-5-mercaptotetrazole was added to give 0.34 g per 1 kg of the mixed emulsion for a coating solution.

### 2) Preparation of Dispersion of Silver Salt of Fatty Acid

88 kg of the recrystallized behenic acid, 422 L of distilled water, 49.2 L of 5 mol/L sodium hydroxide aqueous solution, 120 L of t-butyl alcohol were admixed, and subjected to a reaction with stirring at 75°C for one hour to give a solution of sodium behenate. Separately, 206.2 L of an aqueous solution of 40.4 kg of silver nitrate (pH 4.0) was provided, and kept at a temperature of 10°C. A reaction vessel charged with 635 L of distilled water and 30 L of t-butyl alcohol was kept at 30°C, and thereto were added the total amount of the solution of sodium behenate and the total amount of the aqueous silver nitrate solution with sufficient stirring at a constant flow rate over 93 minutes and 15 seconds, and 90 minutes, respectively. Upon this operation, during first 11 minutes following the initiation of adding the aqueous silver nitrate solution, the added material was restricted to the aqueous silver nitrate solution alone. The addition of the solution of sodium behenate was thereafter started, and during 14 minutes and 15 seconds following the completion of adding the aqueous silver nitrate solution, the added material was restricted to the solution of sodium behenate alone. The temperature inside of the reaction vessel was then set to be 30°C, and the temperature outside was controlled so that the liquid temperature could be kept constant. In addition, the temperature of a pipeline for the addition system of the solution of sodium behenate was kept constant by circulation of warm water outside of a double wall pipe, so that the temperature of the liquid at an outlet in the leading edge of the nozzle for addition was adjusted to be 75°C. Further, the temperature of a pipeline for the addition system of the aqueous silver nitrate solution was kept constant by circulation of cool water outside of a double wall pipe. Position at which the solution of sodium behenate was added and the position, at which the aqueous silver nitrate solution was added, was arranged symmetrically with a shaft for stirring located at a center. Moreover, both of the positions were adjusted to avoid contact with the reaction liquid.

After completing the addition of the solution of sodium behenate, the mixture was left to stand at the temperature as it was for 20 minutes. The temperature of the mixture was then elevated to 35°C over 30 minutes followed by ripening for 210 minutes. Immediately after completing the ripening, solid matters were filtered out with centrifugal filtration. The solid matters were washed with water until the electric conductivity of the filtrated water became 30 µS/cm. A silver salt of a fatty acid was thus obtained. The resulting solid matters were stored as a wet cake without drying.

When the shape of the resulting particles of the silver behenate was evaluated by an electron micrography, a crystal was revealed having a = 0.21 µm, b =0.4 µm and c = 0.4 µm on the average value, with a mean aspect ratio of 2.1, and a variation coefficient of an equivalent spherical diameter distribution of 11% (a, b and c are as defined aforementioned.).

To the wet cake corresponding to 260 kg of a dry solid matter content, were added 19.3 kg of poly(vinyl alcohol) (trade name: PVA-217) and water to give the total amount of 1000 kg. Then, a slurry was obtained from the mixture using a dissolver blade. Additionally, the slurry was subjected to preliminary dispersion with a pipeline mixer (manufactured by MIZUHO Industrial Co., Ltd.: PM-10 type).

Next, a stock liquid after the preliminary dispersion was treated three times using a dispersing machine (trade name: Microfluidizer M-610, manufactured by Microfluidex International Corporation, using Z type Interaction Chamber) with the pressure controlled to be 1150 kg/cm² to give a dispersion of silver behenate. For the cooling manipulation, coiled heat exchangers were equipped in front of and behind the interaction chamber respectively, and accordingly, the temperature for the dispersion was set to be 18°C by regulating the temperature of the cooling medium.

### 3) Preparation of Reducing Agent Dispersion

### <<Preparation of Reducing Agent-1 Dispersion>>

To 10 kg of reducing agent-1 (2,2'-methylenebis-(4-ethyl-6-tertbutylphenol)) and 16 kg of a 10% by weight aqueous solution of modified poly(vinyl alcohol) (manufactured by Kuraray Co., Ltd., Poval MP203) was added 10 kg of water, and thoroughly mixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 3 hours. Thereafter, 0.2 g of a benzisothiazolinone sodium salt and water were added thereto, thereby adjusting the concentration of the reducing agent to be 25% by weight. This dispersion was subjected to heat treatment at 60°C for 5 hours to obtain reducing agent-1 dispersion. Particles of the reducing agent included in the resulting reducing agent dispersion had a median diameter of 0.40 µm, and a maximum particle diameter of 1.4 µm or less. The resultant reducing agent dispersion was subjected to filtration with a polypropylene filter having a pore size of 3.0 µm to remove foreign substances such as dust, and stored.

### <<Preparation of Reducing Agent-2 Dispersion>>

To 10 kg of reducing agent-2 (6,6'-di-t-butyl-4,4'-dimethyl-2,2'-butylidenediphenol)) and 16 kg of a 10% by weight aqueous solution of modified poly(vinyl alcohol) (manufactured by Kuraray Co., Ltd., Poval MP-203) was added 10 kg of water, and thoroughly mixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 3 hours and 30 minutes. Thereafter, 0.2 g of a benzoisothiazolinone sodium salt and water were added thereto, thereby adjusting the concentration of the reducing agent to be 25% by weight. This dispersion was warmed at 40°C for one hour, followed by a subsequent heat treatment at 80°C for one hour to obtain reducing agent-2 dispersion. Particles of the reducing agent included in the resulting reducing agent dispersion had a median diameter of 0.50 µm, and a maximum particle diameter of 1.6 µm or less. The resultant reducing agent dispersion was subjected to filtration with a polypropylene filter having a pore size of 3.0 µm to remove foreign substances such as dust, and stored.

### 4) Preparation of Hydrogen Bonding Compound-1 Dispersion

To 10 kg of hydrogen bonding compound-1(tri(4-t-butylphenyl)phosphineoxide) and 16 kg of a 10% by weight aqueous solution of modified poly(vinyl alcohol) (manufactured by Kuraray Co., Ltd., Poval MP203) was added 10 kg of water, and thoroughly mixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 4 hours. Thereafter, 0.2 g of a benzisothiazolinone sodium salt and water were added thereto, thereby adjusting the concentration of the hydrogen bonding compound to be 25% by weight. This dispersion was warmed at 40°C for one hour, followed by a subsequent heat treatment at 80°C for one hour to obtain hydrogen bonding compound-1 dispersion. Particles of the hydrogen bonding compound included in the resulting hydrogen bonding compound dispersion had a median diameter of 0.45 µm, and a maximum particle diameter of 1.3 µm or less. The resultant hydrogen bonding compound dispersion was subjected to filtration with a polypropylene filter having a pore size of 3.0 µm to remove foreign substances such as dust, and stored.

### 5) Preparation of Development Accelerator-1 Dispersion

To 10 kg of development accelerator-1 and 20 kg of a 10% by weight aqueous solution of modified poly(vinyl alcohol) (manufactured by Kuraray Co., Ltd., Poval MP203) was added 10 kg of water, and thoroughly mixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 3 hours and 30 minutes. Thereafter, 0.2 g of a benzisothiazolinone sodium salt and water were added thereto, thereby adjusting the concentration of the development accelerator to be 20% by weight. Accordingly, development accelerator-1 dispersion was obtained. Particles of the development accelerator included in the resulting development accelerator dispersion had a median diameter of 0.48 µm, and a maximum particle diameter of 1.4 µm or less. The resultant development accelerator dispersion was subjected to filtration with a polypropylene filter having a pore size of 3.0 µm to remove foreign substances such as dust, and stored.

### 6) Preparations of Solid Dispersions of Development Accelerator-2 and Color-tone-adjusting Agent-1

Also concerning solid dispersions of development accelerator-2 and color-tone-adjusting agent-1, dispersion was executed similar to the development accelerator-1, and thus dispersions of 20% by weight and 15% by weight were respectively obtained.

### 7) Preparations of Organic Polyhalogen Compound Dispersion

### <<Preparation of Organic Polyhalogen Compound-1Dispersion>>

10 kg of organic polyhalogen compound-1 (tribromomethane sulfonylbenzene), 10 kg of a 20% by weight aqueous solution of modified poly(vinyl alcohol) (manufactured by Kuraray Co., Ltd., Poval MP203), 0.4 kg of a 20% by weight aqueous solution of sodium triisopropylnaphthalenesulfonate and 14 kg of water were thoroughly admixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 5 hours. Thereafter, 0.2 g of a benzisothiazolinone sodium salt and water were added thereto, thereby adjusting the concentration of the organic polyhalogen compound to be 26% by weight. Accordingly, organic polyhalogen compound-1 dispersion was obtained. Particles of the organic polyhalogen compound included in the resulting organic polyhalogen compound dispersion had a median diameter of 0.41 µm, and a maximum particle diameter of 2.0 µm or less. The resultant organic polyhalogen compound dispersion was subjected to filtration with a polypropylene filter having a pore size of 10.0 µm to remove foreign substances such as dust, and stored.

### <<Preparation of Organic Polyhalogen Compound-2 Dispersion>>

10 kg of organic polyhalogen compound-2 (N-butyl-3-tribromomethane sulfonylbenzamide), 20 kg of a 10% by weight aqueous solution of modified poly(vinyl alcohol) (manufactured by Kuraray Co., Ltd., Poval MP203) and 0.4 kg of a 20% by weight aqueous solution of sodium triisopropylnaphthalenesulfonate were thoroughly admixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 5 hours. Thereafter, 0.2 g of a benzisothiazolinone sodium salt and water were added thereto, thereby adjusting the concentration of the organic polyhalogen compound to be 30% by weight. This dispersion was heated at 40°C for 5 hours to obtain organic polyhalogen compound-2 dispersion. Particles of the organic polyhalogen compound included in the resulting organic polyhalogen compound dispersion had a median diameter of 0.40 µm, and a maximum particle diameter of 1.3 µm or less. The resultant organic polyhalogen compound dispersion was subjected to filtration with a polypropylene filter having a pore size of 3.0 µm to remove foreign substances such as dust, and stored.

### 8) Preparation of Phthalazine Compound-1 Solution

Modified poly(vinyl alcohol) MP-203 in an amount of 8 kg was dissolved in 174.57 kg of water, and then thereto were added 3.15 kg of a 20% by weight aqueous solution of sodium triisopropylnaphthalenesulfonate and 14.28 kg of a 70% by weight aqueous solution of phthalazine compound-1 (6-isopropyl phthalazine) to prepare a 5% by weight phthalazine compound-1 solution.

### 9) Preparations of Aqueous Solution of Mercapto Compound

### <<Preparation of Aqueous Solution of Mercapto Compound-1>>

Mercapto compound-1 (1-(3-sulfophenyl)-5-mercaptotetrazole sodium salt) in an amount of 7 g was dissolved in 993 g of water to give a 0.7% by weight aqueous solution.

### <<Preparation of Aqueous Solution of Mercapto Compound-2>>

Mercapto compound-2 (1-(3-methylureidophenyl)-5-mercaptotetrazole) in an amount of 20 g was dissolved in 980 g of water to give a 2.0% by weight aqueous solution.

### 10) Preparation of Pigment-1 Dispersion

C.I. Pigment Blue 60 in an amount of 64 g and 6.4 g of DEMOL N manufactured by Kao Corporation were added to 250 g of water and thoroughly mixed to give a slurry. Zirconia beads having the mean particle diameter of 0.5 mm were provided in an amount of 800 g, and charged in a vessel with the slurry. Dispersion was performed with a dispersing machine (1/4G sand grinder mill: manufactured by AIMEX Co., Ltd.) for 25 hours. Thereto was added water to adjust so that the concentration of the pigment became 5% by weight to obtain a pigment-1 dispersion. Particles of the pigment included in the resulting pigment dispersion had a mean particle diameter of 0.21 µm.

### 11) Preparation of SBR Latex Solution

To a polymerization tank of a gas monomer reaction apparatus (manufactured by Taiatsu Techno Corporation, TAS-2J type), were charged 287 g of distilled water, 7.73 g of a surfactant (Pionin A-43-S (manufactured by TAKEMOTO OIL & FAT CO., LTD.): solid matter content of 48.5% by weight), 14.06 mL of 1 mol/L sodium hydroxide, 0.15 g of ethylenediamine tetraacetate tetrasodium salt, 255 g of styrene, 11.25 g of acrylic acid, and 3.0 g of tert-dodecyl mercaptan, followed by sealing of the reaction vessel and stirring at a stirring rate of 200 rpm. Degassing was conducted with a vacuum pump, followed by repeating nitrogen gas replacement several times. Thereto was injected 108.75 g of 1,3-butadiene, and the inner temperature is elevated to 60°C. Thereto was added a solution of 1.875 g of ammonium persulfate dissolved in 50 mL of water, and the mixture was stirred for 5 hours as it stands. The temperature was further elevated to 90°C, followed by stirring for 3 hours. After completing the reaction, the inner temperature was lowered to reach to the room temperature, and thereafter the mixture was treated by adding 1 mol/L sodium hydroxide and ammonium hydroxide to give the molar ratio of Na⁺ ion : NH₄⁺ ion = 1 : 5.3, and thus, the pH of the mixture was adjusted to 8.4. Thereafter, filtration with a polypropylene filter having the pore size of 1.0 µm was conducted to remove foreign substances such as dust followed by storage. Accordingly, SBR latex was obtained in an amount of 774.7 g.

Upon the measurement of halogen ion by ion chromatography, concentration of chloride ion was revealed to be 3 ppm. As a result of the measurement of the concentration of the chelating agent by high performance liquid chromatography, it was revealed to be 145 ppm.

The aforementioned latex had a mean particle diameter of 90 nm, Tg of 17°C, solid matter concentration of 44% by weight, the equilibrium moisture content at 25°C and 60%RH of 0.6% by weight, ionic conductance of 4.80 mS/cm (measurement of the ionic conductance performed using a conductivity meter CM-30S manufactured by Toa Electronics Ltd. for the latex stock solution (44% by weight) at 25°C).

### 2. Preparations of Coating Solution

### 1) Preparation of Coating Solution for Image Forming Layer

To the dispersion of silver salt of a fatty acid obtained as described above in an amount of 1000 g and 135 mL of water were serially added 36 g of the pigment-1 dispersion, 25 g of the organic polyhalogen compound-1 dispersion, 39g of the organic polyhalogen compound-2 dispersion, 171 g of the phthalazine compound-1 solution, 1060 g of the SBR latex solution, 153 g of the reducing agent-2 dispersion, 22 g of the hydrogen bonding compound-1 dispersion, 4.8 g of the development accelerator-1 dispersion, 5.2 g of the development accelerator-2 dispersion, 2.1 g of the color-tone-adjusting agent-1 dispersion, and 8 mL of the mercapto compound-2 aqueous solution. The mixed emulsion A for coating solution in an amount of 140 g was added thereto, followed by thorough mixing just prior to the coating, which was fed directly to a coating die, and coated.

Viscosity of the above-described coating solution for image forming layer was 35 [mPa-s] which was measured with a B type viscometer at 40°C (No. 1 rotor, 60 rpm).

Viscosity of the coating solution at 38°C when it was measured using Rheo Stress RS150 manufactured by Haake Co. Ltd. was 38, 49, 48, 34, and 25 [mPa·s], respectively, at the shearing rate of 0.1, 1, 10, 100, 1000

### [1/second]

The amount of zirconium in the coating solution was 0.30 mg per 1 g of silver.

### 2) Preparation of Coating Solution for Intermediate Layer A

To 1000 g of poly(vinyl alcohol) PVA-205 (manufactured by Kuraray Co., Ltd.), 163 g of the pigment-1 dispersion, 33g of a 18.5% by weight aqueous solution of a blue dye-1 (manufactured by Nippon Kayaku Co., Ltd.: Kayafect turquoise RN liquid 150), 27 mL of a 5% by weight aqueous solution of sodium di(2-ethylhexyl)sulfosuccinate, and 4200 mL of a 19% by weight solution of methyl methacrylate/ styrene/ butyl acrylate/ hydroxyethyl methacrylate/ acrylic acid copolymer (mass ratio of the copolymerization of 57/ 8/ 28/ 5/ 2) latex, 27 mL of a 5% by weight aqueous solution of aerosol OT (manufactured by American Cyanamid Co.), 135 mL of a 20% by weight aqueous solution of diammonium phthalate was added water to give total amount of 10000 g. The mixture was adjusted with sodium hydroxide to give the pH of 7.5. Accordingly, the coating solution for the intermediate layer was prepared, and was fed to a coating die to provide 8.9 mL/m².

Viscosity of the coating solution was 58 [mPa·s] which was measured with a B type viscometer at 40°C (No. I rotor, 60 rpm).

### 3) Preparation of Coating Solution for First Layer of Surface Protective Layers

In 840 mL of water were dissolved 100 g of inert gelatin and 10 mg of benzoisothiazolinone, and thereto were added 180 g of a 19% by weight solution of methyl methacrylate/ styrene/ butyl acrylate/ hydroxyethyl methacrylate/ acrylic acid copolymer (mass ratio of the copolymerization of 57/ 8/ 28/ 5/ 2) latex, 46 mL of a 15% by weight methanol solution of phthalic acid, and 5.4 mL of a 5% by weight aqueous solution of sodium di(2-ethylhexyl)sulfosuccinate, and were mixed. Immediately before coating, 40 mL of a 4% by weight chrome alum which had been mixed with a static mixer was fed to a coating die so that the amount of the coating solution became 26.1 mL/m².

Viscosity of the coating solution was 20 [mPa·s] which was measured with a B type viscometer at 40°C (No. 1 rotor, 60 rpm)

### 4) Preparation of Coating Solution for Second Layer of Surface Protective Layers

In 800 mL of water were dissolved 100 g of inert gelatin and 10 mg of benzoisothiazolinone, and thereto were added 10 g of a 10% by weight liquid paraffin emulsion, 30 g of a 10% by weight emulsion of dipentaerythritol hexa-isostearate, 180 g of a 19% by weight solution of methyl methacrylate/ styrene/ butyl acrylate/ hydroxyethyl methacrylate/ acrylic acid copolymer (mass ratio of the copolymerization of 57/ 8/ 28/ 5/ 2) latex, 40 mL of a 15% by weight methanol solution of phthalic acid, 5.5 mL of a 1 % by weight solution of a fluorocarbon surfactant (F-1), 5.5 mL of a 1 % by weight aqueous solution of another fluorocarbon surfactant (F-2), 28 mL of a 5% by weight aqueous solution of sodium di(2-ethylhexyl)sulfosuccinate, 4 g of polymethyl methacrylate fine particles (mean particle diameter of 0.7 µm, volume weighted mean distribution of 30%), and 21 g of polymethyl methacrylate fine particles (mean particle diameter of 3.6 µm, volume weighted mean distribution of 60%), and the obtained mixture was mixed to give a coating solution for the surface protective layer, which was fed to a coating die so that 8.3 mL/m² could be provided.

Viscosity of the coating solution was 19 [mPa·s] which was measured with a B type viscometer at 40°C (No. 1 rotor, 60 rpm).

### 3. Preparations of Photothermographic Material

### 1) Preparation of Photothermographic Material-101

Reverse surface of the back surface was subjected to simultaneous overlaying coating by a slide bead coating method in order of coating solution for the image forming layer, the coating solution for intermediate layer, the coating solution for the first layer of the surface protective layers, and the coating solution for the second layer of the surface protective layers, starting from the undercoated face, and thus sample of photothermographic material was produced. In this method, the temperature of the coating solution was adjusted to 31°C for the image forming layer and intermediate layer, to 36°C for the first layer of the surface protective layers, and to 37°C for the second layer of the surface protective layers.

The coating amount of each compound (g/m²) for the image forming layer is as follows.

| | |
|---|---|
| Silver salt of fatty acid | 5.27 |
| Pigment (C, I. Pigment Blue 60) | 0.036 |
| Organic polyhalogen compound- 1 | 0.014 |
| Organic polyhalogen compound-2 | 0.028 |
| Phthalazine compound-1 | 0.18 |
| SBR latex | 9.43 |
| Reducing agent-2 | 0.77 |
| Hydrogen bonding compound- 1 | 0.112 |
| Development accelerator-1 | 0.019 |
| Development accelerator-2 | 0.016 |
| Color-tone-adjusting agent- 1 | 0.006 |
| Mercapto compound-2 | 0.003 |
| Silver halide (on the basis of Ag content) | 0.13 |

Conditions for coating and drying were as follows.

Coating was performed at the speed of 160 m/min. The clearance between the leading end of the coating die and the support was from 0.10 mm to 0.30 mm. The pressure in the vacuum chamber was set to be lower than atmospheric pressure by 196 Pa to 882 Pa. The support was decharged by ionic wind.

In the subsequent cooling zone, the coating solution was cooled by wind having the dry-bulb temperature of from 10°C to 20°C. Transportation with no contact was carried out, and the coated support was dried with an air of the dry-bulb of from 23°C to 45°C and the wet-bulb of from 15°C to 21°C in a helical type contactless drying apparatus.

After drying, moisture conditioning was performed at 25°C in the humidity of from 40%RH to 60%RH. Then, the film surface was heated to be from 70°C to 90°C, and after heating, the film surface was cooled to 25°C.

Thus prepared photothermographic material had a level of matting of 550 seconds on the image forming layer side, and 130 seconds on the back surface as Beck's smoothness. In addition, measurement of pH of the film surface on the image forming layer side gave the result of 6.0.

### 2) Preparations of Photothermographic Material-102 to -115

Preparations of photothermographic material-102 to -115 were conducted in a similar manner to the process in the preparation of photothermographic material-101, except that the second organic silver salt was added in the image forming layer, the intermediate layer, the first layer of surface protective layers, or the second layer of surface protective layers of the photothermographic material-101, as described in the following Table 1. The following dispersions were employed for the second organic silver salt.

### <Organic Silver Salt A: Silver Behenate Dispersion>

In the case where the second organic silver salt was added in the image forming layer or the intermediate layer, the dispersion of silver salt of a fatty acid described above (organic silver salt A-1) was used as the silver behenate dispersion. The silver potential measured by the method described in [Second organic silver salt incorporated in non-photosensitive layer] was +390 mV.

In the case where the second organic silver salt was added in the first layer of surface protective layers or the second layer of surface protective layers, 40 g of a 5% by weight aqueous solution of sodium di(2-ethylhexyl)sulfosuccinate and 80 g of a 5% by weight aqueous solution of inert gelatin, and 20 g of water were added to the above silver salt of a fatty acid corresponding to 260 kg of a dry solid matter content to give a slurry and then the slurry was subjected to preliminary dispersion with a pipeline mixer.

Next, the obtained preliminary dispersion was treated three times using a dispersing machine (trade name: Microfluidizer M-110EH, manufactured by Microfluidex International Corporation, using Z type Interaction Chamber) with the pressure controlled to be 1320 kg/cm² to give a silver behenate dispersion (organic silver salt A-2). For the cooling manipulation, coiled heat exchangers were equipped in front of and behind the interaction chamber respectively, and accordingly, the temperature for the dispersion was set to be 18°C by regulating the temperature of the cooling medium. The silver potential measured was +392 mV.

### <Organic Silver Salt B: Silver Laurate Dispersion >

In the case where the second organic silver salt was added in the image forming layer or the intermediate layer, the organic silver salt dispersion (organic silver salt B-1) was prepared in a similar manner to the process in the preparation of the dispersion of silver salt of a fatty acid described above except that using 51.8 kg of lauric acid instead of using 88 kg of recrystallized behenic acid. The silver potential measured was +509 mV.

In the case where the second organic silver salt was added in the first layer of surface protective layers or the second layer of surface protective layers, the organic silver salt dispersion (organic silver salt B-2) was prepared in a similar manner to the process in the preparation of the above organic silver salt A-2. The silver potential measured was +510 mV.

### <Organic Silver Salt C: Dispersion of Silver Salt of Benzotriazole>

A dispersion of silver salt of benzotriazole was prepared by the method described in Example 1 of JP-A No. 1-100177. The silver potential measured was +315 mV.

### <Organic Silver Salt D: Dispersion of Silver Salt of 1-Phenyl-5-mercaptotetrazole>

A dispersion of silver salt of 1-phenyl-5-mercaptotetrazole was prepared by the method described in Example 1 of JP-A No. 1-100177. The silver potential measured was +60 mV.

### <Organic Silver Salt E: Silver Phthalate Dispersion>

500 g of disodium phthalate was dissolved into 4500 g of water and the mixture was kept at 50°C. 4.16 liters of an aqueous solution containing 930 g of silver nitrate prepared separately was added to the disodium phthalate solution with stirring over 30 minutes. Thereafter, the resulting mixture was ripened while stirring for one hour, and then solid matters were filtered out with centrifugal filtration. The solid matters were washed with water until the electric conductivity of the filtrated water became 30 µS/cm. Organic silver salt E was prepared using the above organic silver salt corresponding to 123 kg of a dry solid matter content in a similar manner to the process in the preparation of organic silver salt A-2.

### <Organic Silver Salt F: Dispersion of Silver Salt of Polymer P-1>

A dispersion of silver salt of polymer P-1 was prepared by the method described in Example 1 of JP-A No. 2003-330137.

Chemical structures of the compounds used in Examples of the invention are shown below.

Compound 1 that can be one-electron-oxidized to provide a one-electron oxidation product which releases one or more electrons

Compound 2 that can be one-electron-oxidized to provide a one-electron oxidation product which releases one or more electrons

Compound 3 that can be one-electron-oxidized to provide a one-electron oxidation product which releases one or more electrons

Compound 1 having adsorptive group and reducing group

Compound 2 having adsorptive group and reducing group

### 3. Evaluation of Photographic Properties

### 1) Preparation

The obtained sample was cut into a half-cut size (43 cm in length × 35 cm in width), and was wrapped with the following packaging material under an environment of 25°C and 50%RH, and stored for 2 weeks at an ambient temperature.

### «Packaging Material»

A film laminated with PET 10 µm/ PE 12 µm/ aluminum foil 9 µm/ Ny 15 µm/ polyethylene 50 µm containing carbon at 3% by weight:
oxygen permeability at 25°C: 0.02 mL·atm⁻¹m⁻²day⁻¹;
vapor permeability at 25°C: 0.10 g·atm⁻¹m⁻²day⁻¹.

### 2) Exposure and Thermal Development

To each sample, exposure and thermal development (with 3 panel heaters set to 107°C - 121°C - 121°C; test was performed by modifying the apparatus so that time period for thermal development could be changed) with Fuji Medical Dry Laser Imager DRYPIX 7000 (equipped with 660 nm laser diode having a maximum output of 50 mW (IIIB)) were performed. Evaluation on an obtained image was performed with a densitometer.

### 3) Evaluation Condition

### (Photographic Properties)

Fog: Fog is expressed in terms of a density of the unexposed portion.

Sensitivity: Sensitivity is the inverse of the exposure value giving a density of 1.2. The sensitivities are shown in relative value, detecting the sensitivity of Sample No. 101 to be 100.

Dmax: Dmax is a saturated maximum density obtained with increasing the exposure value.

### (Fingerprint Stain before Exposure)

In a dark room under an environment of 25°C and 60RH%, the surfaces of the image forming layer of unexposed sample were touched by 10 persons with a hand, and then subjected to exposure for giving a density of 1.2 and thermal development. The obtained samples were sensory evaluated on the stain by fingerprint before exposure.
⊚ : Almost negligible stain.
O: Stain by fingerprint of one or two persons is observed, but in a slight degree.
Δ : Stain by fingerprint of three or more persons is observed in a serious degree.
× : Stain by fingerprint of five or more persons is observed in a significant degree.

### (Raw stock storability)

The unexposed samples stored under an environment of 30°C and 70RH% for 3 days and in a freezer were subjected to exposure to give a density of 1.2 and thermal development. The obtained samples were evaluated on image tone by the following criteria.
⊚ : No difference in image tones is observed between both samples.
○ : Slight difference in image tones is observed between both samples, but in practically acceptable level.
Δ : Yellowish image tone is observed on the sample stored under an environment of 30°C and 70RH%.
×: Deep yellowish image tone is observed on the sample stored under an environment of 30°C and 70RH%, in practically unacceptable level.

### (Evaluation on Resistance to Scratch after Processing)

The samples subjected to exposure to give a density of 3.0 and thermal development were prepared and the image surfaces thereof were rubbed by a commercial nylon scrubbing pad at a scrubbing speed of 1 cm per second with a load of 20 g/cm². After rubbing thereto, the film surfaces were visually observed and the number of the scratched trace was counted. The smaller the number is, the better the resistance is.

### 4) Results

The obtained results are shown in Table 1.

**TABLE 1**

| Sample No. | Organic Silver Salt in the Non-photosensitive Layer | | | Time Period for Thermal Development (second) | Photographic Properties | | | Fingerprint Stain before Exposure | Raw Stock Storability | Scratch after Processing (number) | Note |
|---|---|---|---|---|---|---|---|---|---|---|---|
| | Dispersion No. | Addition Amount (Ag-mol/m²) | Added Layer | | Fog | Sensi tivity | Dmax | | | | |
| 101 | - | - | - | 14 | 0.18 | 100 | 3.9 | × | × | 2 | Comparative |
| 102 | - | - | - | 24 | 0.21 | 125 | 3.9 | × | × | 2 | Comparative |
| 103 | A-1 | 1 × 10⁻³ | Intermediate Layer | 24 | 0.21 | 123 | 3.9 | × | × | 1 | Comparative |
| 104 | A-1 | 1 × 10⁻³ | Intermediate Layer | 14 | 0.18 | 100 | 3.9 | Δ | Δ | 1 | Comparative |
| 105 | A-2 | 10 × 10³ | First Layer of Surface Protective Layers | 14 | 0.18 | 100 | 3.9 | Δ | Δ | 1 | Comparative |
| 108 | A-1 | 1 × 10⁻³ | Image Forming Layer | 14 | 0.20 | 110 | 4.1 | × | × | 2 | Comparative |
| 107 | B-1 | 1 × 10⁻³ | Intermediate Layer | 14 | 0.18 | 100 | 3.9 | ⊚ | ○ | 1 | Comparative |
| 108 | B-2 | 1 × 10⁻³ | First Layer of Surface Protective Layers | 14 | 0.18 | 100 | 3.9 | ⊚ | ○ | 0 | Comparative |
| 109 | C | 1 × 10⁻³ | First layer of Surface Protective Layers | 14 | 0.18 | 100 | 3.9 | ⊚ | ○ | 0 | Invention |
| 110 | C | 1 × 10⁻³ | First Layer of Surface Protective Layers | 14 | 0.21 | 123 | 3.9 | Δ | × | 0 | Comparative |
| 111 | D | 1 × 10⁻³ | First Layer of Surface Protective Layers | 14 | 0.18 | 100 | 3.9 | ○ | Δ | 0 | Invention |
| 112 | E | 1 × 10⁻³ | First Layer of Surface Protective Layers | 14 | 0.18 | 100 | 3.9 | ○ | Δ | 0 | Comparative |
| 113 | F | 1 × 10⁻³ | First layer of Surface Protective Layers Protective Layers | 14 | 0.18 | 100 | 3.9 | ○ | Δ | 0 | Comparative |
| 114 | C | 1 × 10⁻³ | Second Layer of Surface Protective Layers | 14 | 0.18 | 100 | 3.9 | ⊚ | ○ | 0 | Invention |
| 115 | C | 5 × 10⁻⁴ | First Layer of Surface Protective Layers | 14 | 0.18 | 100 | 3.9 | ○ | ○ | 0 | Invention |

It is apparent from Table 1 that at the time period for thermal development within the range used for the present invention, the samples in which the second organic silver salt was included in the surface protective layer and the intermediate layer, which are disposed above the image forming layer, exhibit excellent results in stain by fingerprint before exposure, raw stock storability, and scratch after processing while maintaining photographic properties. Moreover, when the silver potential of the second organic silver salt fall in a range of from +300 mV to +600 mV, excellent results are attained. When time period for thermal development is long (for example, 24 seconds), the effect of the second organic silver salt is insufficient to depress the stain by fingerprint before exposure. A strict explanation of the above phenomenon is difficult, but it is supposed that they may have some relation with the difference in grain sizes of developed silver formed by respective time for development. Therefore, time period for development within the range employed for the image forming method of the present invention is preferred.

### EXAMPLE 2

### (Preparations of Sample)

### 1) Preparation of Sample No. 201

In sample No. 101 of Example 1, the following second intermediate layer was disposed between the image forming layer and the intermediate layer.

### (Preparation of Coating Solution for Second Intermediate Layer)

The coating solution for the second intermediate layer was prepared in a similar manner to the process in the preparation of coating solution for intermediate layer A except that omitting blue dye-1 and, instead of using poly(vinyl alcohol) PVA-205 and methacrylate/ styrene/ butylacrylate/ hydroxyethyl methacrylate/ acrylic acid copolymer, using the following polymer latex in an amount same as the total amount of the above polymers.

P-8 : A copolymer latex of St(70.5)/ Bu(26.5) / AA (3) (crosslinking, Tg: 23°C).

In the structure above, abbreviations represent monomers as follows. St: styrene, Bu: butadiene, and AA: acrylic acid. The numbers in the parenthesis indicates % by weight.

### 2) Preparations of Sample Nos. 202 to 213

Samples Nos. 202 to 213 were prepared by adding the organic silver salt in the image forming layer, the second intermediate layer, the intermediate layer, or the first layer of surface protective layers as described in Table 2. Evaluation similar to Example 1 was performed. Time period for thermal development was set to 14 seconds.

### (Evaluation of Performance)

The obtained samples were evaluated similar to Example 1, and the obtained results are shown in Table 3.

The samples in which the organic silver salt different from the one in the image froming layer was included in the surface protective layer or the intermediate layers disposed above the image forming layer exhibit excellent results in lower stain by fingerprint before exposure, raw stock storability, and scratch resistance after processing while keeping the photographic properties.

Sample Nos. 202 and 203, in which only silver laurate is used in the non-photosensitive layer, have a tendency to increase fog. However, sample Nos. 204, 209 and 210, in which silver salt of benzotriazole is used in the non-photosensitive layer, no increase in fog is observed and more preferable performances are seen. Further, sample No. 205 to 208, which contain the organic silver salt in plural layers of non-photosensitive layers, exhibit the most excellent performances.

**TABLE 2**

| Sample No. | Image Forming Layer | | Second Intermediate Layer | | Intermediate Layer | | First Layer of Surface Protective Layers | | Note |
|---|---|---|---|---|---|---|---|---|---|
| | Dispersion No. | Addition Amount (Ag-mol/m²) | Dispersion No. | Addition Amount (Ag-mol/m²) | Dispersion No. | Addition Amount (Ag-mol/m²) | Dispersion No. | Addition Amount (Ag-mol/m²) | |
| 201 | - | - | - | - | - | - | - | - | Comparative |
| 202 | - | - | B-1 | 1 × 10⁻³ | - | - | - | - | Invention |
| 203 | - | - | - | - | B-1 | 1 × 10⁻³ | - | - | Invention |
| 204 | - | - | - | - | - | - | C | 1 × 10⁻³ | Invention |
| 205 | - | - | - | - | B-1 | 5 × 10⁻⁴ | C | 5 × 10⁻⁴ | Invention |
| 206 | - | - | B-1 | 5 × 10⁻⁴ | B-1 | 5 × 10⁻⁴ | C | 5 × 10⁻⁴ | Invention |
| 207 | - | - | - | - | A-1 | 5 × 10⁻⁴ | C | - 5 × 10⁻⁴ | Invention |
| 208 | - | - | A-1 | 1 × 10⁻³ | - | - | C | 5 × 10⁻⁴ | Invention |
| 209 | - | - | C | 1 × 10⁻³ | - | - | - | - | Invention |
| 210 | - | - | - | - | C | 1 × 10⁻³ | - | - | Invention |
| 211 | - | - | - | - | - | - | A-2 | 1 × 10⁻³ | Comparative |
| 212 | - | - | - | - | A-2 | 1 × 10⁻³ | - | - | Comparative |
| 213 | C | 1 × 10⁻³ | - | - | - | - | - | - | Comparative |

**TABLE 3**

| Sample No. | Photographic Properties | | | Fingerprint Stain before Exposure | Raw Stock Storability | Scratch after Processing (number) | Note |
|---|---|---|---|---|---|---|---|
| | Fog | Sensitivity | Dmax | | | | |
| 201 | 0.17 | 80 | 3.7 | Δ | × | 2 | Comparative |
| 202 | 0.18 | 80 | 3.8 | ⊚ | Δ | 1 | Invention |
| 203 | 0.18 | 80 | 3.8 | ⊚ | ○ | 0 | Invention |
| 204 | 0.17 | 78 | 3.7 | ⊚ | ○ | 0 | Invention |
| 205 | 0.17 | 80 | 3.7 | ⊚ | ⊚ | 0 | Invention |
| 206 | 0.17 | 80 | 3.8 | ⊚ | ⊚ | 0 | Invention |
| 207 | 0.17 | 80 | 3.8 | ⊚ | ⊚ | 0 | Invention |
| 208 | 0.17 | 80 | 3.7 | ⊚ | ⊚ | 0 | Invention |
| 209 | 0.17 | 80 | 3.7 | ⊚ | ○ | 0 | Invention |
| 210 | 0.17 | 80 | 3.7 | ⊚ | ○ | 0 | Invention |
| 211 | 0.18 | 82 | 3.8 | Δ | × | 2 | Comparative |
| 212 | 0.18 | 82 | 3.8 | Δ | × | 2 | Comparative |
| 213 | 0.17 | 80 | 3.7 | Δ | × | 2 | Comparative |

## Claims

1. An image forming method comprising: using a photothermographic material comprising, on at least one side of a support, an image forming layer comprising at least a photosensitive silver halide, a first non-photosensitive organic silver salt, a reducing agent represented by the following formula (R), and a binder, and at least one non-photosensitive layer which is disposed on the same side as the image forming layer and farther from the support than the image forming layer, and comprises a second organic silver salt which is different from the first non-photosensitive organic silver salt, wherein the first non-photosensitive organic silver salt is a silver behenate and the second organic silver salt is a silver salt of an azole compound, 50 % by weight or more of the binder in the image forming layer is formed by a hydrophobic polymer latex having a glass transition temperature of from 0°C to 80°C, 50 % by weight or more of a binder in the non-photosensitive layer is formed by a hydrophobic polymer latex, and the photothermographic material comprises a developing accelerator represented by the following formula (A-1) or (A-2); imagewise exposing the photothermographic material; and thermal developing for 5 seconds to 15 seconds at 110°C to 130°C after imagewise exposure:
Formula (A-1) Q₁-NHM-Q₂
wherein Q₁ represents an aromatic group or a heterocyclic group which bonds to -NHNH-Q₂ at a carbon atom, and Q₂ represents a carbamoyl group: wherein R₁ represents one selected from an alkyl group, an acyl group, an acylamino group, a sulphonamide group, an alkoxycarbonyl group, or a carbamoyl group; R₂ represents one selected from a hydrogen atom, a halogen atom, an alkyl group, an alkoxy group, an aryloxy group, an alkylthio group, an arylthio group, an acyloxy group, or a carbonate ester group; R₃ and R₄ each independently represent a group capable of substituting for a hydrogen atom on a benzene ring; and R₃ and R₄ may link together to form a condensed ring: wherein R¹¹ and R^{11'} each independently represent a tertiary alkyl group having 4 to 15 carbon atoms; R¹² and R^{12'} each independently represent a hydrogen atom or a substituent which can be bonded to the benzene ring; L represents an -S- group or a -CHR¹³-group; R¹³ represents a hydrogen atom or an alkyl group having 1 to 20 carbon atoms; and X¹ and X^{1'} each independently represent a hydrogen atom or a substituent which can be bonded to the benzene ring.

2. The image forming method according to claim 1, wherein the photothermographic material comprises a fluorocarbon compound which has two or more fluoroalkyl groups having two or more carbon atoms and 11 or fewer fluorine atoms and has at least one of an anionic or nonionic hydrophilic group.

3. The image forming method according to claim 1, wherein the silver salt of an azole compound is a silver salt of a benzotriazole compound.

4. The image forming method according to claim 1, wherein the silver salt of an azole compound is a silver salt of an imidazole compound.

5. The image forming method according to claim 1, wherein a silver potential is from +50 mV to +700 mV (with respect to a standard hydrogen electrode) at 25°C in an aqueous dispersion or solution of the second organic silver salt.

6. The image forming method according to claim 1, wherein 50 % by weight or more of a solvent of a coating solution for the image forming layer is water.

7. The image forming method according to claim 1, wherein 50 % by weight or more of a solvent of a coating solution for the non-photosensitive layer is water.

8. The image forming method according to claim 1, wherein the photothermographic material comprises a non-photosensitive intermediate layer between the image forming layer and the non-photosensitive layer comprising the second organic silver salt which is different from the first non-photosensitive organic silver salt, and 50 % by weight or more of a binder in the non-photosensitive intermediate layer is formed by a hydrophobic polymer latex.

## Patentansprüche

1. Bilderzeugungsverfahren, umfassend: die Verwendung eines photothermographischen Materials, umfassend auf mindestens einer Seite eines Trägers eine Bilderzeugungsschicht, die mindestens ein lichtempfindliches Silberhalogenid, ein erstes nichtlichtempfindliches organisches Silbersalz, ein durch die folgende Formel (R) dargestelltes Reduktionsmittel und ein Bindemittel umfasst, und mindestens eine nicht-lichtempfindliche Schicht, die auf derselben Seite wie die bilderzeugende Schicht und weiter weg liegend vom Träger als die bilderzeugende Schicht angebracht ist und ein zweites organisches Silbersalz umfasst, das von dem ersten nicht-lichtempfindlichen organischen Silbersalz verschieden ist, wobei das erste nicht-lichtempfindliche organische Silbersalz ein Silberbehenat ist und das zweite organische Silbersalz ein Silbersalz einer Azolverbindung ist, 50 Gew.% oder mehr des Bindemittels in der bilderzeugenden Schicht durch einen hydrophoben Polymerlatex mit einer Glasübergangstemperatur von 0°C bis 80°C gebildet wird, 50 Gew.% oder mehr des Bindemittels in der nicht-lichtempfindlichen Schicht durch einen hydrophoben Polymerlatex gebildet wird und das photothermographische Material einen durch die folgende Formel (A-1) oder (A-2) dargestellten Entwicklungsbeschleuniger umfasst; die bildweise Belichtung des photothermographischen Materials; und die thermische Entwicklung für 5 Sekunden bis 15 Sekunden bei 110°C bis 130°C nach der bildweisen Belichtung:
Formel (A-1) Q₁-NHNH-Q₂
worin Q₁ eine aromatische Gruppe oder heterocyclische Gruppe darstellt, die an -NHNH-Q₂ an einem Kohlenstoffatom bindet und Q₂ eine Carbamoylgruppe darstellt: worin R₁ einen Vertreter darstellt, der aus einer Alkylgruppe, einer Acylgruppe, einer Acylaminogruppe, einer Sulfonamidgruppe, einer Alkoxycarbonylgruppe oder einer Carbamoylgruppe ausgewählt wird; R₂ einen Vertreter darstellt, der aus einem Wasserstoffatom, einem Halogenatom, einer Alkylgruppe, einer Alkoxygruppe, einer Aryloxygruppe, einer Alkylthiogruppe, einer Arylthiogruppe, einer Acyloxygruppe oder einer Carbonatestergruppe ausgewählt wird; R₃ und R₄ jeweils unabhängig voneinander eine Gruppe darstellen, die zur Substitution eines Wasserstoffatoms an einen Benzolring geeignet ist; und R₃ und R₄ zur Bildung eines kondensierten Rings miteinander verbunden sein können: worin R¹¹ und R^{11'} jeweils unabhängig voneinander eine tertiäre Alkylgruppe mit 4 bis 15 Kohlenstoffatomen darstellten; R¹² und R^{12'} jeweils unabhängig voneinander ein Wasserstoffatom oder einen Substituenten darstellen, der an den Benzolring gebunden werden kann; L eine -S-Gruppe oder eine -CHR¹³-Gruppe darstellt; R¹³ ein Wasserstoffatom oder eine Alkylgruppe mit 1 bis 20 Kohlenstoffatomen darstellt; und X¹ und X^{1'} jeweils unabhängig voneinander ein Wasserstoffatom oder einen Substituenten darstellen, der an den Benzolring gebunden sein kann.

2. Bilderzeugungsverfahren gemäß Anspruch 1, worin das photothermographische Material eine Fluorkohlenstoffverbindung umfasst, die zwei oder mehrere Fluoralkylgruppen mit zwei oder mehreren Kohlenstoffatomen und 11 oder weniger Fluoratomen aufweist und mindestens eine von einer anionischen oder einer nicht-ionischen hydrophilen Gruppe aufweist.

3. Bilderzeugungsverfahren gemäß Anspruch 1, worin das Silbersalz einer Azolverbindung ein Silbersalz einer Benzotriazolverbindung ist.

4. Bilderzeugungsverfahren gemäß Anspruch 1, worin das Silbersalz einer Azolverbindung ein Silbersalz einer Imidazolverbindung ist.

5. Bilderzeugungsverfahren gemäß Anspruch 1, worin ein Silberpotential +50 mV bis +700 mV (in Bezug auf eine Standardwasserstoffelektrode) bei 25°C in einer wässrigen Dispersion oder Lösung des zweiten organischen Silbersalzes beträgt.

6. Bilderzeugungsverfahren gemäß Anspruch 1, worin 50 Gew.% oder mehr eines Lösungsmittels einer Beschichtungslösung für die Bilderzeugungsschicht Wasser ist.

7. Bilderzeugungsverfahren gemäß Anspruch 1, worin 50 Gew.% oder mehr eines Lösungsmittels einer Beschichtungslösung für die nicht-lichtempfindliche Schicht Wasser ist.

8. Bilderzeugungsverfahren gemäß Anspruch 1, worin das photothermögraphische Material eine nicht-lichtempfindliche Zwischenschicht zwischen der Bilderzeugungsschicht und der nicht-lichtempfindlichen Schicht, umfassend das zweite organische Silbersalz, das vom ersten nicht-lichtempfindlichen organischen Silbersalz verschieden ist, umfasst und 50 Gew.% eines Bindemittels in der nicht-lichtempfindlichen Zwischenschicht durch einen hydrophoben Polymerlatex gebildet wird.

## Revendications

1. Procédé de formation d'image, comprenant les étapes consistant à : utiliser un matériau photothermographique comprenant, sur au moins une face d'un support, une couche de formation d'image comprenant au moins un halogénure d'argent photosensible, un premier sel d'argent organique non photosensible, un agent réducteur représenté par la formule (R) qui suit, et un liant, et au moins une couche non photosensible, qui est disposée sur la même face que la couche de formation d'image, et plus loin du support que la couche de formation d'image, et comprend un second sel d'argent organique différent du premier sel d'argent organique non photosensible, dans lequel le premier sel d'argent organique non photosensible est un béhénate d'argent, et le second sel d'argent organique est un sel d'argent d'un composé d'azole, 50% en poids ou plus du liant dans la couche de formation d'image sont constitués d'un latex de polymère hydrophobe présentant une température de transition vitreuse de 0°C à 80°C, 50% en poids ou plus d'un liant dans la couche non photosensible sont formés par un latex de polymère hydrophobe, et le matériau photothermographique comprend un accélérateur de développement représenté par la formule (A-1) ou (A-2) qui suit ; exposer en forme d'image le matériau photothermographique ; et développer par voie thermique pendant 5 secondes à 15 secondes, à 110°C à 130°C après exposition en forme d'image
Formule (A-1) Q₁-NHNH-Q₂
dans laquelle Q₁ représente un groupement aromatique ou un groupement hétérocyclique qui se lie à -NHNH-Q₂ à l'endroit d'un atome de carbone, et Q₂ représente un groupement carbamoyle : dans laquelle R₁ représente un élément choisi parmi un groupement alkyle, un groupement acyle, un groupement acylamino, un groupement sulfonamide, un groupement alkoxycarbonyle, ou un groupement carboxyle; R₂ représente un élément choisi parmi un atome d'hydrogène, un atome d'halogène, un groupement alkyle, un groupement alkoxy, un groupement aryloxy, un groupement alkylthio, un groupement arylthio, un groupement acyloxy ou un groupement ester carbonate; R₃ et R₄ représentent chacun, indépendamment, un groupement capable de se substituer à un atome d'hydrogène sur un anneau benzène, et R₃ et R₄ peuvent se lier l'un à l'autre pour former un anneau condensé : dans laquelle R¹¹ er R^{11'} représentent chacun indépendamment un groupement alkyle tertiaire comptant 4 à 15 atomes de carbone; R¹² et R^{12'} représentent chacun indépendamment un atome d'hydrogène ou un substituant qui peut être lié à l'anneau benzène; L représente un groupement -S- ou un groupement -CHR¹³ ; R¹³ représente un atome d'hydrogène ou un groupement alkyle comptant 1 à 20 atomes de carbone ; et X¹ et X^{1'} représentent chacun indépendamment un atome d'hydrogène ou un substituant qui peut être lié à l'anneau benzène.

2. Procédé de formation d'image selon la revendication 1, dans lequel le matériau photothermographique comprend un composé fluorocarboné qui présente deux groupements fluoroalkyle ou plus, comptant deux atomes de carbone ou plus, et 11 atomes de fluor ou moins, et présente l'un au moins parmi un groupement hydrophile anionique ou non ionique.

3. Procédé de formation d'image selon la revendication 1, dans lequel le sel d'argent d'un composé d'azole est un sel d'argent d'un composé de benzotriazole.

4. Procédé de formation d'image selon la revendication 1, dans lequel le sel d'argent d'un composé d'azole est un sel d'argent d'un composé d'imidazole.

5. Procédé de formation d'image selon la revendication 1, dans lequel un potentiel d'argent est de +50 mV à +700 mV (par rapport à une électrode à hydrogène standard) à 25°C dans une dispersion ou une solution aqueuse du second sel d'argent organique.

6. Procédé de formation d'image selon la revendication 1, dans lequel 50% en poids ou plus d'un solvant d'une solution d'enduction pour la couche de formation d'image sont constitués d'eau.

7. Procédé de formation d'image selon la revendication 1, dans lequel 50% en poids ou plus d'un solvant d'une solution d'enduction pour la couche non photosensible sont constitués d'eau.

8. Procédé de formation d'image selon la revendication 1, dans lequel le matériau photothermographique comprend une couche intermédiaire non photosensible, entre la couche de formation d'image et la couche non photosensible comprenant le second sel d'argent organique qui est différent du premier sel d'argent organique non photosensible, et 50% en poids ou plus d'un liant dans la couche intermédiaire non photosensible sont constitués pas un latex de polymère hydrophobe.
